



US009417540B2

(12) **United States Patent**  
**Hashimoto et al.**

(10) **Patent No.:** **US 9,417,540 B2**  
(45) **Date of Patent:** **Aug. 16, 2016**

(54) **TONER AND TWO-COMPONENT  
DEVELOPER**

(71) Applicant: **CANON KABUSHIKI KAISHA**,  
Tokyo (JP)

(72) Inventors: **Takeshi Hashimoto**, Moriya (JP);  
**Hideki Kaneko**, Yokohama (JP);  
**Nozomu Komatsu**, Toride (JP);  
**Takakuni Kobori**, Toride (JP); **Yosuke Iwasaki**, Abiko (JP); **Ichiro Kanno**, Abiko (JP); **Kohji Takenaka**, Toride (JP); **Hiroyuki Fujikawa**, Yokohama (JP)

(73) Assignee: **CANON KABUSHIKI KAISHA**,  
Tokyo (JP)

(\*) Notice: Subject to any disclaimer, the term of this patent is extended or adjusted under 35 U.S.C. 154(b) by 0 days.

(21) Appl. No.: **14/568,727**

(22) Filed: **Dec. 12, 2014**

(65) **Prior Publication Data**

US 2015/0185650 A1 Jul. 2, 2015

(30) **Foreign Application Priority Data**

Dec. 26, 2013 (JP) ..... 2013-269462

(51) **Int. Cl.**  
**G03G 9/087** (2006.01)  
**G03G 9/08** (2006.01)

(52) **U.S. Cl.**  
CPC ..... **G03G 9/081** (2013.01); **G03G 9/08755** (2013.01); **G03G 9/08793** (2013.01); **G03G 9/08797** (2013.01)

(58) **Field of Classification Search**  
CPC ..... G03G 9/08755; G03G 9/08748  
USPC ..... 430/109.4  
See application file for complete search history.

(56) **References Cited**

U.S. PATENT DOCUMENTS

|               |                         |                    |
|---------------|-------------------------|--------------------|
| 5,057,392 A * | 10/1991 McCabe          | ..... G03G 9/08755 |
|               |                         | 430/109.2          |
| 5,294,682 A * | 3/1994 Fukuda           | ..... G03G 9/08755 |
|               |                         | 430/109.2          |
| 5,747,210 A * | 5/1998 Emoto            | ..... G03G 9/08755 |
|               |                         | 430/109.4          |
| 6,203,959 B1  | 3/2001 Tanikawa et al.  |                    |
| 7,279,262 B2  | 10/2007 Fujikawa et al. |                    |

|                  |                                              |
|------------------|----------------------------------------------|
| 7,396,626 B2     | 7/2008 Fujikawa et al.                       |
| 7,858,283 B2     | 12/2010 Ishigami et al.                      |
| 7,927,775 B2     | 4/2011 Komatsu et al.                        |
| 7,939,233 B2     | 5/2011 Inoue et al.                          |
| 7,951,518 B2     | 5/2011 Ono et al.                            |
| 8,137,886 B2     | 3/2012 Baba et al.                           |
| 8,288,069 B2     | 10/2012 Fujikawa et al.                      |
| 2004/0131961 A1  | 7/2004 Watanabe et al.                       |
| 2010/0196812 A1* | 8/2010 Koike ..... G03G 9/08755<br>430/108.4 |
| 2013/0288173 A1  | 10/2013 Hashimoto et al.                     |
| 2013/0316282 A1  | 11/2013 Ishigami et al.                      |
| 2014/0030650 A1  | 1/2014 Komatsu et al.                        |
| 2015/0086917 A1  | 3/2015 Iwasaki et al.                        |

FOREIGN PATENT DOCUMENTS

|    |                |         |
|----|----------------|---------|
| EP | 1 271 255 A1   | 1/2003  |
| JP | 10239903 A *   | 9/1998  |
| JP | 2000242030 A * | 9/2000  |
| JP | 2003-280243 A  | 10/2003 |
| JP | 2008-122931 A  | 5/2008  |
| JP | 2009-175755 A  | 8/2009  |
| JP | 2013-33176 A   | 2/2013  |
| JP | 2013-105074 A  | 5/2013  |

OTHER PUBLICATIONS

English language machine translation of JP 10-239903 (Sep. 1998).\*  
English language machine translation of JP 2000-242030 (Sep. 2000).\*

European Search Report dated May 8, 2015 in European Application No. 14004323.3.

Mark, "Phenolic Resins", Encyclopedia of Polymer Science and Technology, Third Edition, 2003, vol. 7, pp. 322-367.

\* cited by examiner

*Primary Examiner* — Christopher Rodee

(74) *Attorney, Agent, or Firm* — Fitzpatrick, Cella, Harper & Scinto

(57) **ABSTRACT**

Provided is a toner obtained by melting and kneading a binder resin containing a polyester resin A and a polyester resin B, a colorant, and a wax, in which in the resin A, the content of a polyhydric alcohol unit derived from an aromatic diol, the content of a polyhydric alcohol unit derived from an oxyalkylene ether of a novolac type phenol resin, and the content of a polyvalent carboxylic acid unit derived from an aliphatic dicarboxylic acid, which contains a straight-chain hydrocarbon having 4 or more to 16 or less carbon atoms as a main chain and has carboxyl groups at both of its terminals, fall within specific ranges, and in the resin B, the content of a polyhydric alcohol unit derived from an aromatic diol and the content of a polyvalent carboxylic acid unit derived from an aromatic dicarboxylic acid or a derivative thereof fall within specific ranges.

**6 Claims, 1 Drawing Sheet**



## 1

TONER AND TWO-COMPONENT  
DEVELOPER

## BACKGROUND OF THE INVENTION

## 1. Field of the Invention

The present invention relates to a toner and a two-component developer to be used in an electrophotographic system, an electrostatic recording system, an electrostatic printing system, or a toner jet system.

## 2. Description of the Related Art

In recent years, requirements for an increase in printing speed and correspondence to energy savings have been additionally growing in association with the widespread use of a full-color copying machine of an electrophotographic system. A technology for melting a toner in an additionally quick manner in a fixing step has been studied for corresponding to high-speed printing. In addition, a technology by which the toner is fixed at an additionally low fixation temperature in order that a power consumption in the fixing step may be reduced has been studied as measures to correspond to the energy savings.

The following method is available for corresponding to the high-speed printing and improving the low-temperature fixability of the toner. The glass transition point and softening point of the binder resin of the toner are reduced, and a binder resin having sharp-melt property is used. In recent years, a polyester resin has been used as a sharp-melt resin suitable for the high-speed printing. On the other hand, the hot offset resistance of a toner that achieves low-temperature fixability is apt to reduce. Accordingly, a toner that can achieve compatibility between its low-temperature fixability and hot offset resistance has been required.

A toner containing polyester resins having different softening points has been studied in order that compatibility between low-temperature fixability and hot offset resistance may be achieved. For example, Japanese Patent Application Laid-Open No. 2003-280243 proposes such a toner that a value for a loss tangent in the range of a loss modulus  $G''$  of from  $1 \times 10^4$  Pa or more to  $1 \times 10^6$  Pa or less and the range of a loss tangent at a loss modulus  $G''$  of  $1 \times 10^3$  Pa are specified. According to Japanese Patent Application Laid-Open No. 2003-280243, a toner that contains a polyester resin containing novolac as a constituent unit, and hence easily achieves characteristic viscoelasticity and has high-speed fixability is obtained.

In addition, Japanese Patent Application Laid-Open No. 2008-122931 proposes a resin for a toner formed of a polyester resin formed of: a linear polyester that has an acid value of from 50 mgKOH/g or more to 200 mgKOH/g or less, and whose glass transition point and flow softening point satisfy a specific relationship; and a nonlinear polyester.

In addition, Japanese Patent Application Laid-Open No. 2013-105074 proposes a toner binder that contains two polyester resins different from each other in softening point and weight-average molecular weight, and whose ratio between loss tangents at specific temperatures falls within a specific range. Japanese Patent Application Laid-Open No. 2013-105074 describes that when an alkane dicarboxylic acid and/or alkene dicarboxylic acid having 4 or more to 8 or less carbon atoms are each/is incorporated at a content of from 0.1 mol % or more to 10 mol % or less into the polycarboxylic acid component of a polyester resin, the storage stability of a toner and the transparency of the binder upon its use in the toner are good. In addition, the literature describes that when a polyoxyalkylene ether of a novolac resin is incorporated at

## 2

a content of from 0.02 mol % or more to 10 mol % or less into the polyol component of a polyester resin, the storage stability of the toner is good.

The toner described in Japanese Patent Application Laid-Open No. 2003-280243, and a toner using the resin for a toner described in Japanese Patent Application Laid-Open No. 2008-122931 or the toner binder described in Japanese Patent Application Laid-Open No. 2013-105074 each have some levels of low-temperature fixability and hot offset resistance by virtue of which the toner is applicable to high-speed printing. However, when any such toner is applied to high-speed printing required in recent years in which images are printed on about 100 sheets of paper per minute, its fixability cannot be said to be sufficient. In addition, after long-term printing, a density fluctuation may enlarge or fogging may occur in a white portion.

In addition, Japanese Patent Application Laid-Open No. 2013-33176 proposes a positively chargeable toner containing a polyester resin obtained by condensing a carboxylic acid component, which is selected from the group consisting of an adipic acid compound and a succinic acid compound substituted with an alkyl group or an alkenyl group, in the presence of a titanium catalyst. The toner described in Japanese Patent Application Laid-Open No. 2013-33176 has a high initial charge quantity, and is suppressed in initial fogging and development ghost. However, Japanese Patent Application Laid-Open No. 2013-33176 describes that when the resin is applied to a negatively chargeable toner, an improving effect on the initial charge quantity and an alleviating effect on the initial fogging are not obtained. In addition, when the toner is applied to high-speed printing, its low-temperature fixability is insufficient, or a density fluctuation or fogging after long-term printing increases in some cases.

## SUMMARY OF THE INVENTION

An object of the present invention is to provide a toner that has solved the problems. Specifically, the object is to provide a toner and a two-component developer each of which: has low-temperature fixability and hot offset resistance corresponding to high-speed printing; and can suppress a fluctuation in image density and the fogging of a white portion after long-term printing.

According to one embodiment of the present invention, there is provided a toner, including:

a binder resin;

a colorant; and

a wax,

the toner being obtained through a step of melting and kneading the binder resin, the colorant, and the wax, in which:

the binder resin includes:

a polyester resin A having polyhydric alcohol unit and polyvalent carboxylic acid unit, and

a polyester resin B having a polyhydric alcohol unit and a polyvalent carboxylic acid unit;

a mass ratio (polyester resin A/polyester resin B) of the polyester resin A to the polyester resin B is from 10/90 or more to 60/40 or less;

the polyester resin A has a softening point of from 120° C. or more to 180° C. or less;

the polyester resin A contains 90 mol % or more of a polyhydric alcohol unit derived from an aromatic diol with respect to a total number of moles of the polyhydric alcohol unit, and contains 0.1 mol % or more to 10.0 mol

% or less of a polyhydric alcohol unit derived from an oxyalkylene ether of a novolac type phenol resin with respect thereto; the polyester resin A contains 15 mol % or more to 50 mol % or less of a polyvalent carboxylic acid unit derived from an aliphatic dicarboxylic acid, which contains a straight-chain hydrocarbon having 4 or more to 16 or less carbon atoms as a main chain and has carboxyl groups at both terminals of the main chain, with respect to a total number of moles of the polyvalent carboxylic acid unit; the polyester resin B has a softening point of from 80° C. or more to 100° C. or less; the polyester resin B contains 90 mol % or more of a polyhydric alcohol unit derived from an aromatic diol with respect to a total number of moles of the polyhydric alcohol unit; and the polyester resin B contains 90 mol % or more of a polyvalent carboxylic acid unit derived from one of an aromatic dicarboxylic acid and a derivative thereof with respect to a total number of moles of the polyvalent carboxylic acid unit.

Further, according to one embodiment of the present invention, there is provided a two-component developer including the toner and a magnetic carrier.

According to the present invention, it is possible to provide a toner and a two-component developer each of which: has low-temperature fixability and hot offset resistance corresponding to high-speed printing; and can suppress a fluctuation in image density and the fogging of a white portion after long-term printing.

Further features of the present invention will become apparent from the following description of exemplary embodiments with reference to the attached drawing.

#### BRIEF DESCRIPTION OF THE DRAWING

FIGURE is a view of a heat spheroidization treatment apparatus that can be used in the present invention.

#### DESCRIPTION OF THE EMBODIMENTS

Preferred Embodiments of the Present Invention will now be described in detail in accordance with the accompanying drawing.

A toner of the present invention is characterized in that: the toner contains, as a binder resin, a polyester resin A containing an aromatic diol as a main component and having a high softening point, and a polyester resin B containing an aromatic diol as a main component and having a low softening point; and the toner is obtained by melting and kneading the binder resin. In addition, the polyester resin A is characterized by having a polyhydric alcohol unit derived from an oxyalkylene ether of a novolac type phenol resin and a polyvalent carboxylic acid unit derived from an aliphatic dicarboxylic acid. In addition, the polyester resin B is characterized in that the main components of a polyhydric alcohol unit and a polyvalent carboxylic acid unit are each a diol or dicarboxylic acid having an aromatic ring. With such construction, the toner can have low-temperature fixability and hot offset resistance corresponding to high-speed printing, and suppress a fluctuation in image density and fogging after long-term printing.

The following procedure has heretofore been adopted: two polyester resins having different softening points are used as a binder resin, whereby the low-temperature fixability of a toner is improved by the polyester resin having the lower

softening point and the hot offset resistance of the toner is improved by the polyester resin having the higher softening point. However, when long-term printing is performed with such toner, a fluctuation in image density or fogging may occur. The foregoing tendency is remarkable particularly in a normal-temperature and low-humidity environment or a high-temperature and high-humidity environment. The inventors of the present invention have considered a cause for the foregoing to be as described below. The polyester resin having the lower softening point is shaved off the surface of the toner by a stress in the long-term printing to change the chargeability of the toner. With the construction of each polyester resin like the present invention, the polyester resin having the lower softening point is hardly shaved off the toner even after the long-term printing, and hence the durable stability of the toner can be improved.

The inventors of the present invention have considered a mechanism for the foregoing to be as described below. The inventors have considered that it is because the mixing of the polyester resin having the lower softening point and the polyester resin having the higher softening point in the melting-kneading step for the toner is insufficient that the chargeability changes owing to the stress due to the long-term printing. It is assumed that when the mixing is insufficient, the polyester resin having the lower softening point is apt to be exposed to the surface of the toner upon production of the toner, and is hence apt to be shaved off by the stress due to the long-term printing. It is preferred that the polyester resin having the lower softening point and the polyester resin having the higher softening point be uniformly dispersed at the time of the melting and kneading in order that the polyester resin having the lower softening point may be hardly exposed to the surface of the toner.

In order that the polyester resins having different softening points may be uniformly dispersed by the melting and kneading, the inventors of the present invention have paid attention to two factors, i.e., compatibility and steric hindrance, and have made extensive studies. As a result, the inventors have found that when components derived from aromatic diols are used as the main components of the polyhydric alcohol unit of the polyester resin having the higher softening point and the polyester resin having the lower softening point, the compatibility therebetween improves. Further, the inventors have found that the steric hindrance at the time of the melting and kneading can be overcome by incorporating, into the polyester resin having the higher softening point, a unit derived from an oxyalkylene ether of a novolac type phenol resin and a unit derived from an aliphatic dicarboxylic acid. As a result, the inventors have found that the durable stability of the toner containing the polyester resins having different softening points improves, and thus have reached the present invention.

The toner of the present invention is characterized in that the toner is obtained by melting and kneading a binder resin, a colorant, and a wax. A polyester resin A and polyester resin B to be incorporated into the binder resin are mixed upon melting and kneading together with the colorant and the wax, whereby the polyester resin B is dispersed in the polyester resin A. Thus, a toner suppressed in density fluctuation and fogging after long-term printing is obtained.

In the toner of the present invention, the binder resin contains the polyester resin A and the polyester resin B. The sum of the contents of the polyester resin A and polyester resin B in 100 parts by mass of the binder resin is preferably 90 parts by mass or more.

Both the polyester resin A and the polyester resin B each have a polyhydric alcohol unit and a polyvalent carboxylic acid unit. The polyhydric alcohol unit in the present invention

is a constituent derived from a polyhydric alcohol component used at the time of the condensation polymerization of a polyester. In addition, the polyvalent carboxylic acid unit in the present invention is a constituent derived from a polyvalent carboxylic acid used at the time of the condensation polymerization of the polyester, or an anhydride or lower alkyl ester thereof.

(Polyester Resin A)

(Softening Point)

The polyester resin A of the present invention is characterized in that its softening point is from 120° C. or more to 180° C. or less. When the softening point of the polyester resin A falls within the range, the hot offset resistance and low-temperature fixability of the toner are good. The softening point is preferably from 125° C. or more to 160° C. or less. When the softening point is less than 120° C., the hot offset resistance of the toner deteriorates, and when the softening point is more than 180° C., the low-temperature fixability of the toner deteriorates.

(Polyhydric Alcohol Unit)

Both the polyester resin A and polyester resin B of the present invention are each characterized in that the resin has a polyhydric alcohol unit and a polyvalent carboxylic acid unit, and contains 90 mol % or more of a polyhydric alcohol unit derived from an aromatic diol with respect to the total number of moles of the polyhydric alcohol unit. When the content of the polyhydric alcohol unit derived from the aromatic diol is less than 90 mol % with respect to the total number of moles of the polyhydric alcohol unit, the fogging of an image worsens. The polyhydric alcohol unit of the polyester resin A and the polyester resin B to be described later have a common structure derived from an aromatic diol. Accordingly, the resins are easily compatible with each other at the time of the melting and kneading, and hence the dispersibility of the polyester resin A and the polyester resin B after the melting and kneading improves.

Examples of the component derived from the aromatic diol include a bisphenol represented by the following chemical formula (1) and a derivative thereof.

(1)



In the chemical formula (1), R represents an ethylene or propylene group, x and y each represent an integer of 0 or more, and the average of "x+y" is from 0 or more to 10 or less.

Above all, the polyester resin A and the polyester resin B are preferably identical to each other in R in the chemical formula (1) because the polyester resin A and the polyester resin B are easily compatible with each other at the time of the melting and kneading. Further, such a propylene oxide adduct of bisphenol A that both R's each represent a propylene group and the average of "x+y" is from 2 or more to 4 or less is preferred in terms of the charging stability of the toner.

In addition, the polyester resin A of the present invention is characterized by containing 0.1 mol % or more to 10.0 mol % or less of a polyhydric alcohol unit derived from an oxyalkylene ether of a novolac type phenol resin with respect to the total number of moles of the polyhydric alcohol unit.

The oxyalkylene ether of the novolac type phenol resin has an alcoholic hydroxyl value of 3 or more and reacts with an

acid component to take a flexible crosslinked structure having a wide network. Accordingly, when the polyester resin B is mixed with the polyester resin A in the melting-kneading step for the toner, steric hindrance near a crosslinking point of the crosslinked structure of the polyester resin A is alleviated, and hence the polyester resin B is easily entangled. As a result, the polyester resin B is dispersed in the polyester resin A well and hence its exposure to the surface of the toner reduces. Accordingly, the toner becomes resistant to a stress after long-term printing. The oxyalkylene ether of the novolac type phenol resin is a reaction product of the novolac type phenol resin and a compound having one epoxy ring in a molecule thereof.

Examples of the novolac type phenol resin include the following: resins each produced by subjecting a phenol and an aldehyde to polycondensation while using an inorganic acid such as hydrochloric acid, phosphoric acid, or sulfuric acid, an organic acid such as p-toluenesulfonic acid or oxalic acid, or a metal salt such as zinc acetate as a catalyst as described in the section "Phenolic Resins" of "Encyclopedia of Polymer Science and Technology" (Interscience Publishers), Vol. 7, page 322.

Examples of the phenol include phenol and a substituted phenol having one or more hydrocarbon groups each having 1 or more to 35 or less carbon atoms, and/or halogen groups as substituents.

Specific examples of the substituted phenol include the following: cresol (ortho-cresol, meta-cresol, or para-cresol), ethylphenol, nonylphenol, octylphenol, phenylphenol, styrenated phenol, isopropenylphenol, 3-chlorophenol, 3-bromophenol, 3,5-xylenol, 2,4-xylenol, 2,6-xylenol, 3,5-dichlorophenol, 2,4-dichlorophenol, 3-chloro-5-methylphenol, dichloroxylenol, dibromoxylenol, 2,4,5-trichlorophenol, and 6-phenyl-2-chlorophenol. Two or more kinds of those phenols may be used in combination. Of those, phenol or a substituted phenol substituted with a hydrocarbon group is preferred. Of those, phenol, cresol, t-butylphenol, or nonylphenol is particularly preferred. Phenol and cresol are preferred because each of phenol and cresol is inexpensive and improves the offset resistance of the toner, and the substituted phenol substituted with a hydrocarbon group such as t-butylphenol or nonylphenol is preferred because the substituted phenol reduces the temperature dependence of the charge quantity of the toner.

Examples of the aldehyde include formalin (formaldehyde solutions having various concentrations), paraformaldehyde, trioxane, and hexamethylenetetramine. Although not particularly limited, the number-average molecular weight of the novolac type phenol resin is preferably from 300 or more to 8,000 or less, more preferably from 400 or more to 3,000 or less, still more preferably from 450 or more to 2,000 or less.

Although not particularly limited, the number-average nucleus number of the phenols in the novolac type phenol resin is preferably from 3 or more to 60 or less, more preferably from 3 or more to 20 or less, still more preferably from 4 or more to 15 or less. In addition, the softening point (JIS K2531: ring and ball method) of the novolac type phenol resin is, although not particularly limited, preferably from 40° C. or more to 180° C. or less, more preferably from 40° C. or more to 150° C. or less, still more preferably from 50° C. or more to 130° C. or less. The softening point is preferably 40° C. or more because blocking of the toner hardly occurs at normal temperature. In addition, the softening point is preferably 180° C. or less because the gelation is hardly caused in a production process for the polyester resin.

Specific examples of the compound having one epoxy ring in a molecule thereof include ethylene oxide (EO), 1,2-propylene oxide (PO), 1,2-butylene oxide, 2,3-butylene oxide,

styrene oxide, and epichlorohydrin. In addition, an aliphatic monohydric alcohol having 1 or more to 20 or less carbon atoms and a glycidyl ether of a monohydric phenol can be used. Of those, EO or PO is preferred. Although not particularly limited, the addition number of moles of the compound having one epoxy ring in a molecule thereof with respect to 1 mol of the novolac type phenol resin is preferably from 1 mol or more to 30 mol or less, more preferably from 2 mol or more to 15 mol or less, still more preferably from 2.5 mol or more to 10 mol or less. In addition, the average addition number of moles of the compound having one epoxy ring in a molecule thereof with respect to one phenolic hydroxyl group in the novolac type phenol resin is, although not particularly limited, preferably from 0.1 mol or more to 10 mol or less, more preferably from 0.1 mol or more to 4 mol or less, still more preferably from 0.2 mol or more to 2 mol or less.

An example of the structure of the oxyalkylene ether of the novolac type phenol resin to be particularly preferably used in the present invention is given below.



In the chemical formula (2), R's each represent an ethylene group or a propylene group, x represents a number of 0 or more, and y1 to y3 each independently represent a number of 0 or more.

Although not particularly limited, the number-average molecular weight of the oxyalkylene ether of the novolac type phenol resin is preferably from 300 or more to 10,000 or less, more preferably from 350 or more to 5,000 or less, still more preferably from 450 or more to 3,000 or less. The number-average molecular weight is preferably 300 or more because the hot offset resistance of the toner is good. In addition, the number-average molecular weight is preferably 10,000 or less because the gelation is hardly caused in the production process for the polyester resin A.

Although not particularly limited, the hydroxyl value (total of an alcoholic hydroxyl group and a phenolic hydroxyl group) of the oxyalkylene ether of the novolac type phenol resin is preferably from 10 mgKOH/g or more to 550 mgKOH/g or less, more preferably from 50 mgKOH/g or more to 500 mgKOH/g or less, still more preferably from 100 mgKOH/g or more to 450 mgKOH/g or less. In addition, a phenolic hydroxyl value out of the hydroxyl value is, although not particularly limited, preferably from 0 mgKOH/g or more to 500 mgKOH/g or less, more preferably from 0 mgKOH/g or more to 350 mgKOH/g or less, still more preferably from 5 mgKOH/g or more to 250 mgKOH/g or less.

The oxyalkylene ether of the novolac type phenol resin is obtained by, for example, subjecting the novolac type phenol resin and the compound having one epoxy ring in a molecule thereof to an addition reaction in the presence of a catalyst (a basic catalyst or an acid catalyst) as required. Although the temperature at which the reaction is performed is not particularly limited, the reaction temperature is preferably from 20° C. or more to 250° C. or less, more preferably from 70° C. or

more to 200° C. or less, and the reaction can be performed under normal pressure, under pressure, or under reduced pressure. In addition, the reaction can be performed in the presence of a solvent (such as xylene or dimethylformamide), or any other dihydric alcohol and/or any other alcohol that is trihydric or more.

When the content of the polyhydric alcohol unit derived from the oxyalkylene ether of the novolac type phenol resin with respect to the total number of moles of the polyhydric alcohol unit in the polyester resin A is less than 0.1 mol %, the amount of the flexible crosslinked structure portion having a wide network reduces. Accordingly, the dispersibility of the polyester resin A and the polyester resin B does not improve, and suppressing effects on a density fluctuation and fogging after long-term printing are not obtained. On the other hand, when the content of the polyhydric alcohol unit is more than 10.0 mol %, the gel content of the polyester resin A becomes excessively large. Accordingly, the polyester resin A and the polyester resin B hardly mix at the time of the melting and kneading, and hence the suppressing effects on the density fluctuation and fogging after the long-term printing are also not obtained.

As a component for forming the polyhydric alcohol unit of the polyester resin A, in addition to the aromatic diol and the oxyalkylene ether of a novolac type phenol resin, the following polyhydric alcohol components may be used as required: ethylene glycol, diethylene glycol, triethylene glycol, 1,2-propylene glycol, 1,3-propylene glycol, 1,4-butanediol, neopentyl glycol, 1,4-butenediol, 1,5-pentanediol, 1,6-hexanediol, 1,4-cyclohexanediethanol, dipropylene glycol, polyethylene glycol, polypropylene glycol, polytetramethylene glycol, sorbit, 1,2,3,6-hexanetetrol, 1,4-sorbitan, pentaerythritol, dipentaerythritol, tripentaerythritol, 1,2,4-butanetriol, 1,2,5-pantanetriol, glycerin, 2-methylpropanetriol, 2-methyl-1,2,4-butanetriol, trimethylolethane, trimethylolpropane, and 1,3,5-trihydroxymethylbenzene.

#### (Polyvalent Carboxylic Acid Unit)

The polyester resin A of the present invention is characterized by containing 15 mol % or more to 50 mol % or less of a polyvalent carboxylic acid unit derived from an aliphatic dicarboxylic acid, which contains a straight-chain hydrocarbon having 4 or more to 16 or less carbon atoms as a main chain and has carboxyl groups at both terminals of the main chain, with respect to the total number of moles of the polyvalent carboxylic acid unit.

When the aliphatic dicarboxylic acid, which contains the straight-chain hydrocarbon having 4 or more to 16 or less carbon atoms as the main chain and has carboxyl groups at both terminals of the main chain, reacts with an alcohol component, the main chain of the polyester resin has a straight-chain hydrocarbon structure in itself and hence the structure of the main chain becomes partially flexible. Accordingly, in the melting-kneading step for the toner, the polyester resin B having the lower softening point to be described later is mixed with the polyester resin A having the higher softening point by using the flexible structure as a starting point, and hence the main chain of the polyester resin A and the polyester resin B are entangled with each other to improve the dispersibility.

Examples of the aliphatic dicarboxylic acid, which contains the straight-chain hydrocarbon having 4 or more to 16 or less carbon atoms as the main chain and has carboxyl groups at both terminals of the main chain, include alkyldicarboxylic acids such as adipic acid, azelaic acid, sebacic acid, tetradecanoic acid, and octadecanoic acid, anhydrides of these acids, and lower alkyl esters of these acids as well as compounds thereof each having a structure in which part of its

main chain is branched with an alkyl group such as a methyl group, an ethyl group, or an octyl group or an alkylene group. The straight-chain hydrocarbon has preferably 4 or more to 12 or less carbon atoms, more preferably 4 or more to 10 or less carbon atoms.

When the aliphatic dicarboxylic acid to be used is an aliphatic dicarboxylic acid, which contains a straight-chain hydrocarbon having 3 or less carbon atoms as a main chain and has carboxyl groups at both terminals of the main chain, the effect by which the main chain of the polyester resin A is made flexible is hardly obtained, and hence a fluctuation in image density and fogging after long-term printing worsen. In addition, when an aliphatic dicarboxylic acid, which contains a straight-chain hydrocarbon having 17 or more carbon atoms as a main chain and has carboxyl groups at both terminals of the main chain, is used, the hot offset resistance of the toner reduces. In addition, when a dicarboxylic acid obtained by bonding a carboxyl group to a cyclohexane skeleton or a cyclohexene skeleton such as 1,4-cyclohexane dicarboxylic acid or cyclohexene-4,5-dicarboxylic acid is used, the effect by which the main chain of the polyester resin A is made flexible is hardly obtained, and hence suppressing effects on the fluctuation in image density and fogging after the long-term printing are not obtained.

When the content of the aliphatic carboxylic acid unit is less than 15 mol %, the amount of a partially flexible structure portion in the main chain of the polyester resin A reduces. Accordingly, its dispersibility with the polyester resin B deteriorates, and hence a fluctuation in image density and fogging after long-term printing worsen. On the other hand, when the content of the aliphatic carboxylic acid unit is more than 50 mol %, the main chain of the polyester resin A becomes excessively flexible, and hence the molecules of the polyester resin A are entangled with each other and the resin hardly mixes with the polyester resin B instead. Accordingly, suppressing effects on the fluctuation in image density and fogging after the long-term printing are not obtained.

As the other polyhydric carboxylic acid unit to be incorporated into the polyester resin A, there are given, for example: aromatic dicarboxylic acid such as phthalic acid, isophthalic acid, and terephthalic acid or anhydrides thereof; a succinic acid substituted with an alkyl group or alkenyl group having 6 or more to 18 or less carbon atoms or anhydrides thereof; and unsaturated dicarboxylic acids such as fumaric acid, maleic acid, and citraconic acid or anhydrides thereof. Of those units, carboxylic acids each having an aromatic ring or derivatives thereof such as terephthalic acid, isophthalic acid, trimellitic acid, pyromellitic acid, benzophenonetetracarboxylic acid, and anhydrides thereof are preferably used because the hot offset resistance of the toner can easily be improved.

#### (Polyester Resin B)

The polyester resin B of the present invention contains a polyhydric alcohol unit and a polyvalent carboxylic acid unit.

#### (Softening Point)

The polyester resin B of the present invention is characterized in that its softening point is from 80° C. or more to 100° C. or less. When the softening point of the polyester resin B falls within the range, the storage stability and low-temperature fixability of the toner are good. The softening point is preferably from 85° C. or more to 100° C. or less. When the softening point is less than 80° C., the storage stability of the toner deteriorates, and when the softening point is more than 100° C., the low-temperature fixability of the toner deteriorates.

#### (Polyhydric Alcohol Unit)

The polyester resin B is characterized by containing 90 mol % or more of a polyhydric alcohol unit derived from an aromatic diol with respect to the total number of moles of the polyhydric alcohol unit. When the content of the polyhydric alcohol unit derived from the aromatic diol is less than 90 mol % with respect to the total number of moles of the polyhydric alcohol unit, fogging worsens. The value is preferably 95 mol % or more, more preferably 100 mol % in order that compatibility between the polyester resin A and the polyester resin B may be secured.

As a component for forming the polyhydric alcohol unit of the polyester resin B other than the aromatic diol, the following polyhydric alcohol components may be used: ethylene glycol, diethylene glycol, triethylene glycol, 1,2-propylene glycol, 1,3-propylene glycol, 1,4-butanediol, neopentyl glycol, 1,4-butenediol, 1,5-pentanediol, 1,6-hexanediol, 1,4-cyclohexanediethanol, dipropylene glycol, polyethylene glycol, polypropylene glycol, polytetramethylene glycol, sorbit, 1,2,3,6-hexanetetrol, 1,4-sorbitan, pentaerythritol, dipentaerythritol, tripentaerythritol, 1,2,4-butanetriol, 1,2,5-pentanetriol, glycerin, 2-methylpropanetriol, 2-methyl-1,2,4-butanetriol, trimethylolethane, trimethylolpropane, and 1,3,5-trihydroxymethyl benzene.

#### (Polyvalent Carboxylic Acid Unit)

The polyester resin B of the present invention is characterized by containing 90 mol % or more of a polyvalent carboxylic acid unit derived from an aromatic dicarboxylic acid or a derivative thereof with respect to the total number of moles of the polyvalent carboxylic acid unit. When the content of the polyvalent carboxylic acid unit derived from an aromatic dicarboxylic acid or a derivative thereof falls within the range, compatibility between the polyester resin B and the polyester resin A is improved, and thus, a fluctuation in image density and fogging after long-term printing can be suppressed. Examples of the aromatic dicarboxylic acid or a derivative thereof include aromatic dicarboxylic acids such as phthalic acid, isophthalic acid, and terephthalic acid or anhydrides thereof.

In addition, the polyester resin B preferably contains 0.1 mol % or more to 10.0 mol % or less of a polyvalent carboxylic acid unit derived from an aliphatic dicarboxylic acid or a derivative thereof with respect to the total number of moles of the polyvalent carboxylic acid unit because the low-temperature fixability of the toner is further improved. Examples of the aliphatic dicarboxylic acid or a derivative thereof include: alkyldicarboxylic acids such as succinic acid, adipic acid, sebacic acid, and azelaic acid or anhydrides thereof; succinic acid substituted with an alkyl group or alkenyl group having 6 or more to 18 or less carbon atoms or anhydrides thereof; and unsaturated dicarboxylic acids such as fumaric acid, maleic acid, and citraconic acid or anhydrides thereof. Of those, succinic acid, adipic acid, fumaric acid and acid anhydrides thereof, and a lower alkyl ester are preferably used. An example of the polyvalent carboxylic acid unit other than those units is a trivalent or tetravalent carboxylic acid such as trimellitic acid, pyromellitic acid, benzophenonetetracarboxylic acid, or anhydrides thereof.

In addition, the acid value of the polyester resin B of the present invention is preferably from 0 mgKOH/g or more to 30 mgKOH/g or less because a change in charge quantity of the toner due to an environment is small, and the acid value is more preferably from 0 mgKOH/g or more to 20 mgKOH/g or less.

#### (Ratio of Resin a to Resin B)

In the present invention, a mass ratio A/B of the polyester resin A to the polyester resin B is characterized by being from

## 11

10/90 or more to 60/40 or less. The mass ratio A/B is preferably from 20/80 or more to 40/60 or less. When the mass ratio A/B falls within the range, the low-temperature fixability of the toner is good, and hence a fluctuation in image density and fogging after long-term printing are suppressed. When the mass ratio A/B is less than 10/90, the hot offset resistance of the toner reduces or the content of the polyester resin A is so small that the polyester resin B is hardly dispersed, and the fluctuation in image density and fogging after the long-term printing worsen. When the mass ratio A/B is more than 60/40, the low-temperature fixability of the toner deteriorates.

## (Glass Transition Temperature)

In addition, a glass transition temperature  $T_g(80)$  and glass transition temperature  $T_g(180)$  of the polyester resin A measured with a differential scanning calorimeter (DSC) preferably have a relationship represented by the following mathematical expression (1). It should be noted that the  $T_g(80)$  is a glass transition temperature measured by increasing the temperature of the resin to 80° C. once, then reducing the temperature to 30° C., and then increasing the temperature again. In addition, the  $T_g(180)$  is a glass transition temperature measured by increasing the temperature of the resin to 180° C. once, then reducing the temperature to 30° C., and then increasing the temperature again. Methods of measuring the  $T_g(80)$  and the  $T_g(180)$  are described in detail in the section "Examples".

$$-1.0 \leq T_g(80) - T_g(180) \leq 1.0 \quad (1)$$

When the polyester resin A satisfies the relationship, the entanglement of the polymer chains of the polyester resin A may be easily loosened, and hence the polyester resin A easily mixes well with the polyester resin B at the time of the melting and kneading. As a result, a fluctuation in image density and fogging after long-term printing are additionally suppressed.

In general, the glass transition point of even one and the same resin is affected by the extent to which its polymer chains are entangled with each other. The resin tends to show a higher glass transition point as the extent of entanglement enlarges. The  $T_g(80)$  is a glass transition temperature measured after the temperature of the polyester resin A has been increased to a temperature lower than the softening point of the resin by 40° C. or more and then reduced. On the other hand, the  $T_g(180)$  is a glass transition temperature measured after the temperature of the polyester resin A has been increased to a temperature equal to or higher than the softening point of the resin to accelerate the motion of its polymer chains, and then has been reduced. Therefore, the  $T_g(80)$  of a resin whose polymer chains are easily entangled with each other and hardly loosened shows a larger value than that of its  $T_g(180)$  because an influence of the entanglement cannot be completely cancelled merely by increasing its temperature to 80° C. On the other hand, the  $T_g(80)$  of a resin whose polymer chains are easily loosened shows a value substantially equal to that of its  $T_g(180)$  because the extent to which its molecular chains are entangled with each other can be reduced merely by increasing its temperature to 80° C., and a difference between both the temperatures falls within the range of  $\pm 1.0^\circ$  C. As described above, the difference between the  $T_g(80)$  and the  $T_g(180)$  originates from the crosslinked structure of the resin. The difference is caused even by a raw material constituting the polyester resin, and even when the same raw material is used, the difference is caused even by a reaction temperature, degree of vacuum, and the like in a polycondensation reaction.

It should be noted that in the case of the polyester resin B, its  $T_g(80)$  and  $T_g(180)$  show substantially the same value irrespective of a raw material and a polycondensation condi-

## 12

tion because the resin does not have a very large amount of a crosslinked structure and has a low softening point, and a difference therebetween falls within the range of  $\pm 1.0^\circ$  C.

## (Wax)

Examples of the wax used for the toner of the present invention include the following: hydrocarbon-based waxes such as a low molecular weight polyethylene, a low molecular weight polypropylene, an alkylene copolymer, a microcrystalline wax, a paraffin wax, and a Fischer-Tropsch wax; 10 oxides of hydrocarbon-based waxes such as an oxidized polyethylene wax or block copolymers thereof; waxes containing a fatty acid ester as a main component such as a carnauba wax; waxes obtained by partially or totally deoxidizing fatty acid esters such as a deoxidized carnauba wax, and further include 15 the following: saturated straight-chain fatty acids such as palmitic acid, stearic acid, and montanic acid; unsaturated fatty acids such as brassidic acid, eleostearic acid, and parinaric acid; saturated alcohols such as stearyl alcohol, aralkyl alcohol, behenyl alcohol, carnaubyl alcohol, ceryl alcohol, 20 and melissyl alcohol; polyhydric alcohols such as sorbitol; esters of fatty acids such as palmitic acid, stearic acid, behenic acid, and montanic acid and alcohols such as stearyl alcohol, aralkyl alcohol, behenyl alcohol, carnaubyl alcohol, ceryl alcohol, and melissyl alcohol; fatty acid amides such as linoleic acid amide, oleic acid amide, and lauric acid amide; 25 saturated fatty acid bisamides such as methylenebisstearyl acid amide, ethylenebiscapric acid amide, ethylenebislauryl acid amide, and hexamethylenebisstearyl acid amide; unsaturated fatty acid amides such as ethylenebisoleic acid amide, hexamethylenebisoleic acid amide, N,N'-dioleylaidipic acid amide, and N,N'-dioleylsebacic acid amide; aromatic bisamides such as m-xylenebisstearyl acid amide and N,N'-distearylisophthalic acid amide; aliphatic metal salts (generally called a metal soap) such as calcium stearate, calcium laurate, 30 zinc stearate, and magnesium stearate; waxes obtained by grafting vinyl-based monomers such as styrene and acrylic acid into aliphatic hydrocarbon-based waxes; partial esters of fatty acids such as behenic acid monoglyceride and polyhydric alcohols; and methyl ester compounds having a hydroxyl group obtained by hydrogenation of a vegetable oil and fat.

Of those waxes, hydrocarbon-based waxes such as a paraffin wax and a Fischer-Tropsch wax or fatty acid ester-based waxes such as a carnauba wax are preferred in terms of improving the low-temperature fixability and hot offset resistance of the toner. In the present invention, hydrocarbon-based waxes are more preferred in terms of additionally improving the hot offset resistance of the toner.

In the present invention, the waxes are preferably used in an amount of from 1 part by mass or more to 20 parts by mass or less with respect to 100 parts by mass of the binder resin.

In addition, the peak temperature of the highest endothermic peak of the wax in an endothermic curve at the time of temperature increase measured with a differential scanning calorimeter (DSC) is preferably from 45° C. or more to 140° C. or less. It is because compatibility between the storage stability and hot offset resistance of the toner can be achieved that the peak temperature of the highest endothermic peak of the wax preferably falls within the range.

## (Polymer C)

60 The binder resin of the toner of the present invention preferably contain a polymer C having a structure in which a vinyl-based resin component and a hydrocarbon compound are bonded to each other. The polymer C is preferably a polymer in which a polyolefin is bonded to the vinyl-based resin component or a polymer having the vinyl-based resin component obtained by bonding a vinyl-based monomer to the polyolefin. The polymer C may improve an affinity

between the polyester resin A or the polyester resin B and the wax in the toner. Accordingly, excessive exudation of the wax to the surface of the toner can be suppressed, and hence a fluctuation in image density and fogging are additionally suppressed. This is why the polymer C is preferably incorporated. The foregoing effect becomes significant particularly when the polymer is combined with a hydrocarbon-based wax.

The content of the polymer C is preferably from 2 parts by mass or more to 10 parts by mass or less, more preferably from 3 parts by mass or more to 8 parts by mass or less in 100 parts by mass of the binder resin. When the content of the polymer C falls within the range, the durable stability of the toner can be additionally improved while its low-temperature fixability is maintained.

The polyolefin in the polymer C is not particularly limited as long as the polyolefin is a polymer or copolymer of an unsaturated hydrocarbon-based monomer having one double bond, and various polyolefins can each be used. A polyethylene- or polypropylene-based polyolefin is particularly preferably used as the polyolefin.

Examples of the vinyl-based monomer used for the vinyl-based resin component in the polymer C include:

styrene-based monomers such as styrene and derivatives thereof such as styrene, o-methyl styrene, m-methyl styrene, p-methyl styrene, p-methoxy styrene, p-phenyl styrene, p-chloro styrene, 3,4-dichloro styrene, p-ethyl styrene, 2,4-dimethyl styrene, p-n-butyl styrene, p-tert-butyl styrene, p-n-hexyl styrene, p-n-octyl styrene, p-n-nonyl styrene, p-n-decyl styrene, and p-n-dodecyl styrene;

amino group-containing a-methylene aliphatic monocarboxylic acid esters such as dimethylaminoethyl methacrylate and diethylaminoethyl methacrylate; and N atom-containing vinyl-based monomers such as acrylic or methacrylic derivatives such as acrylonitrile, methacrylonitrile, and acrylamide;

unsaturated dibasic acids such as maleic acid, citraconic acid, itaconic acid, alkenyl succinic acid, fumaric acid, and mesaconic acid; unsaturated dibasic acid anhydrides such as a maleic acid anhydride, a citraconic acid anhydride, an itaconic acid anhydride, and an alkenyl succinic acid anhydride; half esters of unsaturated dibasic acids such as a methyl maleate half ester, an ethyl maleate half ester, a butyl maleate half ester, a methyl citraconate half ester, an ethyl citraconate half ester, a butyl citraconate half ester, a methyl itaconate half ester, a methyl alkenyl succinate half ester, a methyl fumarate half ester, and a methyl mesaconate half ester; esters of unsaturated dibasic acids such as dimethyl maleate and dimethyl fumarate;  $\alpha,\beta$ -unsaturated acids such as acrylic acid, methacrylic acid, crotonic acid, and cinnamic acid;  $\alpha,\beta$ -unsaturated acid anhydrides such as a crotonic anhydride and a cinnamic anhydride and anhydrides of the  $\alpha,\beta$ -unsaturated acids and lower fatty acids; and carboxyl group-containing vinyl-based monomers such as alkenyl malonic acid, alkenyl glutaric acid, alkenyl adipic acid, and an anhydride and monoester of these acids;

acrylic or methacrylic acid esters such as 2-hydroxyethyl acrylate, 2-hydroxyethyl methacrylate, and 2-hydroxypropyl methacrylate; and hydroxyl group-containing vinyl-based monomers such as 4-(1-hydroxy-1-methylbutyl)styrene and 4-(1-hydroxy-1-methylhexyl)styrene; acrylic acid esters such as methyl acrylate, ethyl acrylate, n-butyl acrylate, isobutyl acrylate, propyl acrylate, n-oc-

yl acrylate, dodecyl acrylate, 2-ethylhexyl acrylate, stearyl acrylate, 2-chloroethyl acrylate, and phenyl acrylate; and

methacrylic acid esters such as a-methylene aliphatic monocarboxylic acid esters such as methyl methacrylate, ethyl methacrylate, propyl methacrylate, n-butyl methacrylate, isobutyl methacrylate, n-octyl methacrylate, dodecyl methacrylate, 2-ethylhexyl methacrylate, stearyl methacrylate, phenyl methacrylate, dimethylaminoethyl methacrylate, and diethylaminoethyl methacrylate.

Preferably, the vinyl-based resin component in the polymer C contains a styrene-based unit, an ester-based unit, an acrylonitrile unit, or a methacrylonitrile unit as a constituent unit.

The polymer C having a structure in which the vinyl-based resin component and the hydrocarbon compound are bonded to each other to be used in the present invention can be obtained by a known method such as a reaction between such vinyl-based monomers as described in the foregoing or a reaction between a monomer for one polymer and the other polymer.

In addition to the polyester resin A, the polyester resin B, and the polymer C, the following "other resin" can be added as a binder resin to be used in the toner of the present invention for the purposes of improving pigment dispersibility, and improving the charging stability and blocking resistance of the toner in such an amount as not to inhibit any effect of the present invention.

(Other Resin)

Examples of the "other resin" include the following resins: monopolymers of styrene or a substitute thereof such as polystyrene, poly-p-chlorostyrene, and polyvinyl toluene; styrene-based copolymers such as a styrene-p-chlorostyrene copolymer, a styrene-vinyltoluene copolymer, a styrene-vinyl naphthaline copolymer, a styrene-acrylate copolymer, a styrene-methacrylate copolymer, a styrene- $\alpha$ -methyl chloromethacrylate copolymer, a styrene-acrylonitrile copolymer, a styrene-vinyl methyl ether copolymer, a styrene-vinyl ethyl ether copolymer, a styrene-vinyl methyl ketone copolymer, and a styrene-acrylonitrile-indene copolymer; and polyvinyl chloride, a phenolic resin, a natural modified phenolic resin, a natural resin-modified maleic resin, an acrylic resin, a methacrylic resin, polyvinyl acetate, a silicone resin, a polyester resin, polyurethane, a polyamide resin, a furan resin, an epoxy resin, a xylene resin, polyvinyl butyral, a terpene resin, a coumarone-indene resin, and a petroleum-based resin.

(Colorant)

Examples of the colorant to be incorporated into each toner particle of the toner of the present invention include the following colorants.

A black colorant is, for example, carbon black or a colorant toned to a black color with a yellow colorant, a magenta colorant, and a cyan colorant. Although one kind of pigment may be used alone as the colorant, a dye and a pigment are preferably used in combination to improve the color definition in terms of the image quality of a full-color image.

As a pigment for a magenta toner, there are given, for example: C.I. Pigment Red 1, 2, 3, 4, 5, 6, 7, 8, 9, 10, 11, 12, 13, 14, 15, 16, 17, 18, 19, 21, 22, 23, 30, 31, 32, 37, 38, 39, 40, 41, 48:2, 48:3, 48:4, 49, 50, 51, 52, 53, 54, 55, 57:1, 58, 60, 63, 64, 68, 81:1, 83, 87, 88, 89, 90, 112, 114, 122, 123, 146, 147, 150, 163, 184, 202, 206, 207, 209, 238, 269, or 282; C.I. Pigment Violet 19; and C.I. Vat Red 1, 2, 10, 13, 15, 23, 29, or 35.

As a dye for a magenta toner, there are given, for example: oil-soluble dyes such as: C.I. Solvent Red 1, 3, 8, 23, 24, 25, 27, 30, 49, 81, 82, 83, 84, 100, 109, or 121; C.I. Disperse Red

## 15

9; C.I. Solvent Violet 8, 13, 14, 21, or 27; and C.I. Disperse Violet 1; and basic dyes such as: C.I. Basic Red 1, 2, 9, 12, 13, 14, 15, 17, 18, 22, 23, 24, 27, 29, 32, 34, 35, 36, 37, 38, 39, or 40; and C.I. Basic Violet 1, 3, 7, 10, 14, 15, 21, 25, 26, 27, or 28.

As a pigment for a cyan toner, there are given, for example: C.I. Pigment Blue 2, 3, 15:2, 15:3, 15:4, 16, or 17; C.I. Vat Blue 6; C.I. Acid Blue 45; and a copper phthalocyanine pigment in which a phthalocyanine skeleton is substituted with 1 or more to 5 or less phthalimidomethyl groups.

C.I. Solvent Blue 70 is given as a dye for a cyan toner.

As a pigment for a yellow toner, there are given, for example: C.I. Pigment Yellow 1, 2, 3, 4, 5, 6, 7, 10, 11, 12, 13, 14, 15, 16, 17, 23, 62, 65, 73, 74, 83, 93, 94, 95, 97, 109, 110, 111, 120, 127, 128, 129, 147, 151, 154, 155, 168, 174, 175, 176, 180, 181, or 185; and C.I. Vat Yellow 1, 3, or 20.

C.I. Solvent Yellow 162 is given as a dye for yellow toner.

The colorant is preferably used in an amount of from 0.1 part by mass or more to 30 parts by mass or less with respect to 100 parts by mass of the binder resin.

(Additive)

A charge control agent may be incorporated into the toner of the present invention as required. Although a known charge control agent can be utilized as the charge control agent to be incorporated into the toner, a metal compound of an aromatic carboxylic acid that is colorless, increases the speed at which the toner is charged, and can stably hold a constant charge quantity is particularly preferred.

As a negative charge control agent, the following are given: a metal salicylate compound, a metal naphthoate compound, a metal dicarboxylate compound, a polymeric compound having a sulfonic acid or a carboxylic acid in a side chain, a polymeric compound having a sulfonic acid salt or a sulfonic acid ester in a side chain, a polymeric compound having a carboxylic acid salt or a carboxylic acid ester in a side chain, a boron compound, a urea compound, a silicon compound, and a calixarene. As a positive charge control agent, the following are given: a quaternary ammonium salt, a polymeric compound having a quaternary ammonium salt in a side chain, a guanidine compound, and an imidazole compound. The charge control agent may be internally added to each toner particle or may be externally added to the toner particle. The charge control agent is preferably added in an amount of from 0.2 part by mass or more to 10 parts by mass or less with respect to 100 parts by mass of the binder resin.

Inorganic fine particles can also be incorporated into the toner of the present invention as required. The inorganic fine particles may be internally added to the particles of the toner or may be mixed as an external additive with the toner particles. The external additive is preferably inorganic fine particles (inorganic fine powder) made of silica, titanium oxide, aluminum oxide, or the like. The inorganic fine particles are preferably hydrophobized with a hydrophobizing agent such as a silane compound, a silicone oil, or a mixture thereof.

An external additive for improving the flowability of the toner is preferably inorganic fine particles having a specific surface area of from 50 m<sup>2</sup>/g or more to 400 m<sup>2</sup>/g or less, and an external additive for stabilizing the durability of the toner is preferably inorganic fine particles having a specific surface area of from 10 m<sup>2</sup>/g or more to 50 m<sup>2</sup>/g or less. A plurality of kinds of inorganic fine particles whose specific surface areas fall within the ranges may be used in combination in order that compatibility between the improvement in the flowability of the toner and the stabilization of its durability may be achieved.

The external additive is preferably used in an amount of from 0.1 part by mass or more to 10.0 parts by mass or less

## 16

with respect to 100 parts by mass of the toner particles. A known mixer such as a Henschel mixer can be used in the mixing of the toner particles and the external additive.

(Two-Component Developer)

5 The toner of the present invention can be used as a one-component system developer. The toner is preferably mixed with a magnetic carrier and used as a two-component developer in order that its dot reproducibility may be additionally improved and a stable image may be obtained over a long time period.

(Magnetic Carrier)

15 Examples of the magnetic carrier include the following: an iron powder whose surface has been oxidized; an unoxidized iron powder; particles of metals such as iron, lithium, calcium, magnesium, nickel, copper, zinc, cobalt, manganese, chromium, and rare earths; particles of alloys thereof; magnetic materials such as oxide particles and ferrite; and a magnetic material-dispersed resin carrier (the so-called resin carrier) containing a magnetic material and a binder resin 20 holding the magnetic material in a state where the magnetic material is dispersed therein.

When the toner of the present invention is mixed with the magnetic carrier and used as a two-component developer, the concentration of the toner in the two-component developer is 25 preferably from 2 mass % or more to 15 mass % or less, more preferably from 4 mass % or more to 13 mass % or less.

(Method of Producing Toner)

30 A method of producing the toner particles is preferably a pulverization method involving melting and kneading the binder resin, the colorant, and the wax, cooling the kneaded product, and pulverizing and classifying the cooled product because the binder resin, the colorant, and the wax need to be melted and kneaded.

35 Hereinafter, an example of a procedure for the production of the toner by the pulverization method is described.

In a raw material-mixing step, predetermined amounts of 40 materials for forming the toner particles, e.g., a binder resin, a wax, a colorant, and other component such as a charge control agent to be used as required are weighed, blended, and mixed. As a mixing apparatus, there are given, for example, a double cone mixer, a V-type mixer, a drum-type mixer, a super mixer, a Henschel mixer, a Nauta mixer, and MECHANIC HYBRID (manufactured by NIPPON COKE & ENGINEERING CO., LTD.).

45 Next, the mixed materials are melted and kneaded to disperse the wax and the like in the binder resin. In the melting-kneading step, a batch kneader such as a pressurizing kneader or a Banbury mixer, or a continuous kneader can be used. A single-screw or a twin-screw extruder is a mainstream 50 because of the advantage of continuous production. Examples thereof include: a twin-screw extruder model KTK (manufactured by Kobe Steel., Ltd.); a twin-screw extruder model TEM (manufactured by Toshiba Machine CO., Ltd.); a PCM kneader (manufactured by Ikegai Corp.); a twin-screw 55 extruder (manufactured by KCK CO., Ltd.); a co-kneader (manufactured by Buss Inc.); and KNEADEX (NIPPON COKE & ENGINEERING CO., LTD.). Further, a resin composition obtained by melting and kneading may be rolled by a twin roll or the like, and cooled with water or the like in a 60 cooling step.

Next, a cooled product of the resin composition is pulverized to a desired particle diameter in a pulverizing step. In the pulverizing step, the cooled product is coarsely pulverized with a pulverizer such as a crusher, a hammer mill, or a feather mill, and is then finely pulverized with, for example, Kryptron System (manufactured by Kawasaki Heavy Industries, Ltd.), Super Rotor (manufactured by Nissin Engineering

Inc.), Turbo Mill (manufactured by FREUND-TURBO CORPORATION), or a fine pulverizer based on an air-jet system.

After that, as required, the resultant particles are classified with an inertial classification type classifier or sieving machine such as Elbow-Jet (manufactured by NITTETSU MINING CO., LTD), or a centrifugal type classifier or sieving machine such as Turboplex (manufactured by Hosokawa Micron Corporation), TSP Separator (manufactured by Hosokawa Micron Corporation), or Faculty (manufactured by Hosokawa Micron Corporation) to obtain a classified product (toner particles). Of those, Faculty (manufactured by Hosokawa Micron Corporation) can perform spheroidization treatment for the toner particles as well as classification and is preferred from the viewpoint of transfer efficiency.

In addition, after the pulverization, the surface treatment of the toner particles such as spheroidization treatment may be performed with Hybridization System (manufactured by NARA MACHINERY CO., LTD.), Mechanofusion System (manufactured by Hosokawa Micron Corporation), Faculty (manufactured by Hosokawa Micron Corporation), or Meteo-rainbow MR Type (manufactured by Nippon Pneumatic Mfg. Co., Ltd.) as required.

The treatment of the surfaces of the toner particles with heat is particularly preferred because the circularity of the toner can be easily increased and its transfer efficiency improves. In addition, the treatment is preferred because of the following reason: the wax is distributed in a large amount near the surfaces of the toner particles by the heating, and hence the wax exhibits its releasing effect in an additionally quick manner in a toner-fixing step and the hot offset resistance of the toner additionally improves. For example, the surfaces can be treated with hot air by using a heat spheroidization treatment apparatus illustrated in FIGURE.

In FIGURE, a mixture supplied in a constant amount by a raw material constant amount-supplying unit 1 is introduced into an introducing tube 3 placed on the central axis of a treatment chamber 6 by a compressed gas adjusted by a compressed gas-adjusting unit 2. The mixture that has passed the introducing tube is uniformly dispersed by a conical protruding member 4 provided in the central portion of a raw material-supplying unit, introduced into supplying tubes 5 radially extending in 8 directions, and introduced from a powder particle-supplying port 14 into the treatment chamber 6 where the mixture is thermally treated.

At this time, the flow of the mixture supplied to the treatment chamber is regulated by a regulating unit 9 for regulating the flow of a mixture, the unit being provided in the treatment chamber. Accordingly, the mixture supplied to the treatment chamber is thermally treated while swirling in the treatment chamber, and is then cooled.

Hot air for thermally treating the supplied mixture is supplied from a hot air inlet portion 7 of a hot air-supplying unit, and the hot air is introduced into the treatment chamber while being spirally swirled by a swirling member 13 for swirling the hot air. With regard to its construction, the swirling member 13 for swirling the hot air has a plurality of blades, and can control the swirl of the hot air depending on the number and angles of the blades. At this time, the bias of the hot air to be swirled can be reduced by a substantially conical distributing member 12. The temperature of the hot air to be supplied into the treatment chamber at a hot air outlet portion 11 of the hot air-supplying unit is preferably from 100°C. to 300°C. It is because of the following reason that the temperature at the outlet portion of the hot air-supplying unit preferably falls within the range: the toner particles can be uniformly subjected to a spheroidization treatment while the fusion and

coalescence of the toner particles due to excessive heating of the mixture are prevented, and the hot offset resistance improves.

Further, the thermally treated toner particles are cooled by cold air supplied from cold air-supplying units 8 (8-1, 8-2, and 8-3), and the temperature of the cold air supplied from the cold air-supplying units 8 is preferably from -20°C. to 30°C. When the temperature of the cold air falls within the range, the thermally treated toner particles can be efficiently cooled, and the fusion and coalescence of the thermally treated toner particles can be prevented without the inhibition of the uniform spheroidization treatment of the mixture. The absolute moisture content of the cold air is preferably from 0.5 g/m<sup>3</sup> or more to 15.0 g/m<sup>3</sup> or less. Next, the thermally treated toner particles that have been cooled are recovered by a recovering unit 10 placed at the lower end of the treatment chamber. It should be noted that the recovering unit is constituted as follows: its tip is provided with a blower (not shown), and the particles are sucked and conveyed by the blower.

In addition, the powder particle-supplying port is provided so that the swirling direction of the supplied mixture and the swirling direction of the hot air may be identical to each other, and the recovering unit is provided in the outer peripheral portion of the treatment chamber so as to maintain the swirling direction of the swirled powder particles. Further, the cold air supplied from the cold air-supplying units 8 is constituted so as to be supplied from the outer peripheral portion of the apparatus into the inner peripheral surface of the treatment chamber from a horizontal and tangential direction. The swirling direction of the toner supplied from the powder particle-supplying port, the swirling direction of the cold air supplied from the cold air-supplying unit, and the swirling direction of the hot air supplied from the hot air-supplying unit are identical to one another. Accordingly, no turbulence occurs in the treatment chamber, a swirl flow in the apparatus is strengthened, a strong centrifugal force is applied to the toner, and the dispersibility of the toner additionally improves, and hence a toner having a small amount of a coalesced particle and a uniform shape can be obtained.

The average circularity of the toner is preferably from 0.930 or more to 0.985 or less. In addition, when the toner particles are subjected to a surface treatment such as a spheroidization treatment or to a surface treatment by a heat treatment, the average circularity is preferably from 0.955 or more to 0.980 or less because compatibility between an improvement in transferability and cleaning property can be achieved.

Further, the surfaces of the toner particles are subjected to an external addition treatment with an external additive as required. A method for the external addition treatment with the external additive is, for example, a method involving blending predetermined amounts of a classified toner and various known external additives, and stirring and mixing the contents through the use of a mixing apparatus such as a double cone mixer, a V-type mixer, a drum-type mixer, a super mixer, a Henschel mixer, a Nauta mixer, MECHANIC HYBRID (manufactured by NIPPON COKE & ENGINEERING CO., LTD.), or NOBILTA (manufactured by Hosokawa Micron Corporation) as an external addition machine.

In addition, the external addition treatment with the external additive can be performed before a surface treatment by a heat treatment. This case is preferred because of the following reason. The external additive is stuck to the surfaces of the toner particles by the heat treatment and hence the surfaces of the toner particles are hardly shaved even by a stress due to long-term printing. Accordingly, even in a normal-temperature and low-humidity environment or a high-temperature

and high-humidity environment, a density fluctuation after the long-term printing is suppressed and fogging after the printing is alleviated.

Hereinafter, the present invention is described by way of examples and the like. Prior to the examples, methods of measuring the various physical properties of the toner and raw materials therefor, and production examples of its binder resin (the polyester resin A, the polyester resin B, and the polymer C) are described.

(Method of Measurement)

<1. Measurement of Softening Point of Resin>

The softening point of the resin is measured through use of a constant-pressure extrusion system capillary rheometer "flow characteristic-evaluating apparatus Flow Tester CFT-500D" (manufactured by Shimadzu Corporation) in accordance with the manual attached to the apparatus. In this apparatus, a measurement sample filled in a cylinder is increased in temperature to be melted while a predetermined load is applied to the measurement sample with a piston from above, and the melted measurement sample is extruded from a die in a bottom part of the cylinder. At this time, a flow curve representing a relationship between a piston descent amount and the temperature is obtained.

In the present invention, a "melting temperature in a 1/2 method" described in the manual attached to the apparatus is defined as a softening point. It should be noted that the melting temperature in the 1/2 method is calculated as described below. First, 1/2 of a difference between a descent amount Smax of the piston at a time when the outflow is finished and a descent amount Smin of the piston at a time when the outflow is started is determined (The 1/2 of the difference is defined as X. X=(Smax-Smin)/2). Then, the temperature in the flow curve when the descent amount of the piston reaches "Smin+X" in the flow curve is the melting temperature in the 1/2 method.

The measurement sample is obtained by subjecting about 1.0 g of the resin to compression molding for about seconds under about 10 MPa through use of a tablet compressing machine (for example, NT-100H, manufactured by NPa SYSTEM Co., Ltd.) under an environment of 25° C. to form the resin into a cylindrical shape having a diameter of about 8 mm.

The measurement conditions of the CFT-500D are as described below.

Test mode: heating method

Starting temperature: 50° C.

Reached temperature: 200° C.

Measurement interval: 1.0° C.

Rate of temperature increase: 4.0° C./min

Piston sectional area: 1.000 cm<sup>2</sup>

Test load (piston load): 10.0 kgf (0.9807 MPa)

Preheating time: 300 seconds

Diameter of hole of die: 1.0 mm

Length of die: 1.0 mm

<2. Measurement of Glass Transition Temperature (Tg (80), TG(180)) of Resin>

The glass transition temperature of the resin is measured with a differential scanning calorimeter "Q1000" (manufactured by TA Instruments) in conformity with ASTM D3418-82. The melting points of indium and zinc are used for the temperature correction of the detecting portion of the apparatus, and the heat of fusion of indium is used for the correction of a heat quantity.

Specifically, about 5 mg of the resin are precisely weighed and loaded into a pan made of aluminum, and then measurement is performed by using an empty pan made of aluminum as a reference in the measuring range of from 30 to 200° C. at

a rate of temperature increase of 10° C./min. It should be noted that in the measurement of Tg(80), the temperature of the resin is increased to 80° C. once and held at the temperature for 10 minutes. Subsequently, the temperature is reduced to 30° C. and then increased again. In the second temperature increase process, a change in specific heat is obtained in the temperature range of from 30 to 100° C. The point of intersection of a line, which connects the midpoints of baselines before and after the appearance of the change in specific heat,

10 and a differential thermal curve at this time is defined as the glass transition temperature (Tg(80)) of the resin. In addition, in the measurement of the Tg(180), the temperature of the resin is increased to 180° C. once and held at the temperature for 10 minutes, is subsequently reduced to 30° C., and is then increased again. In the second temperature increase process, 15 a change in specific heat is obtained in the temperature range of from 30 to 100° C. The point of intersection of a line, which connects the midpoints of baselines before and after the appearance of the change in specific heat, and a differential 20 thermal curve at this time is defined as the glass transition temperature (Tg(180)) of the resin.

<3. Measurement of Highest Endothermic Peak of Wax>

The peak temperature of the highest endothermic peak of the wax is measured with a differential scanning calorimeter "Q1000" (manufactured by TA Instruments) in conformity with ASTM D3418-82. The melting points of indium and zinc are used for the temperature correction of the detecting portion of the apparatus, and the heat of fusion of indium is used for the correction of a heat quantity.

Specifically, about 10 mg of the wax are precisely weighed and loaded into a pan made of aluminum, and then measurement is performed by using an empty pan made of aluminum as a reference in the measurement temperature range of from 30° C. or more to 200° C. or less at a rate of temperature 30 increase of 10° C./min. It should be noted that in the measurement, the temperature of the wax is increased to 200° C. once, is subsequently reduced to 30° C., and is then increased again. The temperature at which the DSC curve shows the highest endothermic peak in the temperature range of from 30° C. or more to 200° C. or less in the second temperature 40 increase process is defined as the peak temperature of the highest endothermic peak of the wax.

<4. Measurement of BET Specific Surface Area of Inorganic Fine Particles>

45 The BET specific surface area of inorganic fine particles is measured in conformity with JIS 28830 (2001). A specific measurement method is as described below.

Used as a measuring apparatus is an "automatic specific surface area/pore distribution-measuring apparatus TriStar 5000 (manufactured by Shimadzu Corporation)" adopting a gas adsorption method based on a constant volume method as a measurement system. The setting of a measurement condition and the analysis of measured data are performed with the dedicated software "TriStar 3000 Version 4.00" included with the apparatus. A vacuum pump, a nitrogen gas piping, and a helium gas piping are connected to the apparatus. A nitrogen gas is used as an adsorption gas and a value calculated by a BET multipoint method is defined as the BET specific surface area of the inorganic fine particles in the present invention.

60 It should be noted that the BET specific surface area is calculated as described below.

First, the inorganic fine particles are caused to adsorb the nitrogen gas, and an equilibrium pressure P (Pa) in a sample cell and a nitrogen adsorption amount V<sub>a</sub> (mol/g) of the external additive at that time are measured. Then, an adsorption isotherm is obtained, whose axis of abscissa indicates a relative pressure P<sub>r</sub> as a value obtained by dividing the equilib-

rium pressure  $P$  (Pa) in the sample cell by a saturated vapor pressure  $P_0$  (Pa) of nitrogen and whose axis of ordinate indicates the nitrogen adsorption amount  $V_a$  (mol/g). Next, a monomolecular layer adsorption amount  $V_m$  (mol/g) as an adsorption amount needed for forming a monomolecular layer on the surface of the external additive is determined by applying the following BET equation.

$$Pr/V_a(1-Pr) = 1/(V_m \times C) + (C-1) \times Pr/(V_m \times C)$$

Here,  $C$  represents a BET parameter and is a variable that varies depending on the kind of the measurement sample, the kind of the adsorption gas, and an adsorption temperature.

The BET equation can be interpreted as a straight line having a slope of  $(C-1)/(V_m \times C)$  and an intercept of  $1/(V_m \times C)$  when the X-axis indicates the  $Pr$  and the Y-axis indicates the  $Pr/V_a(1-Pr)$ . The straight line is referred to as "BET plot."

$$\text{Slope of straight line} = (C-1)/(V_m \times C)$$

$$\text{Intercept of straight line} = 1/(V_m \times C)$$

When an actual value for the  $Pr$  and an actual value for the  $Pr/V_a(1-Pr)$  are plotted on a graph, and a straight line is drawn by the method of least squares, values for the slope and intercept of the straight line can be calculated. The  $V_m$  and the  $C$  can be calculated by substituting those values into the mathematical expression and solving the resultant simultaneous equations.

Further, a BET specific surface area  $S$  ( $\text{m}^2/\text{g}$ ) of the inorganic fine particles is calculated from the  $V_m$  calculated here and a sectional area ( $0.162 \text{ nm}^2$ ) occupied by a nitrogen molecule based on the following equation.

$$S = V_m \times N \times 0.162 \times 10^{-18}$$

Here,  $N$  represents Avogadro's number ( $\text{mol}^{-1}$ ).

Although the measurement involving using the apparatus is in conformity with the "TriStar 3000 Instruction Manual V4.0" included with the apparatus, the measurement is specifically performed by the following procedure.

The tare mass of a dedicated sample cell made of a glass (having a stem diameter of  $\frac{3}{8}$  inch and a volume of about 5 ml) that has been sufficiently washed and dried is precisely weighed. Then, about 0.1 g of the external additive is loaded into the sample cell by using a funnel.

The sample cell into which the inorganic fine particles have been loaded is set in a "pretreatment apparatus VACUPREP 061 (manufactured by Shimadzu Corporation)" having connected thereto a vacuum pump and a nitrogen gas piping, and vacuum deaeration is continued for about 10 hours at  $23^\circ \text{C}$ . It should be noted that at the time of the vacuum deaeration, the inside of the sample cell is gradually deaerated while a valve is adjusted so that the inorganic fine particles may not be sucked by the vacuum pump. As the deaeration progresses, a pressure in the sample cell gradually reduces and finally reaches about 0.4 Pa (about 3 mmTorr). After the completion of the vacuum deaeration, a nitrogen gas is gradually injected into the sample cell to return the pressure in the sample cell to atmospheric pressure, and the sample cell is removed from the pretreatment apparatus. Then, the mass of the sample cell is precisely weighed, and the accurate mass of the external additive is calculated from a difference between the mass and the tare mass. It should be noted that at this time, the sample cell is lidded with a rubber stopper during the weighing so that the external additive in the sample cell may not be contaminated by, for example, moisture in the air.

Next, a dedicated "isothermal jacket" is attached to the stem portion of the sample cell containing the inorganic fine particles. Then, a dedicated filler rod is inserted into the

sample cell and the sample cell is set in the analysis port of the apparatus. It should be noted that the isothermal jacket is a tubular member that can take up liquid nitrogen to a certain level by virtue of capillarity, and has an inner surface constituted of a porous material and an outer surface constituted of an impervious material.

Subsequently, the free space of the sample cell including a connecting tool is measured. The free space is calculated by: measuring the volume of the sample cell at  $23^\circ \text{C}$ . with a helium gas; then similarly measuring the volume of the sample cell after the cooling of the sample cell with liquid nitrogen with a helium gas; and converting a difference between these volumes. In addition, the saturated vapor pressure  $P_0$  (Pa) of nitrogen is separately measured in an automatic manner with a  $P_0$  tube built in the apparatus.

Next, the inside of the sample cell is subjected to vacuum deaeration and then the sample cell is cooled with liquid nitrogen while the vacuum deaeration is continued. After that, a nitrogen gas is introduced into the sample cell in a stepwise manner and the toner is caused to adsorb a nitrogen molecule. At this time, the adsorption isotherm is obtained by measuring the equilibrium pressure  $P$  (Pa) whenever necessary and the adsorption isotherm is transformed into the BET plot. It should be noted that the number of points of the relative pressure  $Pr$  at which data is collected is set to a total of 6, i.e., 0.05, 0.10, 0.15, 0.20, 0.25, and 0.30. A straight line is drawn on the measured data thus obtained by the method of least squares, and the  $V_m$  is calculated from the slope and intercept of the straight line. Further, the BET specific surface area of the inorganic fine particles is calculated by using the value for the  $V_m$  as described above.

<5. Measurement of Weight-Average Particle Diameter (D4) of Toner Particles>

The weight-average particle diameter (D4) of the toner particles is measured with the number of effective measurement channels of 25,000 by using a precision particle size distribution-measuring apparatus based on a pore electrical resistance method provided with a  $100\text{-}\mu\text{m}$  aperture tube "Coulter Counter Multisizer 3" (trademark, manufactured by Beckman Coulter, Inc.) and dedicated software included therewith "Beckman Coulter Multisizer 3 Version 3.51" (manufactured by Beckman Coulter, Inc.) for setting measurement conditions and analyzing measurement data. Then, the measurement data is analyzed to calculate the diameter.

An electrolyte aqueous solution prepared by dissolving guaranteed sodium chloride in deionized water so as to have a concentration of about 1 mass %, for example, "ISOTON II" (manufactured by Beckman Coulter, Inc.) can be used in the measurement.

It should be noted that the dedicated software is set as described below prior to the measurement and the analysis.

In the "change standard measurement method (SOM)" screen of the dedicated software, the total count number of a control mode is set to 50,000 particles, the number of times of measurement is set to 1, and a value obtained by using "standard particles each having a particle diameter of  $10.0 \text{ }\mu\text{m}$ " (manufactured by Beckman Coulter, Inc.) is set as a  $K_d$  value. A threshold and a noise level are automatically set by pressing a threshold/noise level measurement button. In addition, a current is set to  $1,600 \text{ pA}$ , a gain is set to 2, and an electrolyte solution is set to "ISOTON II", and a check mark is placed in a check box as to whether the aperture tube is flushed after the measurement.

In the "setting for conversion from pulse to particle diameter" screen of the dedicated software, a bin interval is set to a logarithmic particle diameter, the number of particle diam-

eter bins is set to 256, and a particle diameter range is set to the range of from 2  $\mu\text{m}$  or more to 60  $\mu\text{m}$  or less.

A specific measurement method is as described below in sections (1) to (7).

(1) About 200 ml of the electrolyte aqueous solution are charged into a 250-ml round-bottom beaker made of glass dedicated for the Multisizer 3. The beaker is set in a sample stand, and the electrolyte aqueous solution in the beaker is stirred with a stirrer rod at 24 rotations/sec in a counterclockwise direction. Then, dirt and bubbles in the aperture tube are removed by the "aperture flush" function of the analytical software.

(2) About 30 ml of the electrolyte aqueous solution are charged into a 100-ml flat-bottom beaker made of glass. About 0.3 ml of a diluted solution prepared by diluting "Contaminon N" (a 10 mass % aqueous solution of a neutral detergent for washing a precision measuring device formed of a nonionic surfactant, an anionic surfactant, and an organic builder and having a pH of 7 manufactured by Wako Pure Chemical Industries, Ltd.) with deionized water by three mass fold is added as a dispersant to the electrolyte aqueous solution.

(3) In an ultrasonic dispersing unit, two oscillators each having an oscillatory frequency of 50 kHz are built so as to be out of phase by 180°. A predetermined amount of deionized water is charged into the water tank of the ultrasonic dispersing unit "Ultrasonic Dispersion System Tetora 150" (manufactured by Nikkaki Bios Co., Ltd.) having an electrical output of 120 W. About 2 ml of the "Contaminon N" are charged into the water tank.

(4) The beaker in the section (2) is set in the beaker fixing hole of the ultrasonic dispersing unit, and the ultrasonic dispersing unit is operated. Then, the height position of the beaker is adjusted in order that the liquid level of the electrolyte aqueous solution in the beaker may resonate with an ultrasonic wave from the ultrasonic dispersing unit to the fullest extent possible.

(5) About 10 mg of toner are gradually added to and dispersed in the electrolyte aqueous solution in the beaker in the section (4) in a state in which the electrolyte aqueous solution is irradiated with the ultrasonic wave. Then, the ultrasonic dispersion treatment is continued for an additional 60 seconds. It should be noted that the temperature of water in the water tank is adjusted so as to be from 10° C. or more to 40° C. or less upon ultrasonic dispersion.

(6) The electrolyte aqueous solution in the section (5) in which the toner has been dispersed is dropped with a pipette to the round-bottom beaker in the section (1) placed in the sample stand, and the concentration of the toner to be measured is adjusted to about 5%. Then, measurement is performed until the particle diameters of 50,000 particles are measured.

(7) The measurement data is analyzed with the dedicated software included with the apparatus, and the weight-average particle diameter (D4) is calculated. It should be noted that an "average diameter" on the "analysis/volume statistics (arithmetic average)" screen of the dedicated software when the dedicated software is set to show a graph in a vol % unit is the weight-average particle diameter (D4).

#### <6. Measurement of Average Circularity of Toner>

The average circularity of the toner is measured under measurement and analysis conditions at the time of calibration operation with a flow-type particle image analyzer "FPIA-3000" (manufactured by Sysmex Corporation).

The measurement principle of the flow-type particle image analyzer "FPIA-3000" (manufactured by Sysmex Corporation) is as follows: a flowing particle is photographed as a

static image and the image is analyzed. A sample loaded into a sample chamber is fed into a flat sheath flow cell by a sample suction syringe. The sample fed into the flat sheath flow cell is sandwiched between sheath liquids to form a flat flow. The sample passing the inside of the flat sheath flow cell is irradiated with strobe light at an interval of 1/60 second, and hence the flowing particle can be photographed as the static image. In addition, the particle is photographed in a state of being in focus because the flow is flat. The particle image is taken with a CCD camera, the taken image is subjected to image processing at an image processing resolution of 512×512 pixels (0.37×0.37  $\mu\text{m}$  per pixel), the borders of the respective particle images are sampled, and a projected area S, perimeter L, and the like of each particle image are measured.

Next, a circle-equivalent diameter and a circularity are determined by using the area S and the perimeter L. The circle-equivalent diameter refers to the diameter of a circle having the same area as the projected area of a particle image, and the circularity C is defined as a value obtained by dividing the perimeter of a circle determined from the circle-equivalent diameter by the perimeter of a particle projected image and is calculated from the following equation.

$$\text{Circularity } C=2\times(\pi\times S)^{1/2}/L$$

When a particle image is circular, its circularity becomes 1.000. As the degree of unevenness of the outer periphery of the particle image enlarges, the value for the circularity reduces. After the circularity of each particle has been calculated, the circularity range of from 0.200 to 1.000 is divided into 800 sections, the arithmetic average of the resultant circularities is calculated, and the value is defined as an average circularity.

A specific measurement method is as described below. First, about 20 ml of ion-exchanged water from which an impure solid and the like have been removed in advance are charged into a container made of a glass. About 0.2 ml of a diluted solution prepared by diluting "Contaminon N" with deionized water by about three mass fold is added as a dispersant to the container. Further, about 0.02 g of a measurement sample is added to the container, and then the mixture is subjected to a dispersion treatment with an ultrasonic dispersing unit for 2 minutes so that a dispersion liquid for measurement may be obtained. At that time, the dispersion liquid is appropriately cooled so as to have a temperature of 10° C. or more to 40° C. or less. A desktop ultrasonic cleaning and dispersing unit having an oscillatory frequency of 50 kHz and an electrical output of 150 W (such as "VS-150" (manufactured by VELVO-CLEAR)) is used as the ultrasonic dispersing unit. A predetermined amount of deionized water is charged into a water tank, and about 2 ml of the Contaminon N are added to the water tank.

The flow-type particle image analyzer mounted with a standard objective lens (magnification: 10) is used in the measurement, and a particle sheath "PSE-900A" (manufactured by Sysmex Corporation) is used as a sheath liquid. The dispersion liquid prepared in accordance with the procedure is introduced into the flow-type particle image analyzer, and 3,000 toner particles are subjected to measurement according to the total count mode of an HPF measurement mode. Then, the number percentage (%) and average circularity of the toner particles in the range can be calculated by setting a binarization threshold at the time of particle analysis to 85% and specifying particle diameters to be analyzed. The average circularity of the toner is determined by limiting to one corresponding to a circle-equivalent diameter of 1.98  $\mu\text{m}$  or more to 39.69  $\mu\text{m}$  or less.

25

On the measurement, automatic focusing is performed with standard latex particles (obtained by diluting, for example, "RESEARCH AND TEST PARTICLES Latex Microsphere Suspensions 5200A" manufactured by Duke Scientific with deionized water) prior to the initiation of the measurement. After that, focusing is preferably performed every two hours from the initiation of the measurement.

It should be noted that in this example, a flow-type particle image analyzer which had been subjected to a calibration operation by Sysmex Corporation and received a calibration certificate issued by Sysmex Corporation was used. The measurement was performed under measurement and analysis conditions identical to those at the time of the reception of the calibration certificate except that particle diameters to be analyzed were limited to ones each corresponding to a circle-equivalent diameter of 1.98  $\mu\text{m}$  or more to less than 39.69  $\mu\text{m}$ .

<7. Measurement of Acid Value of Resin>

The acid value of a polyester resin is measured by the following method. The acid value refers to the number of milligrams of potassium hydroxide needed for neutralizing an acid in 1 g of a sample. The acid value of the polyester resin is measured in conformity with JIS K 0070-1992. Specifically, the measurement is performed by the following procedure.

(1) Preparation of Reagent

1.0 Gram of phenolphthalein is dissolved in 90 ml of ethyl alcohol (95 vol %) and deionized water is added to the solution to increase its volume to 100 ml. Thus, a phenolphthalein solution is obtained.

7 Grams of special grade potassium hydroxide are dissolved in 5 ml of deionized water and ethyl alcohol (95 vol %) is added to the solution to increase its volume to 1 liter. The solution is charged into an alkali-resistant container so as to be out of contact with a carbon dioxide gas or the like, and is left to stand for 3 days. After that, the solution is filtered to provide a potassium hydroxide solution. The resultant potassium hydroxide solution is stored in an alkali-resistant container. The factor of the potassium hydroxide solution is determined as follows: 25 ml of a 0.1 mol/l hydrochloric acid are taken in an Erlenmeyer flask, several droplets of the phenolphthalein solution are added to the flask, the hydrochloric acid is titrated with the potassium hydroxide solution, and the amount of the potassium hydroxide solution needed for neutralization is used in the determination. A hydrochloric acid produced in conformity with JIS K 8001-1998 is used as the 0.1 mol/l hydrochloric acid.

(2) Operation

(A) Main Test

2.0 Grams of a sample of a pulverized polyester resin are precisely weighed in a 200-ml Erlenmeyer flask, and 100 ml of a mixed solution containing toluene and ethanol at a ratio of 2:1 are added to dissolve the sample over 5 hours. Next, several droplets of the phenolphthalein solution are added as an indicator and the solution is titrated with the potassium hydroxide solution. It should be noted that the end point of the titration is defined as the point at which the light pink color of the indicator continues for about 30 seconds.

(B) Blank Test

The same titration as the foregoing operations is performed except that no sample is used (i.e., only the mixed solution containing toluene and ethanol at a ratio of 2:1 is used).

(3) The acid value is calculated by substituting the obtained result into the following equation.

$$A = [(C-B) \times f \times 5.61] / S$$

Here, A represents the acid value (mgKOH/g), B represents the addition amount (ml) of the potassium hydroxide solution

26

in the blank test, C represents the addition amount (ml) of the potassium hydroxide solution in the main test, f represents the factor of the potassium hydroxide solution, and S represents the sample (g).

5 (Production Example of Binder Resin)

PRODUCTION EXAMPLE A1

56.2 Parts by mass (0.158 mol: 97 mol % with respect to the total number of moles of polyhydric alcohols) of a polyoxypropylene(2.2)-2,2-bis(4-hydroxyphenyl)propane, 16.9 parts by mass (0.102 mol: 55 mol % with respect to the total number of moles of polyvalent carboxylic acids) of terephthalic acid, 1.1 parts by mass (0.0016 mol: 3 mol % with respect to the total number of moles of the polyhydric alcohols) of a novolac type phenol resin (adduct with 5 mol of ethylene oxide having a nucleus number of about 5), 6.4 parts by mass (0.044 mol: 25 mol % with respect to the total number of moles of the polyvalent carboxylic acids) of adipic acid, and 0.6 part by mass of titanium tetrabutoxide were loaded into a 4-liter four-necked flask made of a glass. Then, a temperature gauge, a stirring rod, a condenser, and a nitrogen-introducing tube were attached to the four-necked flask, and the four-necked flask was placed in a mantle heater. Next, an atmosphere in the flask was replaced with a nitrogen gas, and then a temperature in the flask was gradually increased while the contents were stirred. The contents were subjected to a reaction for 2 hours while being stirred at a temperature of 200° C. (first reaction step). After that, 5.8 parts by mass (0.030 mol: 20 mol % with respect to the total number of moles of the polyvalent carboxylic acids) of trimellitic anhydride were added to the resultant, and the mixture was subjected to a reaction at 180° C. for 10 hours (second reaction step). Thus, a polyester resin A1 was obtained.

The polyester resin A1 had a softening point of 150° C. and an acid value of 20 mgKOH/g. In addition, the resin had a Tg(80) of 60.0° C. and a Tg(180) of 59.8° C. Table 1 shows components constituting the polyhydric alcohol unit of the polyester resin A1 and components constituting the polyvalent carboxylic acid unit thereof. In addition, Table 2 shows the physical properties of the polyester resin A1.

PRODUCTION EXAMPLE A2

A polyester resin A2 was obtained by performing a reaction in the same manner as in Production Example A1 except that in the second reaction step, after the addition of trimellitic anhydride, the pressure in the flask was reduced to from 500 Pa or more to 2,000 Pa or less, and the reaction was performed at 160° C. for 5 hours. Table 2 shows the physical properties of the polyester resin A2.

PRODUCTION EXAMPLES A3 TO A6, A20, AND A21

Polyester resins A3 to A6, A20, and A21 were each obtained by performing a reaction in the same manner as in Production Example A1 except that the reaction time for the second reaction step was changed.

PRODUCTION EXAMPLES A7 TO A11, A22, AND A23

Polyester resins A7 to A11, A22, and A23 were each obtained by performing a reaction in the same manner as in Production Example A1 except that the polyhydric alcohol components used in the first reaction step and their molar

27

ratios were changed as shown in Table 1. At that time, the number of parts by mass of each raw material was adjusted so that the total number of moles of the polyhydric alcohols became equal to that of Production Example A1.

#### PRODUCTION EXAMPLES A12 TO A17 AND A24 to A27

Polyester resins A12 to A17 and A24 to A27 were each obtained by performing a reaction in the same manner as in Production Example A1 except that the polyvalent carboxylic acid components used in the first reaction step and their molar ratios were changed as shown in Table 1. At that time, the number of parts by mass of each raw material was adjusted so that the total number of moles of the polyvalent carboxylic acids became equal to that of Production Example A1.

#### PRODUCTION EXAMPLE A18

A polyester resin A18 was obtained by performing a reaction in the same manner as in Production Example A1 except that: the polyvalent carboxylic acid components used in the first reaction step and the second reaction step, and their molar ratios were changed as shown in Table 1; and the reaction time for the second reaction step was changed to 12 hours. At that time, the number of parts by mass of each raw material was adjusted so that the total number of moles of the polyvalent carboxylic acids became equal to that of Production Example A1.

#### PRODUCTION EXAMPLE A19

A polyester resin A19 was obtained by performing a reaction in the same manner as in Production Example A1 except that: the polyvalent carboxylic acid components used in the first reaction step and the second reaction step, and their molar ratios were changed as shown in Table 1; and the reaction time for the second reaction step was changed to 7 hours. At that time, the number of parts by mass of each raw material was adjusted so that the total number of moles of the polyvalent carboxylic acids became equal to that of Production Example A1.

#### PRODUCTION EXAMPLE B1

59.3 Parts by mass (0.167 mol: 100 mol % with respect to the total number of moles of polyhydric alcohols) of a polyoxypropylene(2.2)-2,2-bis(4-hydroxyphenyl)propane, 24.2 parts by mass (0.146 mol: 94 mol % with respect to the total number of moles of polyvalent carboxylic acids) of terephthalic acid, 0.48 part by mass (0.0016 mol: 1 mol % with respect to the total number of moles of the polyvalent carboxylic acids) of fumaric acid, and 0.5 part by mass of titanium tetrabutoxide were loaded into a 4-liter four-necked flask made of a glass. Then, a temperature gauge, a stirring rod, a condenser, and a nitrogen-introducing tube were attached to the four-necked flask, and the four-necked flask was placed in a mantle heater. Next, an atmosphere in the flask was replaced with a nitrogen gas, and then a temperature

28

in the flask was gradually increased while the contents were stirred. The contents were subjected to a reaction for 4 hours while being stirred at a temperature of 200° C. (first reaction step). After that, 1.6 parts by mass (0.008 mol: 5 mol % with respect to the total number of moles of the polyvalent carboxylic acids) of trimellitic anhydride were added to the resultant, and the mixture was subjected to a reaction at 180° C. for 1 hour (second reaction step). Thus, a polyester resin B1 was obtained.

The polyester resin B1 had a softening point of 90° C. and an acid value of 6 mgKOH/g. In addition, the resin had a Tg(80) of 56.0° C. and a Tg(180) of 56.0° C. Table 1 shows the polyhydric alcohol components constituting the polyhydric alcohol unit of the polyester resin B1 and the polyvalent carboxylic acid components constituting the polyvalent carboxylic acid unit thereof. Table 2 shows the physical properties of the polyester resin B1.

#### PRODUCTION EXAMPLES B2 TO B5, B7, AND B15

Polyester resins B2 to B5, B7, and B15 were each obtained by performing a reaction in the same manner as in Production Example B1 except that the polyvalent carboxylic acid components used in the first reaction step and their molar ratios were changed as shown in Table 1. At that time, the number of parts by mass of each raw material was adjusted so that the total number of moles of the polyvalent carboxylic acids became equal to that of Production Example B1.

#### PRODUCTION EXAMPLES B6 AND B12

Polyester resins B6 and B12 were each obtained by performing a reaction in the same manner as in Production Example B1 except that: the polyvalent carboxylic acid components used in the first reaction step and their molar ratios were changed as shown in Table 1; and the second reaction step was not performed. At that time, the number of parts by mass of each raw material was adjusted so that the total number of moles of the polyvalent carboxylic acids became equal to that of Production Example B1.

#### PRODUCTION EXAMPLES B8 TO B11, B13, AND B14

Polyester resins B8 to B11, B13, and B14 were each obtained by performing a reaction in the same manner as in Production Example B1 except that the reaction time for the first reaction step was changed.

#### PRODUCTION EXAMPLE B16

Polyester resin B16 was obtained by performing a reaction in the same manner as in Production Example B1 except that the polyhydric alcohol components used in the first reaction step and their molar ratios were changed as shown in Table 1. At that time, the number of parts by mass of each raw material was adjusted so that the total number of moles of the polyhydric alcohols became equal to that of Production Example B1.

TABLE 1

| Polyester resin | Polyhydric alcohol component (mol %) |     |       |      | Polyvalent carboxylic acid component (mol %) |    |     |     |               |     |     |       |
|-----------------|--------------------------------------|-----|-------|------|----------------------------------------------|----|-----|-----|---------------|-----|-----|-------|
|                 | component (mol %)                    |     |       |      | Second reaction step                         |    |     |     |               |     |     |       |
|                 | First reaction step                  |     |       |      | First reaction step                          |    |     |     | reaction step |     |     |       |
| BPA-PO          | NBP                                  | EG  | Total | TPA  | SUA                                          | AA | SEA | TDA | ODA           | FA  | TMA | Total |
| A1              | 97                                   | 3   | 100   | 55   | 25                                           |    |     |     |               |     | 20  | 100   |
| A2              | 97                                   | 3   | 100   | 55   | 25                                           |    |     |     |               |     | 20  | 100   |
| A3              | 97                                   | 3   | 100   | 55   | 25                                           |    |     |     |               |     | 20  | 100   |
| A4              | 97                                   | 3   | 100   | 55   | 25                                           |    |     |     |               |     | 20  | 100   |
| A5              | 97                                   | 3   | 100   | 55   | 25                                           |    |     |     |               |     | 20  | 100   |
| A6              | 97                                   | 3   | 100   | 55   | 25                                           |    |     |     |               |     | 20  | 100   |
| A7              | 99                                   | 1   | 100   | 55   | 25                                           |    |     |     |               |     | 20  | 100   |
| A8              | 99.5                                 | 0.5 | 100   | 55   | 25                                           |    |     |     |               |     | 20  | 100   |
| A9              | 99.8                                 | 0.2 | 100   | 55   | 25                                           |    |     |     |               |     | 20  | 100   |
| A10             | 99.9                                 | 0.1 | 100   | 55   | 25                                           |    |     |     |               |     | 20  | 100   |
| A11             | 90                                   | 10  | 100   | 55   | 25                                           |    |     |     |               |     | 20  | 100   |
| A12             | 97                                   | 3   | 100   | 65   | 15                                           |    |     |     |               |     | 20  | 100   |
| A13             | 97                                   | 3   | 100   | 45   | 35                                           |    |     |     |               |     | 20  | 100   |
| A14             | 97                                   | 3   | 100   | 30   | 50                                           |    |     |     |               |     | 20  | 100   |
| A15             | 97                                   | 3   | 100   | 55   |                                              | 25 |     |     |               |     | 20  | 100   |
| A16             | 97                                   | 3   | 100   | 55   |                                              | 25 |     |     |               |     | 20  | 100   |
| A17             | 97                                   | 3   | 100   | 55   |                                              |    | 25  |     |               |     | 20  | 100   |
| A18             | 97                                   | 3   | 100   | 65   | 25                                           |    |     |     |               |     | 10  | 100   |
| A19             | 97                                   | 3   | 100   | 45   | 25                                           |    |     |     |               |     | 30  | 100   |
| A20             | 97                                   | 3   | 100   | 55   | 25                                           |    |     |     |               |     | 20  | 100   |
| A21             | 97                                   | 3   | 100   | 55   | 25                                           |    |     |     |               |     | 20  | 100   |
| A22             | 100                                  | 0   | 100   | 55   | 25                                           |    |     |     |               |     | 20  | 100   |
| A23             | 85                                   | 15  | 100   | 55   | 25                                           |    |     |     |               |     | 20  | 100   |
| A24             | 97                                   | 3   | 100   | 80   |                                              |    |     |     |               |     | 20  | 100   |
| A25             | 97                                   | 3   | 100   | 70   | 10                                           |    |     |     |               |     | 20  | 100   |
| A26             | 97                                   | 3   | 100   | 20   | 60                                           |    |     |     |               |     | 20  | 100   |
| A27             | 97                                   | 3   | 100   | 55   | 25                                           |    |     |     |               |     | 20  | 100   |
| B1              | 100                                  |     | 100   | 94   |                                              |    |     |     |               | 1   | 5   | 100   |
| B2              | 100                                  |     | 100   | 94.5 |                                              |    |     |     |               | 0.5 | 5   | 100   |
| B3              | 100                                  |     | 100   | 94.8 |                                              |    |     |     |               | 0.2 | 5   | 100   |
| B4              | 100                                  |     | 100   | 94.9 |                                              |    |     |     |               | 0.1 | 5   | 100   |
| B5              | 100                                  |     | 100   | 92   |                                              |    |     |     |               | 3   | 5   | 100   |
| B6              | 100                                  |     | 100   | 90   |                                              |    |     |     |               | 10  |     | 100   |
| B7              | 100                                  |     | 100   | 95   |                                              |    |     |     |               |     | 5   | 100   |
| B8              | 100                                  |     | 100   | 95   |                                              |    |     |     |               |     | 5   | 100   |
| B9              | 100                                  |     | 100   | 95   |                                              |    |     |     |               |     | 5   | 100   |
| B10             | 100                                  |     | 100   | 95   |                                              |    |     |     |               |     | 5   | 100   |
| B11             | 100                                  |     | 100   | 95   |                                              |    |     |     |               |     | 5   | 100   |
| B12             | 100                                  |     | 100   | 100  |                                              |    |     |     |               |     |     | 100   |
| B13             | 100                                  |     | 100   | 94   |                                              |    |     |     |               | 1   | 5   | 100   |
| B14             | 100                                  |     | 100   | 94   |                                              |    |     |     |               | 1   | 5   | 100   |
| B15             | 80                                   | 20  | 100   | 94   |                                              |    |     |     |               | 1   | 5   | 100   |
| B16             | 100                                  |     | 100   | 80   |                                              |    |     |     |               | 15  | 5   | 100   |

BPA-PO propylene oxide adduct of bisphenol A (average addition number of moles: 2.2 mol)

NBP novolac type phenol resin (adduct with 5 mol of ethylene oxide having a nucleus number of about 5)

EG ethylene glycol

TPA terephthalic acid

SUA succinic acid

AA adipic acid

SEA sebaciec acid

TDA tetradecanedioic acid

ODA octadecanedioic acid

FA fumaric acid

TMA trimellitic anhydride

TABLE 2

TABLE 2-continued

| Polyester resin | Softening point | Tg(80)   | Tg(180)  | Acid value       |          | Polyester resin | Softening point | Tg(80)   | Tg(180)  | Acid value       |          |
|-----------------|-----------------|----------|----------|------------------|----------|-----------------|-----------------|----------|----------|------------------|----------|
|                 |                 |          |          | Tg(80) - Tg(180) | [mg/KOH] |                 |                 |          |          | Tg(80) - Tg(180) | [mg/KOH] |
| A1              | 150° C.         | 60.0° C. | 59.8° C. | 0.2° C.          | 20       | A8              | 150° C.         | 59.8° C. | 59.0° C. | 0.8° C.          | 20       |
| A2              | 150° C.         | 61.0° C. | 59.8° C. | 1.2° C.          | 20       | A9              | 150° C.         | 59.6° C. | 59.0° C. | 0.6° C.          | 20       |
| A3              | 140° C.         | 59.4° C. | 59.0° C. | 0.4° C.          | 20       | A10             | 150° C.         | 59.6° C. | 59.0° C. | 0.6° C.          | 20       |
| A4              | 125° C.         | 53.6° C. | 53.2° C. | 0.4° C.          | 20       | A11             | 150° C.         | 61.2° C. | 60.8° C. | 0.4° C.          | 20       |
| A5              | 160° C.         | 60.4° C. | 60.2° C. | 0.2° C.          | 20       | A12             | 150° C.         | 59.6° C. | 59.4° C. | 0.2° C.          | 20       |
| A6              | 175° C.         | 64.2° C. | 63.8° C. | 0.4° C.          | 20       | 65 A13          | 150° C.         | 59.2° C. | 59.0° C. | 0.2° C.          | 20       |
| A7              | 150° C.         | 59.8° C. | 59.4° C. | 0.4° C.          | 20       | A14             | 150° C.         | 58.8° C. | 59.0° C. | -0.2° C.         | 20       |

TABLE 2-continued

| Polyester resin | Softening point | Tg(80)   | Tg(180)  | Tg(80) - Tg(180) | Acid value [mg/KOH] |
|-----------------|-----------------|----------|----------|------------------|---------------------|
| A15             | 150° C.         | 58.4° C. | 58.8° C. | -0.4° C.         | 20                  |
| A16             | 150° C.         | 57.8° C. | 58.2° C. | -0.4° C.         | 20                  |
| A17             | 150° C.         | 58.0° C. | 57.8° C. | 0.2° C.          | 20                  |
| A18             | 150° C.         | 58.4° C. | 58.2° C. | 0.2° C.          | 8                   |
| A19             | 150° C.         | 60.2° C. | 60.2° C. | 0.0° C.          | 50                  |
| A20             | 115° C.         | 53.0° C. | 52.8° C. | 0.2° C.          | 20                  |
| A21             | 185° C.         | 66.2° C. | 65.8° C. | 0.4° C.          | 20                  |
| A22             | 150° C.         | 61.2° C. | 61.2° C. | 0.0° C.          | 20                  |
| A23             | 150° C.         | 59.8° C. | 59.6° C. | 0.2° C.          | 20                  |
| A24             | 150° C.         | 60.4° C. | 59.6° C. | 0.8° C.          | 20                  |
| A25             | 150° C.         | 61.4° C. | 61.0° C. | 0.4° C.          | 20                  |
| A26             | 150° C.         | 59.6° C. | 58.8° C. | 0.8° C.          | 20                  |
| A27             | 150° C.         | 60.4° C. | 59.8° C. | 0.6° C.          | 20                  |
| B1              | 90° C.          | 56.0° C. | 56.0° C. | 0.0° C.          | 6                   |
| B2              | 90° C.          | 56.0° C. | 56.0° C. | 0.0° C.          | 6                   |
| B3              | 90° C.          | 56.0° C. | 56.0° C. | 0.0° C.          | 6                   |
| B4              | 90° C.          | 56.0° C. | 56.0° C. | 0.0° C.          | 6                   |
| B5              | 90° C.          | 55.6° C. | 55.6° C. | 0.0° C.          | 6                   |
| B6              | 90° C.          | 55.0° C. | 55.0° C. | 0.0° C.          | 2                   |
| B7              | 90° C.          | 56.0° C. | 56.0° C. | 0.0° C.          | 6                   |
| B8              | 86° C.          | 53.4° C. | 53.4° C. | 0.0° C.          | 6                   |
| B9              | 82° C.          | 50.8° C. | 50.8° C. | 0.0° C.          | 6                   |
| B10             | 94° C.          | 57.2° C. | 57.2° C. | 0.0° C.          | 6                   |
| B11             | 99° C.          | 61.2° C. | 61.2° C. | 0.0° C.          | 6                   |
| B12             | 90° C.          | 55.6° C. | 55.6° C. | 0.0° C.          | 2                   |
| B13             | 77° C.          | 49.4° C. | 49.4° C. | 0.0° C.          | 6                   |
| B14             | 103° C.         | 65.6° C. | 65.6° C. | 0.0° C.          | 6                   |
| B15             | 90° C.          | 54.6° C. | 54.6° C. | 0.0° C.          | 6                   |
| B16             | 90° C.          | 54.2° C. | 54.2° C. | 0.0° C.          | 6                   |

## PRODUCTION EXAMPLE C1

Materials shown in Table 3 below were loaded into an autoclave having a volume of 4 L and an atmosphere in the system was replaced with nitrogen. After that, a temperature in the system was increased and held at 180° C. while the materials were stirred. 50 Parts by mass of a 2 mass % solution of di-tert-butyl peroxide in xylene were continuously dropped to the system for 5 hours and the mixture was cooled. After that, the solvent was separated and removed. Thus, a polymer C1 in which a copolymer was grafted to the polyethylene was obtained. The polymer C1 had a softening point (Tm) of 110° C. and a glass transition temperature (Tg) of 64° C., and the weight-average molecular weight (Mw) and number-average molecular weight (Mn) of the THF soluble matter of the polymer C1 measured by GPC were 7,400 and 2,800, respectively. No peak corresponding to the polyethylene having one or more unsaturated bonds as a raw material was observed.

TABLE 3

| Material                                                                                                            | Part(s) by mass |
|---------------------------------------------------------------------------------------------------------------------|-----------------|
| Polyethylene having one or more unsaturated bonds (Mw: 1,400, Mn: 850, endothermic peak measured with DSC: 100° C.) | 20              |
| Styrene                                                                                                             | 59              |
| n-Butyl acrylate                                                                                                    | 18.5            |
| Acrylonitrile                                                                                                       | 2.5             |

## EXAMPLE 1

Materials shown in Table 4 below were mixed with a Henschel mixer (Model FM-75 manufactured by NIPPON COKE & ENGINEERING CO., LTD.) at a number of rotations of 20

rotations/sec for a time of rotation of 5 minutes. After that, the mixture was kneaded with a twin-screw extruder (Model PCM-30 manufactured by Ikegai Corporation) whose temperature had been set to 130° C.

TABLE 4

| Material | Part(s) by mass                                                        |
|----------|------------------------------------------------------------------------|
| 10       | Polyester resin A1                                                     |
|          | Polyester resin B1                                                     |
|          | Polymer C1                                                             |
|          | Hydrocarbon wax (peak temperature of highest endothermic peak: 78° C.) |
|          | C.I. Pigment Blue 15:3                                                 |
|          | Aluminum compound of 3,5-di-t-butylsalicylic acid                      |

The resultant kneaded product was cooled and coarsely pulverized with a hammer mill to 1 mm or less to provide a 20 coarsely pulverized product. The resultant coarsely pulverized product was finely pulverized with a mechanical pulverizer (T-250 manufactured by FREUND-TURBO CORPORATION). Further, the finely pulverized product was classified with a Faculty F-300 (manufactured by Hosokawa B7 Micron Corporation) to provide toner particles. Its operating conditions were as follows: the number of rotations of a classification rotor was set to 130 rotations/sec and the number of rotations of a dispersion rotor was set to 120 rotations/sec.

30 4.0 Parts by mass of hydrophobic silica fine particles subjected to a surface treatment with 4 mass % of hexamethyldisilazane and having a BET specific surface area of 25 m<sup>2</sup>/g, and 0.5 part by mass of titanium oxide fine particles subjected to a surface treatment with 16 mass % of isobutyltrimethoxysilane and having a BET specific surface area of 180 m<sup>2</sup>/g were added to 100 parts by mass of the toner particles, and the contents were mixed with a Henschel mixer (Model FM-75 manufactured by NIPPON COKE & ENGINEERING CO., LTD.) at a number of rotations of 30 rotations/sec for a time of rotation of 10 minutes. The toner particles were thermally treated with the surface treatment apparatus illustrated in

35 FIGURE to provide thermally treated toner particles. Its operating conditions were as follows: a feeding amount was set to 5 kg/hr, a hot air temperature was set to 210° C., a hot air flow rate was set to 6 m<sup>3</sup>/min, a cold air temperature was set to 5° C., a cold air flow rate was set to 4 m<sup>3</sup>/min, a cold air absolute moisture content was set to 3 g/m<sup>3</sup>, a blower flow rate was set to 20 m<sup>3</sup>/min, and an injection air flow rate was set to 1 m<sup>3</sup>/min.

40 50 1.0 Part by mass of hydrophobic silica fine particles subjected to a surface treatment with 4 mass % of hexamethyldisilazane and having a BET specific surface area of 25 m<sup>2</sup>/g, and 0.8 part by mass of hydrophobic silica fine particles subjected to a surface treatment with 10 mass % of polydimethylsiloxane and having a BET specific surface area of 100 m<sup>2</sup>/g were added to 100 parts by mass of the heat treated toner particles, and the contents were mixed with a Henschel mixer (Model FM-75 manufactured by NIPPON COKE & ENGINEERING CO., LTD.) at a number of rotations of 30 rotations/sec for a time of rotation of 10 minutes to obtain a toner 1. The toner 1 had a weight-average particle diameter (D4) of 6.2 μm and an average circularity of 0.965.

## EXAMPLE 2

65 A toner 2 was produced in the same manner as in Example 1 except that in Example 1, the external addition step (addi-

tion of the silica fine particles) was not performed before the heat treatment step with the surface treatment apparatus. The toner 2 had a weight-average particle diameter (D4) of 6.2  $\mu\text{m}$  and an average circularity of 0.955.

## EXAMPLE 3

A toner 3 was produced in the same manner as in Example 2 except that the heat treatment with the surface treatment apparatus was not performed. The toner 3 had a weight-average particle diameter (D4) of 6.2  $\mu\text{m}$  and an average circularity of 0.955.

## EXAMPLE 4

A toner 4 was produced in the same manner as in Example 3 except that the apparatus used in the classification after the fine pulverization was changed from the Faculty F-300 (manufactured by Hosokawa Micron Corporation) to a rotary classifier TSP-200 (manufactured by Hosokawa Micron Corporation). The operating condition of the rotary classifier TSP-200 (manufactured by Hosokawa Micron Corporation) was as follows: the number of rotations of a classification rotor was set to 50.0 rotations/sec. The toner 4 had a weight-average particle diameter (D4) of 6.2  $\mu\text{m}$  and an average circularity of 0.950.

## EXAMPLES 5 AND 6

Toners 5 and 6 were each produced in the same manner as in Example 4 except that the number of parts by mass of the polymer C was changed as shown in Table 5. The toners 5 and 6 each had a weight-average particle diameter (D4) of 6.2  $\mu\text{m}$  and an average circularity of 0.950.

## EXAMPLES 7 TO 39

Toners 7 to 39 were each produced in the same manner as in Example 4 except that the hydrocarbon wax was changed to an ester wax (peak temperature of the highest endothermic peak: 85° C.) and the other materials were also changed as shown in Table 5. Each of those toners had a weight-average particle diameter (D4) of 6.2  $\mu\text{m}$  and an average circularity of 0.950.

## COMPARATIVE EXAMPLES 1 TO 14

Toners 40 to 53 were each produced in the same manner as in Example 4 except that the polyester resin A and the polyester resin B were changed as shown in Table 5. Each of those toners had a weight-average particle diameter (D4) of 6.2  $\mu\text{m}$  and an average circularity of 0.950.

TABLE 5

|            | Toner    | Kind | Polyester resin A |      | Polyester resin B |           | Polymer C | Max              |      |
|------------|----------|------|-------------------|------|-------------------|-----------|-----------|------------------|------|
|            |          |      | Part (s) by mass  | Kind | Part (s) by mass  | ratio A/B |           | Part (s) by mass | Kind |
| Example 1  | Toner 1  | A1   | 25                | B1   | 75                | 25/75     | 5         | Hydrocarbon wax  | 6    |
| Example 2  | Toner 2  | A1   | 25                | B1   | 75                | 25/75     | 5         | Hydrocarbon wax  | 6    |
| Example 3  | Toner 3  | A1   | 25                | B1   | 75                | 25/75     | 5         | Hydrocarbon wax  | 6    |
| Example 4  | Toner 4  | A1   | 25                | B1   | 75                | 25/75     | 5         | Hydrocarbon wax  | 6    |
| Example 5  | Toner 5  | A1   | 25                | B1   | 75                | 25/75     | 2         | Hydrocarbon wax  | 6    |
| Example 6  | Toner 6  | A1   | 25                | B1   | 75                | 25/75     | None      | Hydrocarbon wax  | 6    |
| Example 7  | Toner 7  | A1   | 25                | B1   | 75                | 25/75     | None      | Ester wax        | 6    |
| Example 8  | Toner 8  | A1   | 25                | B2   | 75                | 25/75     | None      | "                | 6    |
| Example 9  | Toner 9  | A1   | 25                | B3   | 75                | 25/75     | None      | "                | 6    |
| Example 10 | Toner 10 | A1   | 25                | B4   | 75                | 25/75     | None      | "                | 6    |
| Example 11 | Toner 11 | A1   | 25                | B5   | 75                | 25/75     | None      | "                | 6    |
| Example 12 | Toner 12 | A1   | 25                | B6   | 75                | 25/75     | None      | "                | 6    |
| Example 13 | Toner 13 | A1   | 25                | B7   | 75                | 25/75     | None      | "                | 6    |
| Example 14 | Toner 14 | A2   | 25                | B7   | 75                | 25/75     | None      | "                | 6    |
| Example 15 | Toner 15 | A1   | 15                | B7   | 85                | 15/85     | None      | "                | 6    |
| Example 16 | Toner 16 | A1   | 40                | B7   | 60                | 40/60     | None      | "                | 6    |
| Example 17 | Toner 17 | A1   | 55                | B7   | 45                | 55/45     | None      | "                | 6    |
| Example 18 | Toner 18 | A3   | 25                | B7   | 75                | 25/75     | None      | "                | 6    |
| Example 19 | Toner 19 | A4   | 25                | B7   | 75                | 25/75     | None      | "                | 6    |
| Example 20 | Toner 20 | A5   | 25                | B7   | 75                | 25/75     | None      | "                | 6    |
| Example 21 | Toner 21 | A6   | 25                | B7   | 75                | 25/75     | None      | "                | 6    |
| Example 22 | Toner 22 | A1   | 25                | B8   | 75                | 25/75     | None      | "                | 6    |
| Example 23 | Toner 23 | A1   | 25                | B9   | 75                | 25/75     | None      | "                | 6    |
| Example 24 | Toner 24 | A1   | 25                | B10  | 75                | 25/75     | None      | "                | 6    |
| Example 25 | Toner 25 | A1   | 25                | B11  | 75                | 25/75     | None      | "                | 6    |
| Example 26 | Toner 26 | A7   | 25                | B7   | 75                | 25/75     | None      | "                | 6    |
| Example 27 | Toner 27 | A8   | 25                | B7   | 75                | 25/75     | None      | "                | 6    |
| Example 28 | Toner 28 | A9   | 25                | B7   | 75                | 25/75     | None      | "                | 6    |
| Example 29 | Toner 29 | A10  | 25                | B7   | 75                | 25/75     | None      | "                | 6    |
| Example 30 | Toner 30 | A11  | 25                | B7   | 75                | 25/75     | None      | "                | 6    |
| Example 31 | Toner 31 | A12  | 25                | B7   | 75                | 25/75     | None      | "                | 6    |
| Example 32 | Toner 32 | A13  | 25                | B7   | 75                | 25/75     | None      | "                | 6    |
| Example 33 | Toner 33 | A14  | 25                | B7   | 75                | 25/75     | None      | "                | 6    |
| Example 34 | Toner 34 | A15  | 25                | B7   | 75                | 25/75     | None      | "                | 6    |
| Example 35 | Toner 35 | A16  | 25                | B7   | 75                | 25/75     | None      | "                | 6    |

TABLE 5-continued

|                        | Polyester resin A |      | Polyester resin B |                  | Mass | Polymer C | Max              |                 |                  |
|------------------------|-------------------|------|-------------------|------------------|------|-----------|------------------|-----------------|------------------|
|                        | Toner             | Kind | Part (s) by mass  | Part (s) by mass |      | ratio A/B | Part (s) by mass | Kind            | Part (s) by mass |
| Example 36             | Toner 36          | A17  | 25                | B7               | 75   | 25/75     | None             | "               | 6                |
| Example 37             | Toner 37          | A1   | 25                | B12              | 75   | 25/75     | None             | "               | 6                |
| Example 38             | Toner 38          | A18  | 25                | B7               | 75   | 25/75     | None             | "               | 6                |
| Example 39             | Toner 39          | A19  | 25                | B7               | 75   | 25/75     | None             | "               | 6                |
| Comparative Example 1  | Toner 40          | A1   | 5                 | B1               | 95   | 5/95      | 5                | Hydrocarbon wax | 6                |
| Comparative Example 2  | Toner 41          | A1   | 65                | B1               | 35   | 65/35     | 5                | Hydrocarbon wax | 6                |
| Comparative Example 3  | Toner 42          | A20  | 25                | B1               | 75   | 25/75     | 5                | Hydrocarbon wax | 6                |
| Comparative Example 4  | Toner 43          | A21  | 25                | B1               | 75   | 25/75     | 5                | Hydrocarbon wax | 6                |
| Comparative Example 5  | Toner 44          | A1   | 25                | B13              | 75   | 25/75     | 5                | Hydrocarbon wax | 6                |
| Comparative Example 6  | Toner 45          | A1   | 25                | B14              | 75   | 25/75     | 5                | Hydrocarbon wax | 6                |
| Comparative Example 7  | Toner 46          | A22  | 25                | B1               | 75   | 25/75     | 5                | Hydrocarbon wax | 6                |
| Comparative Example 8  | Toner 47          | A23  | 25                | B1               | 75   | 25/75     | 5                | Hydrocarbon wax | 6                |
| Comparative Example 9  | Toner 48          | A24  | 25                | B1               | 75   | 25/75     | 5                | Hydrocarbon wax | 6                |
| Comparative Example 10 | Toner 49          | A25  | 25                | B1               | 75   | 25/75     | 5                | Hydrocarbon wax | 6                |
| Comparative Example 11 | Toner 50          | A26  | 25                | B1               | 75   | 25/75     | 5                | Hydrocarbon wax | 6                |
| Comparative Example 12 | Toner 51          | A27  | 25                | B1               | 75   | 25/75     | 5                | Hydrocarbon wax | 6                |
| Comparative Example 13 | Toner 52          | A1   | 25                | B15              | 75   | 25/75     | 5                | Hydrocarbon wax | 6                |
| Comparative Example 14 | Toner 53          | A1   | 25                | B16              | 75   | 25/75     | 5                | Hydrocarbon wax | 6                |

## EXAMPLE 101

## 1. Production of Magnetic Core Particles

Ferrite raw materials shown in Table 6 below were weighed. After that, the raw materials were pulverized and mixed with a dry ball mill using a zirconia ball ( $\phi 10$  mm) for 2 hours.

TABLE 6

| Ferrite raw material     |        |                                                                          |
|--------------------------|--------|--------------------------------------------------------------------------|
| Material                 | Mass % | Composition of ferrite                                                   |
| $\text{Fe}_2\text{O}_3$  | 60.2   | $a = 0.39, b = 0.11, c = 0.01, \text{ and } d = 0.50$                    |
| $\text{MnCO}_3$          | 33.9   | in $(\text{MnO})_a(\text{MgO})_b(\text{SrO})_c(\text{Fe}_2\text{O}_3)_d$ |
| $\text{Mg}(\text{OH})_2$ | 4.8    |                                                                          |
| $\text{SrCO}_3$          | 1.1    |                                                                          |

Next, the mixture was calcined with a burner-type kiln in the air at  $1,000^\circ \text{C}$ . for 3 hours to produce a calcined ferrite of the composition shown in the right column of Table 6. The calcined ferrite was pulverized with a crusher to about 0.5 mm. After that, 30 parts by mass of water were added to 100 parts by mass of the calcined ferrite, and the mixture was pulverized with a wet ball mill using a zirconia ball ( $\phi 10$  mm) for 2 hours. A slurry thus obtained was pulverized with a wet bead mill using zirconia beads ( $\phi 1.0$  mm) for 4 hours to provide a ferrite slurry. 2.0 Parts by mass of a polyvinyl alcohol with respect to 100 parts by mass of the calcined ferrite were added as a binder to the ferrite slurry, and the mixture was granulated with a spray dryer (manufacturer: OHKAWARA KAKOHKI CO., LTD.) into spherical particles each having a diameter of about  $36 \mu\text{m}$ .

<sup>35</sup> Next, the spherical particles were calcined in an electric furnace under a nitrogen atmosphere (having an oxygen concentration of 1.00 vol % or less) at  $1,150^\circ \text{C}$ . for 4 hours in order that a calcination atmosphere was controlled. Agglomerated particles obtained by the calcination were shredded and then coarse particles were removed by sieving with a sieve having an aperture of  $250 \mu\text{m}$ . Thus, magnetic core particles 1 were obtained.

## 2. Production of Coating Resin

<sup>45</sup> Materials shown in Table 7 below were added to a four-necked separable flask mounted with a reflux condenser, a temperature gauge, a nitrogen-introducing tube, and a stirring apparatus, and a nitrogen gas was introduced to sufficiently establish a nitrogen atmosphere in the flask. After that, a <sup>50</sup> temperature in the flask was warmed to  $80^\circ \text{C}$ ., 2.0 parts by mass of azobisisobutyronitrile were added to the mixture, and the whole was refluxed and polymerized for 5 hours. Hexane was injected into the resultant reaction product to precipitate and deposit a copolymer, and the precipitate was separated by <sup>55</sup> filtration. After that, the precipitate was dried in a vacuum to provide a coating resin 1.

TABLE 7

| Material                                                                                              | Part(s) by mass |
|-------------------------------------------------------------------------------------------------------|-----------------|
| Cyclohexyl methacrylate monomer                                                                       | 26.8            |
| Methyl methacrylate monomer                                                                           | 0.2             |
| Methyl methacrylate macromonomer                                                                      | 8.4             |
| (macromonomer having a methacryloyl group at one terminal and mass-average molecular weight of 5,000) |                 |

TABLE 7-continued

| Material            | Part(s)<br>by mass |
|---------------------|--------------------|
| Toluene             | 31.3               |
| Methyl ethyl ketone | 31.3               |

## 3. Production of Magnetic Carrier

20.0 Parts by mass of the coating resin 1 and 80.0 parts by mass of toluene were dispersed and mixed with a bead mill to provide a resin liquid 1.

Next, 100 parts by mass of the magnetic core particles 1 were loaded into a Nauta mixer. Further, the resin liquid 1 was charged into the Nauta mixer so that its amount in terms of a resin component became 2.0 parts by mass. Under reduced pressure, the contents were heated to a temperature of 70° C. and mixed at 100 rpm, followed by the performance of solvent removal and an application operation over 4 hours. After that, the resultant sample was transferred to a *Julia* mixer and thermally treated under a nitrogen atmosphere at a temperature of 100° C. for 2 hours. After that, the resultant was classified with a sieve having an aperture of 70 µm to provide a magnetic carrier 1. The resultant magnetic carrier 1 had a 50% particle diameter (D50) on a volume distribution basis of 38.2 µm.

## 4. Production of Two-Component Developer

The toner 1 and the magnetic carrier 1 were mixed with a V-type mixer (Model V-10: TOKUJU CORPORATION) at a number of rotations of 0.5 rotation/sec for a time of rotation of 5 minutes so that a toner concentration became 8 mass %. Thus, a two-component developer 1 was obtained. The developer was subjected to the following evaluations.

## 5. Evaluation for Developability

A full-color copying machine imageRUNNER ADVANCE C9075PRO manufactured by Canon Inc. as an image-forming apparatus was reconstructed so that its process speed could be freely set, and the two-component developer 1 was evaluated.

An image output evaluation (A4 horizontal, print percentage: 80%, 5,000-sheet continuous passing) was performed under each of a normal-temperature and normal-humidity environment (having a temperature of 23° C. and a relative humidity of 50%), a normal-temperature and low-humidity environment (having a temperature of 23° C. and a relative humidity of 5%), and a high-temperature and high-humidity environment (having a temperature of 30° C. and a relative humidity of 80%), and under the following condition: the process speed was changed to 450 mm/sec. During a 5,000-sheet continuous passing time, sheet passing was performed under the same development condition and transfer condition (no calibration) as those of the first sheet. Used as evaluation paper was copier paper GF-0081 (A4, basis weight: 81.4 g/m<sup>2</sup>, sold by Canon Marketing Japan Inc.). Under each of the evaluation environments, the toner laid-on level of an FFH image (solid portion) on the paper was adjusted to 0.45 mg/cm<sup>2</sup>. The FFH image refers to a value obtained by representing 256 gray levels in a hexadecimal notation, and is such an image that OOH represents the first gray level (white portion) and FFH represents the 256-th gray level (solid portion).

The items and evaluation criteria of the image output evaluation at the initial stage (first sheet) and at the time of the 5,000-sheet continuous passing are shown below. In addition, Tables 9 to 11 show the results of the evaluations.

## (1) Measurement of Image Density

The image densities of FFH image portions, i.e., solid portions at the initial stage (first sheet) and on the 5,000-th sheet were measured with an X-Rite Color Reflection Densitometer (500 Series: manufactured by X-Rite), and a difference A between both the image densities was ranked by the following criteria.

## (Evaluation Criteria)

- A: Less than 0.05 (The image density is extremely excellent.)  
 10 B: From 0.05 or more to less than 0.10 (The image density is good.)  
 C: From 0.10 or more to less than 0.20 (The image density is at the level at which the effect of the present invention is obtained.)  
 15 D: 0.20 or more (The image density is at the level at which the effect of the present invention is not sufficiently obtained.)

## (2) Measurement of Fogging

An average reflectance Dr (%) of the evaluation paper before the image output was measured with a reflectometer ("REFLECTOMETER MODEL TC-6DS" manufactured by Tokyo Denshoku CO., LTD.). In addition, reflectances Ds (%) of OOH image portions, i.e., white portions at the initial stage (first sheet) and on the 5,000-th sheet were measured. Fogging (%) was calculated from the resultant Dr and Ds's (the initial stage (first sheet) and the 5,000-th sheet) by using the following equation. The resultant value for the fogging was ranked in accordance with the following evaluation criteria.

$$30 \text{ Fogging } (\%) = Dr(\%) - Ds(\%)$$

## (Evaluation Criteria)

- A: Less than 0.5% (The fogging is extremely excellent.)  
 B: From 0.5% or more to less than 1.0% (The fogging is good.)  
 35 C: From 1.0% or more to less than 2.0% (The fogging is at the level at which the effect of the present invention is obtained.)  
 D: 2.0% or more (The fogging is at the level at which the effect of the present invention is not sufficiently obtained.)  
 40

## (6. Evaluation for Fixability (Low-Temperature Fixability and Hot Offset Resistance))

A full-color copying machine imageRUNNER ADVANCE C9075PRO manufactured by Canon Inc. was reconstructed so that its fixation temperature and process speed could be freely set, and the two-component developer 1 was tested for its fixation temperature region. An unfixed image was produced according to a monochromatic mode while the toner laid-on level of the image on the paper under a normal-temperature and normal-humidity environment (having a temperature of 23° C. and a relative humidity of from 50% or more to 60% or less) was adjusted to 1.2 mg/cm<sup>2</sup>. Copier paper GF-0081 (A4, basis weight: 81.4 g/m<sup>2</sup>, sold by Canon Marketing Japan Inc.) was used as evaluation paper, and the image was formed at an image print percentage of 25%. After that, under the normal-temperature and normal-humidity environment (having a temperature of 23° C. and a relative humidity of from 50% or more to 60% or less), the process speed was set to 450 mm/sec, the fixation temperature was increased from 100° C. in increments of 5° C., and a temperature width in which no offset occurred (equal to or more than a fixable temperature and equal to or less than the temperature at which an offset occurred) was defined as a fixable region. The lower limit temperature of the fixable region was defined as a lower-limit fixation temperature and the upper limit temperature thereof was defined as a hot offset resistance temperature.

The lower-limit fixation temperature and the hot offset resistance temperature were ranked by the following criteria. Table 12 shows the results of the evaluation.

(Evaluation Criteria for Lower-Limit Fixation Temperature)

A: Less than 140° C. (The temperature is extremely excellent.)

B: From 140° C. or more to less than 150° C. (The temperature is good.)

C: From 150° C. or more to less than 160° C. (The temperature is at the level at which the effect of the present invention is obtained.)

D: 160° C. or more (The temperature is at the level at which the effect of the present invention is not sufficiently obtained.)

(Evaluation Criteria for Hot Offset Resistance Temperature)

A: 210° C. or more (The temperature is extremely excellent.)

B: From 200° C. or more to less than 210° C. (The temperature is good.)

C: From 190° C. or more to less than 195° C. (The temperature is at the level at which the effect of the present invention is obtained.)

D: Less than 190° C. (The temperature is at the level at which the effect of the present invention is not sufficiently obtained.)

#### EXAMPLES 102 TO 139 AND COMPARATIVE EXAMPLES 101 to 114

Evaluations were performed in the same manner as in Example 1 except that the two-component developer to be used in the evaluations was changed to two-component developers shown in Table 8. Tables 9 to 12 show the results of the evaluations.

TABLE 8

|             | Toner                   | Magnetic carrier   | Two-component developer    |                            |
|-------------|-------------------------|--------------------|----------------------------|----------------------------|
| Example 101 | Toner 1                 | Magnetic carrier 1 | Two-component developer 1  |                            |
| Example 102 | Toner 2                 | Magnetic carrier 1 | Two-component developer 2  |                            |
| Example 103 | Toner 3                 | Magnetic carrier 1 | Two-component developer 3  |                            |
| Example 104 | Toner 4                 | Magnetic carrier 1 | Two-component developer 4  |                            |
| Example 105 | Toner 5                 | Magnetic carrier 1 | Two-component developer 5  |                            |
| Example 106 | Toner 6                 | Magnetic carrier 1 | Two-component developer 6  |                            |
| Example 107 | Toner 7                 | Magnetic carrier 1 | Two-component developer 7  |                            |
| Example 108 | Toner 8                 | Magnetic carrier 1 | Two-component developer 8  |                            |
| Example 109 | Toner 9                 | Magnetic carrier 1 | Two-component developer 9  |                            |
| Example 110 | Toner 10                | Magnetic carrier 1 | Two-component developer 10 |                            |
| Example 111 | Toner 11                | Magnetic carrier 1 | Two-component developer 11 |                            |
| Example 112 | Toner 12                | Magnetic carrier 1 | Two-component developer 12 |                            |
| Example 113 | Toner 13                | Magnetic carrier 1 | Two-component developer 13 |                            |
| Example 114 | Toner 14                | Magnetic carrier 1 | Two-component developer 14 |                            |
| Example 115 | Toner 15                | Magnetic carrier 1 | Two-component developer 15 |                            |
| Example 116 | Toner 16                | Magnetic carrier 1 | Two-component developer 16 |                            |
| 5           | Example 117             | Toner 17           | Magnetic carrier 1         | Two-component developer 17 |
|             | Example 118             | Toner 18           | Magnetic carrier 1         | Two-component developer 18 |
|             | Example 119             | Toner 19           | Magnetic carrier 1         | Two-component developer 19 |
| 10          | Example 120             | Toner 20           | Magnetic carrier 1         | Two-component developer 20 |
|             | Example 121             | Toner 21           | Magnetic carrier 1         | Two-component developer 21 |
|             | Example 122             | Toner 22           | Magnetic carrier 1         | Two-component developer 22 |
| 15          | Example 123             | Toner 23           | Magnetic carrier 1         | Two-component developer 23 |
|             | Example 124             | Toner 24           | Magnetic carrier 1         | Two-component developer 24 |
|             | Example 125             | Toner 25           | Magnetic carrier 1         | Two-component developer 25 |
| 20          | Example 126             | Toner 26           | Magnetic carrier 1         | Two-component developer 26 |
|             | Example 127             | Toner 27           | Magnetic carrier 1         | Two-component developer 27 |
|             | Example 128             | Toner 28           | Magnetic carrier 1         | Two-component developer 28 |
| 25          | Example 129             | Toner 29           | Magnetic carrier 1         | Two-component developer 29 |
|             | Example 130             | Toner 30           | Magnetic carrier 1         | Two-component developer 30 |
|             | Example 131             | Toner 31           | Magnetic carrier 1         | Two-component developer 31 |
|             | Example 132             | Toner 32           | Magnetic carrier 1         | Two-component developer 32 |
| 30          | Example 133             | Toner 33           | Magnetic carrier 1         | Two-component developer 33 |
|             | Example 134             | Toner 34           | Magnetic carrier 1         | Two-component developer 34 |
|             | Example 135             | Toner 35           | Magnetic carrier 1         | Two-component developer 35 |
| 35          | Example 136             | Toner 36           | Magnetic carrier 1         | Two-component developer 36 |
|             | Example 137             | Toner 37           | Magnetic carrier 1         | Two-component developer 37 |
|             | Example 138             | Toner 38           | Magnetic carrier 1         | Two-component developer 38 |
| 40          | Example 139             | Toner 39           | Magnetic carrier 1         | Two-component developer 39 |
|             | Comparative Example 101 | Toner 40           | Magnetic carrier 1         | Two-component developer 40 |
|             | Comparative Example 102 | Toner 41           | Magnetic carrier 1         | Two-component developer 41 |
| 45          | Comparative Example 103 | Toner 42           | Magnetic carrier 1         | Two-component developer 42 |
|             | Comparative Example 104 | Toner 43           | Magnetic carrier 1         | Two-component developer 43 |
|             | Comparative Example 105 | Toner 44           | Magnetic carrier 1         | Two-component developer 44 |
| 50          | Comparative Example 106 | Toner 45           | Magnetic carrier 1         | Two-component developer 45 |
|             | Comparative Example 107 | Toner 46           | Magnetic carrier 1         | Two-component developer 46 |
|             | Comparative Example 108 | Toner 47           | Magnetic carrier 1         | Two-component developer 47 |
| 55          | Comparative Example 109 | Toner 48           | Magnetic carrier 1         | Two-component developer 48 |
|             | Comparative Example 110 | Toner 49           | Magnetic carrier 1         | Two-component developer 49 |
|             | Comparative Example 111 | Toner 50           | Magnetic carrier 1         | Two-component developer 50 |
| 60          | Comparative Example 112 | Toner 51           | Magnetic carrier 1         | Two-component developer 51 |
|             | Comparative Example 113 | Toner 52           | Magnetic carrier 1         | Two-component developer 52 |
| 65          | Comparative Example 114 | Toner 53           | Magnetic carrier 1         | Two-component developer 53 |

TABLE 8-continued

TABLE 9

| (under normal-temperature and normal-humidity environment) |  |  |  |  |  |  |  |  |  |
|------------------------------------------------------------|--|--|--|--|--|--|--|--|--|
|------------------------------------------------------------|--|--|--|--|--|--|--|--|--|

|                         | Image density |                |              |      |             | 5 | Image density |                |              |      |     |  |
|-------------------------|---------------|----------------|--------------|------|-------------|---|---------------|----------------|--------------|------|-----|--|
|                         | Density       |                | Fogging      |      |             |   | Density       |                | Fogging      |      |     |  |
|                         | First sheet   | 5,000-th sheet | difference Δ | Rank | First sheet |   | First sheet   | 5,000-th sheet | difference Δ | Rank |     |  |
| Example 101             | 1.50          | 1.48           | 0.02         | A    | 0.1         | A | 0.2           | A              | 0.02         | A    | 0.1 |  |
| Example 102             | 1.50          | 1.48           | 0.02         | A    | 0.1         | A | 0.2           | A              | 0.02         | A    | 0.1 |  |
| Example 103             | 1.50          | 1.48           | 0.02         | A    | 0.1         | A | 0.2           | A              | 0.02         | A    | 0.1 |  |
| Example 104             | 1.50          | 1.48           | 0.02         | A    | 0.1         | A | 0.3           | A              | 0.02         | A    | 0.1 |  |
| Example 105             | 1.50          | 1.48           | 0.02         | A    | 0.1         | A | 0.3           | A              | 0.03         | A    | 0.2 |  |
| Example 106             | 1.50          | 1.47           | 0.03         | A    | 0.2         | A | 0.6           | B              | 0.03         | A    | 0.2 |  |
| Example 107             | 1.50          | 1.47           | 0.03         | A    | 0.2         | A | 0.6           | B              | 0.03         | A    | 0.2 |  |
| Example 108             | 1.50          | 1.47           | 0.03         | A    | 0.2         | A | 0.6           | B              | 0.03         | A    | 0.2 |  |
| Example 109             | 1.50          | 1.47           | 0.03         | A    | 0.2         | A | 0.6           | B              | 0.03         | A    | 0.2 |  |
| Example 110             | 1.50          | 1.47           | 0.03         | A    | 0.2         | A | 0.6           | B              | 0.03         | A    | 0.2 |  |
| Example 111             | 1.50          | 1.47           | 0.03         | A    | 0.2         | A | 0.6           | B              | 0.03         | A    | 0.2 |  |
| Example 112             | 1.50          | 1.47           | 0.03         | A    | 0.2         | A | 0.6           | B              | 0.03         | A    | 0.2 |  |
| Example 113             | 1.50          | 1.47           | 0.03         | A    | 0.2         | A | 0.6           | B              | 0.08         | B    | 0.5 |  |
| Example 114             | 1.50          | 1.42           | 0.08         | B    | 0.5         | B | 1.6           | C              | 0.08         | B    | 1.0 |  |
| Example 115             | 1.50          | 1.42           | 0.08         | B    | 0.6         | B | 1.0           | C              | 0.03         | A    | 0.5 |  |
| Example 116             | 1.50          | 1.47           | 0.03         | A    | 0.2         | A | 0.5           | B              | 0.03         | A    | 0.5 |  |
| Example 117             | 1.50          | 1.47           | 0.03         | A    | 0.2         | A | 0.5           | B              | 0.03         | A    | 0.6 |  |
| Example 118             | 1.50          | 1.47           | 0.03         | A    | 0.2         | A | 0.6           | B              | 0.05         | B    | 1.2 |  |
| Example 119             | 1.50          | 1.45           | 0.05         | B    | 0.6         | B | 1.2           | C              | 0.04         | A    | 0.6 |  |
| Example 120             | 1.50          | 1.46           | 0.04         | A    | 0.2         | A | 0.6           | B              | 0.08         | B    | 0.9 |  |
| Example 121             | 1.50          | 1.42           | 0.08         | B    | 0.4         | A | 0.9           | B              | 0.06         | B    | 0.7 |  |
| Example 122             | 1.50          | 1.44           | 0.06         | B    | 0.3         | A | 0.7           | B              | 0.08         | B    | 1.0 |  |
| Example 123             | 1.50          | 1.42           | 0.08         | B    | 0.6         | B | 1.0           | C              | 0.04         | A    | 0.6 |  |
| Example 124             | 1.50          | 1.46           | 0.04         | A    | 0.2         | A | 0.6           | B              | 0.03         | A    | 0.5 |  |
| Example 125             | 1.50          | 1.47           | 0.03         | A    | 0.2         | A | 0.5           | B              | 0.06         | B    | 0.9 |  |
| Example 126             | 1.50          | 1.44           | 0.06         | B    | 0.4         | A | 0.9           | B              | 0.08         | B    | 0.9 |  |
| Example 127             | 1.50          | 1.42           | 0.08         | B    | 0.4         | A | 0.9           | B              | 0.08         | B    | 1.0 |  |
| Example 128             | 1.50          | 1.42           | 0.08         | B    | 0.5         | B | 1.0           | C              | 0.08         | B    | 1.2 |  |
| Example 129             | 1.50          | 1.42           | 0.08         | B    | 0.6         | B | 1.2           | C              | 0.09         | B    | 1.2 |  |
| Example 130             | 1.50          | 1.41           | 0.09         | B    | 0.6         | B | 1.2           | C              | 0.07         | B    | 1.0 |  |
| Example 131             | 1.50          | 1.43           | 0.07         | B    | 0.5         | B | 1.0           | C              | 0.04         | A    | 0.6 |  |
| Example 132             | 1.50          | 1.46           | 0.04         | A    | 0.2         | A | 0.6           | B              | 0.09         | B    | 1.4 |  |
| Example 133             | 1.50          | 1.41           | 0.09         | B    | 0.8         | B | 1.4           | C              | 0.06         | B    | 0.7 |  |
| Example 134             | 1.50          | 1.44           | 0.06         | B    | 0.4         | A | 0.7           | B              | 0.07         | B    | 0.9 |  |
| Example 135             | 1.50          | 1.43           | 0.07         | B    | 0.5         | B | 0.9           | B              | 0.10         | C    | 0.7 |  |
| Example 136             | 1.50          | 1.40           | 0.10         | C    | 0.7         | B | 1.2           | C              | 0.04         | A    | 0.8 |  |
| Example 137             | 1.50          | 1.46           | 0.04         | A    | 0.2         | A | 0.8           | B              | 0.04         | A    | 0.7 |  |
| Example 138             | 1.50          | 1.46           | 0.04         | A    | 0.3         | A | 0.7           | B              | 0.03         | A    | 0.6 |  |
| Example 139             | 1.50          | 1.47           | 0.03         | A    | 0.2         | A | 0.6           | B              | 0.13         | C    | 2.1 |  |
| Comparative Example 101 | 1.50          | 1.37           | 0.13         | C    | 1.2         | C | 2.1           | D              | 0.01         | A    | 0.5 |  |
| Comparative Example 102 | 1.50          | 1.47           | 0.03         | A    | 0.2         | A | 0.5           | B              | 0.08         | B    | 2.0 |  |
| Comparative Example 103 | 1.50          | 1.42           | 0.08         | B    | 1.0         | C | 1.8           | C              | 0.08         | B    | 1.2 |  |
| Comparative Example 104 | 1.50          | 1.42           | 0.08         | B    | 0.6         | B | 1.2           | C              | 0.09         | B    | 1.4 |  |
| Comparative Example 105 | 1.50          | 1.41           | 0.09         | B    | 0.7         | B | 1.4           | C              | 0.04         | A    | 0.5 |  |
| Comparative Example 106 | 1.50          | 1.46           | 0.04         | A    | 0.2         | A | 0.5           | B              | 0.15         | D    | 2.2 |  |
| Comparative Example 107 | 1.50          | 1.35           | 0.15         | D    | 0.6         | B | 2.2           | D              | 0.17         | D    | 2.0 |  |
| Comparative Example 108 | 1.50          | 1.33           | 0.17         | D    | 1.1         | C | 2.0           | D              | 0.13         | C    | 2.5 |  |
| Comparative Example 109 | 1.50          | 1.33           | 0.17         | D    | 1.5         | C | 2.5           | D              | 0.10         | C    | 2.0 |  |
| Comparative Example 110 | 1.50          | 1.40           | 0.10         | C    | 1.2         | C | 2.0           | D              | 0.12         | C    | 2.0 |  |
| Comparative Example 111 | 1.50          | 1.37           | 0.13         | C    | 1.5         | C | 2.2           | D              | 0.13         | C    | 2.2 |  |
| Comparative Example 112 | 1.50          | 1.35           | 0.15         | D    | 1.3         | C | 2.3           | D              | 0.15         | D    | 2.3 |  |
| Comparative Example 113 | 1.50          | 1.40           | 0.10         | C    | 1.0         | C | 1.8           | C              | 0.10         | C    | 2.0 |  |
| Comparative Example 114 | 1.50          | 1.38           | 0.12         | C    | 1.5         | C | 1.8           | C              | 0.12         | C    | 2.0 |  |

TABLE 10

| (under normal-temperature and low-humidity environment) |  |  |  |  |  |  |  |  |  |
|---------------------------------------------------------|--|--|--|--|--|--|--|--|--|
|---------------------------------------------------------|--|--|--|--|--|--|--|--|--|

|                         | Image density |                |              |      |             | 5 | Image density |                |              |      |     |  |
|-------------------------|---------------|----------------|--------------|------|-------------|---|---------------|----------------|--------------|------|-----|--|
|                         | Density       |                | Fogging      |      |             |   | Density       |                | Fogging      |      |     |  |
|                         | First sheet   | 5,000-th sheet | difference Δ | Rank | First sheet |   | First sheet   | 5,000-th sheet | difference Δ | Rank |     |  |
| Example 101             | 1.50          | 1.48           | 0.02         | A    | 0.1         | A | 0.2           | A              | 0.02         | A    | 0.1 |  |
| Example 102             | 1.50          | 1.48           | 0.02         | A    | 0.1         | A | 0.2           | A              | 0.02         | A    | 0.2 |  |
| Example 103             | 1.50          | 1.48           | 0.02         | A    | 0.1         | A | 0.2           | A              | 0.02         | A    | 0.3 |  |
| Example 104             | 1.50          | 1.48           | 0.02         | A    | 0.1         | A | 0.3           | A              | 0.02         | A    | 0.3 |  |
| Example 105             | 1.50          | 1.48           | 0.02         | A    | 0.1         | A | 0.3           | A              | 0.03         | A    | 0.6 |  |
| Example 106             | 1.50          | 1.47           | 0.03         | A    | 0.2         | A | 0.6           | B              | 0.03         | A    | 0.6 |  |
| Example 107             | 1.50          | 1.47           | 0.03         | A    | 0.2         | A | 0.6           | B              | 0.03         | A    | 0.6 |  |
| Example 108             | 1.50          | 1.47           | 0.03         | A    | 0.2         | A | 0.6           | B              | 0.03         | A    | 0.6 |  |
| Example 109             | 1.50          | 1.47           | 0.03         | A    | 0.2         | A | 0.6           | B              | 0.03         | A    | 0.6 |  |
| Example 110             | 1.50          | 1.47           | 0.03         | A    | 0.2         | A | 0.6           | B              | 0.03         | A    | 0.6 |  |
| Example 111             | 1.50          | 1.47           | 0.03         | A    | 0.2         | A | 0.6           | B              | 0.03         | A    | 0.6 |  |
| Example 112             | 1.50          | 1.47           | 0.03         | A    | 0.2         | A | 0.6           | B              | 0.03         | A    | 0.6 |  |
| Example 113             | 1.50          | 1.47           | 0.03         | A    | 0.2         | A | 0.6           | B              | 0.08         | B    | 1.6 |  |
| Example 114             | 1.50          | 1.42           | 0.08         | B    | 0.5         | B | 1.6           | C              | 0.08         | B    | 1.0 |  |
| Example 115             | 1.50          | 1.42           | 0.08         | B    | 0.6         | B | 1.0           | C              | 0.03         | A    | 0.5 |  |
| Example 116             | 1.50          | 1.47           | 0.03         | A    | 0.2         | A | 0.5           | B              | 0.03         | A    | 0.5 |  |
| Example 117             | 1.50          | 1.47           | 0.03         | A    | 0.2         | A | 0.5           | B              | 0.03         | A    | 0.6 |  |
| Example 118             | 1.50          | 1.47           | 0.03         | A    | 0.2         | A | 0.6           | B              | 0.05         | B    | 1.2 |  |
| Example 119             | 1.50          | 1.46           | 0.04         | B    | 0.6         | B | 1.2           | C              | 0.04         | A    | 0.6 |  |
| Example 120             | 1.50          | 1.42           | 0.08         | A    | 0.2         | A | 0.6           | B              | 0.08         | B    | 0.9 |  |
| Example 121             | 1.50          | 1.42           | 0.08         | B    | 0.4         | A | 0.9           | B              | 0.06         | B    | 0.7 |  |
| Example 122             | 1.50          | 1.44           | 0.06         | B    | 0.3         | A | 0.7           | B              | 0.08         | B    | 1.0 |  |
| Example 123             | 1.50          | 1.42           | 0.08         | B    | 0.6         | B | 1.0           | C              | 0.04         | A    | 0.6 |  |
| Example 124             | 1.50          | 1.46           | 0.04         | A    | 0.2         | A | 0.6           | B              | 0.03         | A    | 0.5 |  |
| Example 125             | 1.50          | 1.47           | 0.03         | A    | 0.2         | A | 0.5           | B              | 0.06         | B    | 0.9 |  |
| Example 126             | 1.50          | 1.44           | 0.06         | B    | 0.4         | A | 0.9           | B              | 0.08         | B    | 0.9 |  |
| Example 127             | 1.50          | 1.42           | 0.08         | B    | 0.4         | A | 0.9           | B              | 0.08         | B    | 1.0 |  |
| Example 128             | 1.50          | 1.42           | 0.08         | B    | 0.5         | B | 1.0           | C              | 0.08         | B    | 1.2 |  |
| Example 129             | 1.50          | 1.42           | 0.08         | B    | 0.6         | B | 1.2           | C              | 0.09         | B    | 1.2 |  |
| Example 130             | 1.50          | 1.41           | 0.09         | B    | 0.6         | B | 1.2           | C              | 0.07         | B    | 1.0 |  |
| Example 131             | 1.50          | 1.43           | 0.07         | B    | 0.5         | B | 1.0           | C              | 0.04         | A    | 0.6 |  |
| Example 132             | 1.50          | 1.46           | 0.04         | A    | 0.2         | A | 0.6           | B              | 0.09         | B    | 1.4 |  |
| Example 133             | 1.50          | 1.41           | 0.09         | B    | 0.8         | B | 1.4           | C              | 0.06         | B    | 0.7 |  |
| Example 134             | 1.50          | 1.44           | 0.06         | B    | 0.4         | A | 0.7           | B              | 0.07         | B    | 0.9 |  |
| Example 135             | 1.50          | 1.43           | 0.07         | B    | 0.5         | B | 0.9           | B              | 0.10         | C    | 0.7 |  |
| Example 136             | 1.50          | 1.40           | 0.10         | C    | 0.7         | B | 1.2           | C              | 0.04         | A    | 0.8 |  |
| Example 137             | 1.50          | 1.46           | 0.04         | A    | 0.2         | A | 0.8           | B              | 0.04         | A    | 0.7 |  |
| Example 138             | 1.50          | 1.46           | 0.04         | A    | 0.3         | A | 0.7           | B              | 0.03         | A    | 0.6 |  |
| Comparative Example 101 | 1.50          | 1.37           | 0.13         | C    | 1.2         | C | 2.1           | D              | 0.13         | C    | 2.1 |  |
| Comparative Example 102 | 1.50          | 1.47           | 0.03         | A    | 0.2         | A | 0.5           | B              | 0.08         | B    | 2.0 |  |
| Comparative Example 103 | 1.50          | 1.42           | 0.08         | B    | 1.0         | C | 1.8           | C              | 0.08         | B    | 1.2 |  |
| Comparative Example 104 | 1.50          | 1.42           | 0.08         | B    | 0.6         | B | 1.2           | C              | 0.09         | B    | 1.4 |  |
| Comparative Example 105 | 1.50          | 1.41           | 0.09         | B    | 0.7         | B | 1.4           | C              | 0.04         | A    | 0.5 |  |
| Comparative Example 106 | 1.50          | 1.46           | 0.04         | A    | 0.2         | A | 0.5           | B              | 0.15         | D    | 2.2 |  |
| Comparative Example 107 | 1.50          | 1.35           | 0.15         | D    | 0.6         | B | 2.2           | D</td          |              |      |     |  |

TABLE 11

| (under high-temperature and high-humidity environment) |                |                     |      |             |                |      |             |                |               |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
|--------------------------------------------------------|----------------|---------------------|------|-------------|----------------|------|-------------|----------------|---------------|------|------|------|---|-----|---|-----|---|---------------|---------------|------|------|------|-----|-----|-----|-----|---------------|---------------|------|------|------|-----|-----|-----|-----|-------------|---------------|-------------|------|------|------|-----|-----|-----|-------------|---------------|---------------|------|------|------|-----|-----|-----|-------------|---------------|---------------|-------------|------|------|------|-----|-----|-------------|---------------|---------------|-------------|------|------|------|-----|-----|-------------|---------------|---------------|---------------|-------------|------|------|------|-----|-------------|---------------|---------------|---------------|-------------|------|------|------|-----|-------------|---------------|---------------|---------------|-------------|-------------|------|------|------|-------------|---------------|---------------|---------------|---------------|-------------|------|------|------|-------------|---------------|---------------|---------------|---------------|-------------|-------------|------|------|-------------|---------------|---------------|---------------|---------------|-------------|-------------|------|------|-------------|---------------|---------------|---------------|---------------|-------------|-------------|------|------|-------------|---------------|---------------|---------------|---------------|-------------|-------------|------|------|-------------|---------------|---------------|---------------|---------------|---------------|-------------|------|------|-------------|---------------|---------------|---------------|---------------|---------------|-------------|------|------|-------------|---------------|---------------|---------------|---------------|---------------|-------------|------|------|-------------|---------------|---------------|---------------|---------------|---------------|-------------|------|------|-------------|---------------|---------------|---------------|---------------|---------------|-------------|------|------|-------------|---------------|---------------|---------------|---------------|---------------|-------------|------|------|-------------|---------------|---------------|---------------|---------------|---------------|-------------|------|------|------|---------------|---------------|---------------|---------------|---------------|-------------|------|------|------|---------------|---------------|---------------|---------------|---------------|-------------|------|------|------|---------------|---------------|---------------|---------------|---------------|-------------|------|------|------|---------------|---------------|---------------|---------------|---------------|-------------|------|------|------|-------------|---------------|---------------|---------------|---------------|-------------|------|------|------|-----|---------------|---------------|---------------|---------------|-------------|------|------|------|-----|---------------|---------------|---------------|---------------|-------------|------|------|------|-----|---------------|---------------|---------------|---------------|-------------|------|------|------|-----|-----|---------------|---------------|---------------|-------------|------|------|------|-----|-----|---------------|---------------|---------------|-------------|------|------|------|-----|-----|---------------|---------------|---------------|-------------|------|------|------|-----|-----|-----|---------------|---------------|-------------|------|------|------|-----|-----|-----|---------------|---------------|-------------|-------------|------|------|------|-----|-----|---------------|---------------|---------------|-------------|------|------|------|-----|-----|-----|---------------|---------------|-------------|------|------|------|-----|-----|-----|---------------|---------------|---------------|------|------|------|-----|-----|-----|---------------|---------------|---------------|------|------|------|-----|-----|-----|-----|---------------|---------------|---------------|------|------|------|-----|-----|-----|---------------|---------------|---------------|------|------|------|-----|-----|-----|-----|---------------|---------------|------|------|------|-----|-----|-----|-----|---------------|---------------|---------------|------|------|------|-----|-----|-----|-----|---------------|---------------|------|------|------|-----|-----|-----|-----|---------------|---------------|------|------|------|-----|-----|-----|-----|----|---------------|---------------|------|------|------|-----|-----|-----|-----|---------------|---------------|------|------|------|-----|-----|-----|-----|----|---------------|------|------|------|---|-----|---|-----|---|---------------|---------------|------|------|------|-----|-----|-----|-----|----|---------------|------|------|------|---|-----|---|-----|---|---------------|------|------|------|---|-----|---|-----|---|----|-------------|--|--|--|--|--|--|--|--|
| Image density                                          |                |                     |      |             |                |      |             |                |               |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Den-<br>sity                                           |                |                     |      |             |                |      |             |                |               |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Fogging                                                |                |                     |      |             | Fogging        |      |             |                |               |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| First sheet                                            | 5,000-th sheet | difference $\Delta$ | Rank | First sheet | 5,000-th sheet | Rank | First sheet | 5,000-th sheet | Rank          |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 101                                            | 1.50           | 1.48                | 0.02 | A           | 0.1            | A    | 0.2         | A              | 5             |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 102                                            | 1.50           | 1.47                | 0.03 | A           | 0.2            | A    | 0.4         | A              | Example 103   | 1.50 | 1.47 | 0.03 | A | 0.2 | A | 0.4 | A | 10            | Example 104   | 1.50 | 1.47 | 0.03 | A   | 0.2 | A   | 0.4 | A             | Example 105   | 1.50 | 1.47 | 0.03 | A   | 0.2 | A   | 0.4 | A           | 15            | Example 106 | 1.50 | 1.46 | 0.04 | A   | 0.3 | A   | 0.7         | B             | Example 107   | 1.50 | 1.46 | 0.04 | A   | 0.3 | A   | 0.7         | B             | 20            | Example 108 | 1.50 | 1.46 | 0.04 | A   | 0.3 | A           | 0.7           | B             | Example 109 | 1.50 | 1.46 | 0.04 | A   | 0.3 | A           | 0.7           | B             | 25            | Example 110 | 1.50 | 1.46 | 0.04 | A   | 0.3         | A             | 0.7           | B             | Example 111 | 1.50 | 1.46 | 0.04 | A   | 0.3         | A             | 0.7           | B             | 30          | Example 112 | 1.50 | 1.46 | 0.04 | A           | 0.3           | A             | 0.7           | B             | Example 113 | 1.50 | 1.46 | 0.04 | A           | 0.3           | A             | 0.7           | B             | 35          | Example 114 | 1.50 | 1.42 | 0.08        | B             | 0.6           | B             | 1.8           | C           | Example 115 | 1.50 | 1.41 | 0.09        | B             | 0.7           | B             | 1.2           | C           | Example 116 | 1.50 | 1.46 | 0.04        | A             | 0.3           | A             | 0.6           | B           | Example 117 | 1.50 | 1.46 | 0.04        | A             | 0.3           | A             | 0.6           | B             | Example 118 | 1.50 | 1.46 | 0.04        | A             | 0.3           | A             | 0.7           | B             | Example 119 | 1.50 | 1.44 | 0.06        | B             | 0.7           | B             | 1.4           | C             | Example 120 | 1.50 | 1.45 | 0.05        | B             | 0.3           | A             | 0.7           | B             | Example 121 | 1.50 | 1.41 | 0.09        | B             | 0.5           | B             | 1.1           | C             | Example 122 | 1.50 | 1.43 | 0.07        | B             | 0.4           | A             | 0.9           | B             | Example 123 | 1.50 | 1.41 | 0.09        | B             | 0.8           | B             | 1.2           | C             | Example 124 | 1.50 | 1.45 | 0.05 | B             | 0.3           | A             | 0.7           | B             | Example 125 | 1.50 | 1.46 | 0.04 | A             | 0.3           | A             | 0.7           | B             | Example 126 | 1.50 | 1.43 | 0.07 | B             | 0.5           | B             | 1.1           | C             | Example 127 | 1.50 | 1.41 | 0.09 | B             | 0.5           | B             | 1.0           | C             | Example 128 | 1.50 | 1.41 | 0.09 | B           | 0.6           | B             | 1.2           | C             | Example 129 | 1.50 | 1.41 | 0.09 | B   | 0.7           | B             | 1.4           | C             | Example 130 | 1.50 | 1.40 | 0.10 | C   | 0.7           | B             | 1.4           | C             | Example 131 | 1.50 | 1.42 | 0.08 | B   | 0.6           | B             | 1.2           | C             | Example 132 | 1.50 | 1.45 | 0.05 | B   | 0.3 | A             | 0.7           | B             | Example 133 | 1.50 | 1.43 | 0.07 | B   | 0.9 | B             | 1.4           | C             | Example 134 | 1.50 | 1.43 | 0.07 | B   | 0.5 | B             | 0.8           | B             | Example 135 | 1.50 | 1.42 | 0.08 | B   | 0.7 | B   | 0.9           | B             | Example 136 | 1.50 | 1.38 | 0.12 | C   | 0.9 | B   | 1.3           | C             | 40          | Example 137 | 1.50 | 1.46 | 0.04 | A   | 0.3 | A             | 0.9           | B             | Example 138 | 1.50 | 1.45 | 0.05 | B   | 0.4 | A   | 0.8           | B             | Example 139 | 1.50 | 1.46 | 0.04 | A   | 0.3 | A   | 0.7           | B             | Comparative 1 | 1.50 | 1.33 | 0.17 | D   | 1.4 | C   | 2.5           | D             | Example 101   | 1.50 | 1.46 | 0.04 | A   | 0.4 | A   | 0.8 | B             | 45            | Comparative 1 | 1.50 | 1.42 | 0.08 | B   | 1.2 | C   | 2.2           | D             | Comparative 1 | 1.50 | 1.41 | 0.09 | B   | 0.8 | B   | 1.4 | C             | Comparative 1 | 1.50 | 1.37 | 0.13 | C   | 1.0 | C   | 2.0 | D             | 50            | Comparative 1 | 1.50 | 1.45 | 0.05 | B   | 0.3 | A   | 0.7 | B             | Comparative 1 | 1.50 | 1.32 | 0.18 | D   | 0.7 | B   | 2.5 | D             | Comparative 1 | 1.50 | 1.30 | 0.20 | D   | 1.3 | C   | 2.3 | D  | 55            | Comparative 1 | 1.50 | 1.31 | 0.19 | D   | 2.0 | D   | 3.0 | D             | Comparative 1 | 1.50 | 1.38 | 0.12 | C   | 1.6 | C   | 2.6 | D  | Comparative 1 | 1.50 | 1.35 | 0.15 | D | 1.8 | C | 2.4 | D | 60            | Comparative 1 | 1.50 | 1.33 | 0.17 | D   | 1.5 | C   | 2.6 | D  | Comparative 1 | 1.50 | 1.38 | 0.12 | C | 1.5 | C | 3.5 | D | Comparative 1 | 1.50 | 1.36 | 0.14 | C | 1.8 | C | 2.4 | D | 65 | Example 114 |  |  |  |  |  |  |  |  |
| Example 103                                            | 1.50           | 1.47                | 0.03 | A           | 0.2            | A    | 0.4         | A              | 10            |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 104                                            | 1.50           | 1.47                | 0.03 | A           | 0.2            | A    | 0.4         | A              | Example 105   | 1.50 | 1.47 | 0.03 | A | 0.2 | A | 0.4 | A | 15            | Example 106   | 1.50 | 1.46 | 0.04 | A   | 0.3 | A   | 0.7 | B             | Example 107   | 1.50 | 1.46 | 0.04 | A   | 0.3 | A   | 0.7 | B           | 20            | Example 108 | 1.50 | 1.46 | 0.04 | A   | 0.3 | A   | 0.7         | B             | Example 109   | 1.50 | 1.46 | 0.04 | A   | 0.3 | A   | 0.7         | B             | 25            | Example 110 | 1.50 | 1.46 | 0.04 | A   | 0.3 | A           | 0.7           | B             | Example 111 | 1.50 | 1.46 | 0.04 | A   | 0.3 | A           | 0.7           | B             | 30            | Example 112 | 1.50 | 1.46 | 0.04 | A   | 0.3         | A             | 0.7           | B             | Example 113 | 1.50 | 1.46 | 0.04 | A   | 0.3         | A             | 0.7           | B             | 35          | Example 114 | 1.50 | 1.42 | 0.08 | B           | 0.6           | B             | 1.8           | C             | Example 115 | 1.50 | 1.41 | 0.09 | B           | 0.7           | B             | 1.2           | C             | Example 116 | 1.50        | 1.46 | 0.04 | A           | 0.3           | A             | 0.6           | B             | Example 117 | 1.50        | 1.46 | 0.04 | A           | 0.3           | A             | 0.6           | B             | Example 118 | 1.50        | 1.46 | 0.04 | A           | 0.3           | A             | 0.7           | B             | Example 119 | 1.50        | 1.44 | 0.06 | B           | 0.7           | B             | 1.4           | C             | Example 120   | 1.50        | 1.45 | 0.05 | B           | 0.3           | A             | 0.7           | B             | Example 121   | 1.50        | 1.41 | 0.09 | B           | 0.5           | B             | 1.1           | C             | Example 122   | 1.50        | 1.43 | 0.07 | B           | 0.4           | A             | 0.9           | B             | Example 123   | 1.50        | 1.41 | 0.09 | B           | 0.8           | B             | 1.2           | C             | Example 124   | 1.50        | 1.45 | 0.05 | B           | 0.3           | A             | 0.7           | B             | Example 125   | 1.50        | 1.46 | 0.04 | A           | 0.3           | A             | 0.7           | B             | Example 126   | 1.50        | 1.43 | 0.07 | B    | 0.5           | B             | 1.1           | C             | Example 127   | 1.50        | 1.41 | 0.09 | B    | 0.5           | B             | 1.0           | C             | Example 128   | 1.50        | 1.41 | 0.09 | B    | 0.6           | B             | 1.2           | C             | Example 129   | 1.50        | 1.41 | 0.09 | B    | 0.7           | B             | 1.4           | C             | Example 130   | 1.50        | 1.40 | 0.10 | C    | 0.7         | B             | 1.4           | C             | Example 131   | 1.50        | 1.42 | 0.08 | B    | 0.6 | B             | 1.2           | C             | Example 132   | 1.50        | 1.45 | 0.05 | B    | 0.3 | A             | 0.7           | B             | Example 133   | 1.50        | 1.43 | 0.07 | B    | 0.9 | B             | 1.4           | C             | Example 134   | 1.50        | 1.43 | 0.07 | B    | 0.5 | B   | 0.8           | B             | Example 135   | 1.50        | 1.42 | 0.08 | B    | 0.7 | B   | 0.9           | B             | Example 136   | 1.50        | 1.38 | 0.12 | C    | 0.9 | B   | 1.3           | C             | 40            | Example 137 | 1.50 | 1.46 | 0.04 | A   | 0.3 | A   | 0.9           | B             | Example 138 | 1.50 | 1.45 | 0.05 | B   | 0.4 | A   | 0.8           | B             | Example 139 | 1.50        | 1.46 | 0.04 | A    | 0.3 | A   | 0.7           | B             | Comparative 1 | 1.50        | 1.33 | 0.17 | D    | 1.4 | C   | 2.5 | D             | Example 101   | 1.50        | 1.46 | 0.04 | A    | 0.4 | A   | 0.8 | B             | 45            | Comparative 1 | 1.50 | 1.42 | 0.08 | B   | 1.2 | C   | 2.2           | D             | Comparative 1 | 1.50 | 1.41 | 0.09 | B   | 0.8 | B   | 1.4 | C             | Comparative 1 | 1.50          | 1.37 | 0.13 | C    | 1.0 | C   | 2.0 | D             | 50            | Comparative 1 | 1.50 | 1.45 | 0.05 | B   | 0.3 | A   | 0.7 | B             | Comparative 1 | 1.50 | 1.32 | 0.18 | D   | 0.7 | B   | 2.5 | D             | Comparative 1 | 1.50          | 1.30 | 0.20 | D    | 1.3 | C   | 2.3 | D   | 55            | Comparative 1 | 1.50 | 1.31 | 0.19 | D   | 2.0 | D   | 3.0 | D             | Comparative 1 | 1.50 | 1.38 | 0.12 | C   | 1.6 | C   | 2.6 | D  | Comparative 1 | 1.50          | 1.35 | 0.15 | D    | 1.8 | C   | 2.4 | D   | 60            | Comparative 1 | 1.50 | 1.33 | 0.17 | D   | 1.5 | C   | 2.6 | D  | Comparative 1 | 1.50 | 1.38 | 0.12 | C | 1.5 | C | 3.5 | D | Comparative 1 | 1.50          | 1.36 | 0.14 | C    | 1.8 | C   | 2.4 | D   | 65 | Example 114   |      |      |      |   |     |   |     |   |               |      |      |      |   |     |   |     |   |    |             |  |  |  |  |  |  |  |  |
| Example 105                                            | 1.50           | 1.47                | 0.03 | A           | 0.2            | A    | 0.4         | A              | 15            |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 106                                            | 1.50           | 1.46                | 0.04 | A           | 0.3            | A    | 0.7         | B              | Example 107   | 1.50 | 1.46 | 0.04 | A | 0.3 | A | 0.7 | B | 20            | Example 108   | 1.50 | 1.46 | 0.04 | A   | 0.3 | A   | 0.7 | B             | Example 109   | 1.50 | 1.46 | 0.04 | A   | 0.3 | A   | 0.7 | B           | 25            | Example 110 | 1.50 | 1.46 | 0.04 | A   | 0.3 | A   | 0.7         | B             | Example 111   | 1.50 | 1.46 | 0.04 | A   | 0.3 | A   | 0.7         | B             | 30            | Example 112 | 1.50 | 1.46 | 0.04 | A   | 0.3 | A           | 0.7           | B             | Example 113 | 1.50 | 1.46 | 0.04 | A   | 0.3 | A           | 0.7           | B             | 35            | Example 114 | 1.50 | 1.42 | 0.08 | B   | 0.6         | B             | 1.8           | C             | Example 115 | 1.50 | 1.41 | 0.09 | B   | 0.7         | B             | 1.2           | C             | Example 116 | 1.50        | 1.46 | 0.04 | A    | 0.3         | A             | 0.6           | B             | Example 117   | 1.50        | 1.46 | 0.04 | A    | 0.3         | A             | 0.6           | B             | Example 118   | 1.50        | 1.46        | 0.04 | A    | 0.3         | A             | 0.7           | B             | Example 119   | 1.50        | 1.44        | 0.06 | B    | 0.7         | B             | 1.4           | C             | Example 120   | 1.50        | 1.45        | 0.05 | B    | 0.3         | A             | 0.7           | B             | Example 121   | 1.50        | 1.41        | 0.09 | B    | 0.5         | B             | 1.1           | C             | Example 122   | 1.50          | 1.43        | 0.07 | B    | 0.4         | A             | 0.9           | B             | Example 123   | 1.50          | 1.41        | 0.09 | B    | 0.8         | B             | 1.2           | C             | Example 124   | 1.50          | 1.45        | 0.05 | B    | 0.3         | A             | 0.7           | B             | Example 125   | 1.50          | 1.46        | 0.04 | A    | 0.3         | A             | 0.7           | B             | Example 126   | 1.50          | 1.43        | 0.07 | B    | 0.5         | B             | 1.1           | C             | Example 127   | 1.50          | 1.41        | 0.09 | B    | 0.5         | B             | 1.0           | C             | Example 128   | 1.50          | 1.41        | 0.09 | B    | 0.6  | B             | 1.2           | C             | Example 129   | 1.50          | 1.41        | 0.09 | B    | 0.7  | B             | 1.4           | C             | Example 130   | 1.50          | 1.40        | 0.10 | C    | 0.7  | B             | 1.4           | C             | Example 131   | 1.50          | 1.42        | 0.08 | B    | 0.6  | B             | 1.2           | C             | Example 132   | 1.50          | 1.45        | 0.05 | B    | 0.3  | A           | 0.7           | B             | Example 133   | 1.50          | 1.43        | 0.07 | B    | 0.9  | B   | 1.4           | C             | Example 134   | 1.50          | 1.43        | 0.07 | B    | 0.5  | B   | 0.8           | B             | Example 135   | 1.50          | 1.42        | 0.08 | B    | 0.7  | B   | 0.9           | B             | Example 136   | 1.50          | 1.38        | 0.12 | C    | 0.9  | B   | 1.3 | C             | 40            | Example 137   | 1.50        | 1.46 | 0.04 | A    | 0.3 | A   | 0.9           | B             | Example 138   | 1.50        | 1.45 | 0.05 | B    | 0.4 | A   | 0.8           | B             | Example 139   | 1.50        | 1.46 | 0.04 | A    | 0.3 | A   | 0.7 | B             | Comparative 1 | 1.50        | 1.33 | 0.17 | D    | 1.4 | C   | 2.5 | D             | Example 101   | 1.50        | 1.46        | 0.04 | A    | 0.4  | A   | 0.8 | B             | 45            | Comparative 1 | 1.50        | 1.42 | 0.08 | B    | 1.2 | C   | 2.2 | D             | Comparative 1 | 1.50        | 1.41 | 0.09 | B    | 0.8 | B   | 1.4 | C             | Comparative 1 | 1.50          | 1.37 | 0.13 | C    | 1.0 | C   | 2.0 | D             | 50            | Comparative 1 | 1.50 | 1.45 | 0.05 | B   | 0.3 | A   | 0.7 | B             | Comparative 1 | 1.50          | 1.32 | 0.18 | D    | 0.7 | B   | 2.5 | D             | Comparative 1 | 1.50          | 1.30 | 0.20 | D    | 1.3 | C   | 2.3 | D   | 55            | Comparative 1 | 1.50 | 1.31 | 0.19 | D   | 2.0 | D   | 3.0 | D             | Comparative 1 | 1.50          | 1.38 | 0.12 | C    | 1.6 | C   | 2.6 | D   | Comparative 1 | 1.50          | 1.35 | 0.15 | D    | 1.8 | C   | 2.4 | D   | 60            | Comparative 1 | 1.50 | 1.33 | 0.17 | D   | 1.5 | C   | 2.6 | D  | Comparative 1 | 1.50          | 1.38 | 0.12 | C    | 1.5 | C   | 3.5 | D   | Comparative 1 | 1.50          | 1.36 | 0.14 | C    | 1.8 | C   | 2.4 | D   | 65 | Example 114   |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 107                                            | 1.50           | 1.46                | 0.04 | A           | 0.3            | A    | 0.7         | B              | 20            |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 108                                            | 1.50           | 1.46                | 0.04 | A           | 0.3            | A    | 0.7         | B              | Example 109   | 1.50 | 1.46 | 0.04 | A | 0.3 | A | 0.7 | B | 25            | Example 110   | 1.50 | 1.46 | 0.04 | A   | 0.3 | A   | 0.7 | B             | Example 111   | 1.50 | 1.46 | 0.04 | A   | 0.3 | A   | 0.7 | B           | 30            | Example 112 | 1.50 | 1.46 | 0.04 | A   | 0.3 | A   | 0.7         | B             | Example 113   | 1.50 | 1.46 | 0.04 | A   | 0.3 | A   | 0.7         | B             | 35            | Example 114 | 1.50 | 1.42 | 0.08 | B   | 0.6 | B           | 1.8           | C             | Example 115 | 1.50 | 1.41 | 0.09 | B   | 0.7 | B           | 1.2           | C             | Example 116   | 1.50        | 1.46 | 0.04 | A    | 0.3 | A           | 0.6           | B             | Example 117   | 1.50        | 1.46 | 0.04 | A    | 0.3 | A           | 0.6           | B             | Example 118   | 1.50        | 1.46        | 0.04 | A    | 0.3  | A           | 0.7           | B             | Example 119   | 1.50          | 1.44        | 0.06 | B    | 0.7  | B           | 1.4           | C             | Example 120   | 1.50          | 1.45        | 0.05        | B    | 0.3  | A           | 0.7           | B             | Example 121   | 1.50          | 1.41        | 0.09        | B    | 0.5  | B           | 1.1           | C             | Example 122   | 1.50          | 1.43        | 0.07        | B    | 0.4  | A           | 0.9           | B             | Example 123   | 1.50          | 1.41        | 0.09        | B    | 0.8  | B           | 1.2           | C             | Example 124   | 1.50          | 1.45          | 0.05        | B    | 0.3  | A           | 0.7           | B             | Example 125   | 1.50          | 1.46          | 0.04        | A    | 0.3  | A           | 0.7           | B             | Example 126   | 1.50          | 1.43          | 0.07        | B    | 0.5  | B           | 1.1           | C             | Example 127   | 1.50          | 1.41          | 0.09        | B    | 0.5  | B           | 1.0           | C             | Example 128   | 1.50          | 1.41          | 0.09        | B    | 0.6  | B           | 1.2           | C             | Example 129   | 1.50          | 1.41          | 0.09        | B    | 0.7  | B           | 1.4           | C             | Example 130   | 1.50          | 1.40          | 0.10        | C    | 0.7  | B    | 1.4           | C             | Example 131   | 1.50          | 1.42          | 0.08        | B    | 0.6  | B    | 1.2           | C             | Example 132   | 1.50          | 1.45          | 0.05        | B    | 0.3  | A    | 0.7           | B             | Example 133   | 1.50          | 1.43          | 0.07        | B    | 0.9  | B    | 1.4           | C             | Example 134   | 1.50          | 1.43          | 0.07        | B    | 0.5  | B    | 0.8         | B             | Example 135   | 1.50          | 1.42          | 0.08        | B    | 0.7  | B    | 0.9 | B             | Example 136   | 1.50          | 1.38          | 0.12        | C    | 0.9  | B    | 1.3 | C             | 40            | Example 137   | 1.50          | 1.46        | 0.04 | A    | 0.3  | A   | 0.9           | B             | Example 138   | 1.50          | 1.45        | 0.05 | B    | 0.4  | A   | 0.8 | B             | Example 139   | 1.50          | 1.46        | 0.04 | A    | 0.3  | A   | 0.7 | B             | Comparative 1 | 1.50          | 1.33        | 0.17 | D    | 1.4  | C   | 2.5 | D             | Example 101   | 1.50          | 1.46        | 0.04 | A    | 0.4  | A   | 0.8 | B   | 45            | Comparative 1 | 1.50        | 1.42 | 0.08 | B    | 1.2 | C   | 2.2 | D             | Comparative 1 | 1.50        | 1.41        | 0.09 | B    | 0.8  | B   | 1.4 | C             | Comparative 1 | 1.50          | 1.37        | 0.13 | C    | 1.0  | C   | 2.0 | D   | 50            | Comparative 1 | 1.50        | 1.45 | 0.05 | B    | 0.3 | A   | 0.7 | B             | Comparative 1 | 1.50          | 1.32 | 0.18 | D    | 0.7 | B   | 2.5 | D             | Comparative 1 | 1.50          | 1.30 | 0.20 | D    | 1.3 | C   | 2.3 | D   | 55            | Comparative 1 | 1.50          | 1.31 | 0.19 | D    | 2.0 | D   | 3.0 | D             | Comparative 1 | 1.50          | 1.38 | 0.12 | C    | 1.6 | C   | 2.6 | D   | Comparative 1 | 1.50          | 1.35 | 0.15 | D    | 1.8 | C   | 2.4 | D   | 60            | Comparative 1 | 1.50          | 1.33 | 0.17 | D    | 1.5 | C   | 2.6 | D   | Comparative 1 | 1.50          | 1.38 | 0.12 | C    | 1.5 | C   | 3.5 | D   | Comparative 1 | 1.50          | 1.36 | 0.14 | C    | 1.8 | C   | 2.4 | D   | 65 | Example 114   |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 109                                            | 1.50           | 1.46                | 0.04 | A           | 0.3            | A    | 0.7         | B              | 25            |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 110                                            | 1.50           | 1.46                | 0.04 | A           | 0.3            | A    | 0.7         | B              | Example 111   | 1.50 | 1.46 | 0.04 | A | 0.3 | A | 0.7 | B | 30            | Example 112   | 1.50 | 1.46 | 0.04 | A   | 0.3 | A   | 0.7 | B             | Example 113   | 1.50 | 1.46 | 0.04 | A   | 0.3 | A   | 0.7 | B           | 35            | Example 114 | 1.50 | 1.42 | 0.08 | B   | 0.6 | B   | 1.8         | C             | Example 115   | 1.50 | 1.41 | 0.09 | B   | 0.7 | B   | 1.2         | C             | Example 116   | 1.50        | 1.46 | 0.04 | A    | 0.3 | A   | 0.6         | B             | Example 117   | 1.50        | 1.46 | 0.04 | A    | 0.3 | A   | 0.6         | B             | Example 118   | 1.50          | 1.46        | 0.04 | A    | 0.3  | A   | 0.7         | B             | Example 119   | 1.50          | 1.44        | 0.06 | B    | 0.7  | B   | 1.4         | C             | Example 120   | 1.50          | 1.45        | 0.05        | B    | 0.3  | A    | 0.7         | B             | Example 121   | 1.50          | 1.41          | 0.09        | B    | 0.5  | B    | 1.1         | C             | Example 122   | 1.50          | 1.43          | 0.07        | B           | 0.4  | A    | 0.9         | B             | Example 123   | 1.50          | 1.41          | 0.09        | B           | 0.8  | B    | 1.2         | C             | Example 124   | 1.50          | 1.45          | 0.05        | B           | 0.3  | A    | 0.7         | B             | Example 125   | 1.50          | 1.46          | 0.04        | A           | 0.3  | A    | 0.7         | B             | Example 126   | 1.50          | 1.43          | 0.07          | B           | 0.5  | B    | 1.1         | C             | Example 127   | 1.50          | 1.41          | 0.09          | B           | 0.5  | B    | 1.0         | C             | Example 128   | 1.50          | 1.41          | 0.09          | B           | 0.6  | B    | 1.2         | C             | Example 129   | 1.50          | 1.41          | 0.09          | B           | 0.7  | B    | 1.4         | C             | Example 130   | 1.50          | 1.40          | 0.10          | C           | 0.7  | B    | 1.4         | C             | Example 131   | 1.50          | 1.42          | 0.08          | B           | 0.6  | B    | 1.2         | C             | Example 132   | 1.50          | 1.45          | 0.05          | B           | 0.3  | A    | 0.7  | B             | Example 133   | 1.50          | 1.43          | 0.07          | B           | 0.9  | B    | 1.4  | C             | Example 134   | 1.50          | 1.43          | 0.07          | B           | 0.5  | B    | 0.8  | B             | Example 135   | 1.50          | 1.42          | 0.08          | B           | 0.7  | B    | 0.9  | B             | Example 136   | 1.50          | 1.38          | 0.12          | C           | 0.9  | B    | 1.3  | C           | 40            | Example 137   | 1.50          | 1.46          | 0.04        | A    | 0.3  | A    | 0.9 | B             | Example 138   | 1.50          | 1.45          | 0.05        | B    | 0.4  | A    | 0.8 | B             | Example 139   | 1.50          | 1.46          | 0.04        | A    | 0.3  | A    | 0.7 | B             | Comparative 1 | 1.50          | 1.33          | 0.17        | D    | 1.4  | C    | 2.5 | D   | Example 101   | 1.50          | 1.46          | 0.04        | A    | 0.4  | A    | 0.8 | B   | 45            | Comparative 1 | 1.50          | 1.42        | 0.08 | B    | 1.2  | C   | 2.2 | D             | Comparative 1 | 1.50          | 1.41        | 0.09 | B    | 0.8  | B   | 1.4 | C   | Comparative 1 | 1.50          | 1.37        | 0.13 | C    | 1.0  | C   | 2.0 | D   | 50            | Comparative 1 | 1.50        | 1.45        | 0.05 | B    | 0.3  | A   | 0.7 | B             | Comparative 1 | 1.50          | 1.32        | 0.18 | D    | 0.7  | B   | 2.5 | D   | Comparative 1 | 1.50          | 1.30        | 0.20 | D    | 1.3  | C   | 2.3 | D   | 55            | Comparative 1 | 1.50          | 1.31 | 0.19 | D    | 2.0 | D   | 3.0 | D             | Comparative 1 | 1.50          | 1.38 | 0.12 | C    | 1.6 | C   | 2.6 | D   | Comparative 1 | 1.50          | 1.35          | 0.15 | D    | 1.8  | C   | 2.4 | D   | 60            | Comparative 1 | 1.50          | 1.33 | 0.17 | D    | 1.5 | C   | 2.6 | D   | Comparative 1 | 1.50          | 1.38 | 0.12 | C    | 1.5 | C   | 3.5 | D   | Comparative 1 | 1.50          | 1.36          | 0.14 | C    | 1.8  | C   | 2.4 | D   | 65  | Example 114   |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 111                                            | 1.50           | 1.46                | 0.04 | A           | 0.3            | A    | 0.7         | B              | 30            |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 112                                            | 1.50           | 1.46                | 0.04 | A           | 0.3            | A    | 0.7         | B              | Example 113   | 1.50 | 1.46 | 0.04 | A | 0.3 | A | 0.7 | B | 35            | Example 114   | 1.50 | 1.42 | 0.08 | B   | 0.6 | B   | 1.8 | C             | Example 115   | 1.50 | 1.41 | 0.09 | B   | 0.7 | B   | 1.2 | C           | Example 116   | 1.50        | 1.46 | 0.04 | A    | 0.3 | A   | 0.6 | B           | Example 117   | 1.50          | 1.46 | 0.04 | A    | 0.3 | A   | 0.6 | B           | Example 118   | 1.50          | 1.46        | 0.04 | A    | 0.3  | A   | 0.7 | B           | Example 119   | 1.50          | 1.44        | 0.06 | B    | 0.7  | B   | 1.4 | C           | Example 120   | 1.50          | 1.45          | 0.05        | B    | 0.3  | A    | 0.7 | B           | Example 121   | 1.50          | 1.41          | 0.09        | B    | 0.5  | B    | 1.1 | C           | Example 122   | 1.50          | 1.43          | 0.07        | B           | 0.4  | A    | 0.9  | B           | Example 123   | 1.50          | 1.41          | 0.09          | B           | 0.8  | B    | 1.2  | C           | Example 124   | 1.50          | 1.45          | 0.05          | B           | 0.3         | A    | 0.7  | B           | Example 125   | 1.50          | 1.46          | 0.04          | A           | 0.3         | A    | 0.7  | B           | Example 126   | 1.50          | 1.43          | 0.07          | B           | 0.5         | B    | 1.1  | C           | Example 127   | 1.50          | 1.41          | 0.09          | B           | 0.5         | B    | 1.0  | C           | Example 128   | 1.50          | 1.41          | 0.09          | B             | 0.6         | B    | 1.2  | C           | Example 129   | 1.50          | 1.41          | 0.09          | B             | 0.7         | B    | 1.4  | C           | Example 130   | 1.50          | 1.40          | 0.10          | C             | 0.7         | B    | 1.4  | C           | Example 131   | 1.50          | 1.42          | 0.08          | B             | 0.6         | B    | 1.2  | C           | Example 132   | 1.50          | 1.45          | 0.05          | B             | 0.3         | A    | 0.7  | B           | Example 133   | 1.50          | 1.43          | 0.07          | B             | 0.9         | B    | 1.4  | C           | Example 134   | 1.50          | 1.43          | 0.07          | B             | 0.5         | B    | 0.8  | B    | Example 135   | 1.50          | 1.42          | 0.08          | B             | 0.7         | B    | 0.9  | B    | Example 136   | 1.50          | 1.38          | 0.12          | C             | 0.9         | B    | 1.3  | C    | 40            | Example 137   | 1.50          | 1.46          | 0.04          | A           | 0.3  | A    | 0.9  | B             | Example 138   | 1.50          | 1.45          | 0.05          | B           | 0.4  | A    | 0.8  | B           | Example 139   | 1.50          | 1.46          | 0.04          | A           | 0.3  | A    | 0.7  | B   | Comparative 1 | 1.50          | 1.33          | 0.17          | D           | 1.4  | C    | 2.5  | D   | Example 101   | 1.50          | 1.46          | 0.04          | A           | 0.4  | A    | 0.8  | B   | 45            | Comparative 1 | 1.50          | 1.42          | 0.08        | B    | 1.2  | C    | 2.2 | D   | Comparative 1 | 1.50          | 1.41          | 0.09        | B    | 0.8  | B    | 1.4 | C   | Comparative 1 | 1.50          | 1.37          | 0.13        | C    | 1.0  | C    | 2.0 | D   | 50            | Comparative 1 | 1.50          | 1.45        | 0.05 | B    | 0.3  | A   | 0.7 | B   | Comparative 1 | 1.50          | 1.32        | 0.18 | D    | 0.7  | B   | 2.5 | D   | Comparative 1 | 1.50          | 1.30        | 0.20        | D    | 1.3  | C    | 2.3 | D   | 55            | Comparative 1 | 1.50          | 1.31        | 0.19 | D    | 2.0  | D   | 3.0 | D   | Comparative 1 | 1.50          | 1.38        | 0.12 | C    | 1.6  | C   | 2.6 | D   | Comparative 1 | 1.50          | 1.35          | 0.15 | D    | 1.8  | C   | 2.4 | D   | 60            | Comparative 1 | 1.50          | 1.33 | 0.17 | D    | 1.5 | C   | 2.6 | D   | Comparative 1 | 1.50          | 1.38          | 0.12 | C    | 1.5  | C   | 3.5 | D   | Comparative 1 | 1.50          | 1.36          | 0.14 | C    | 1.8  | C   | 2.4 | D   | 65  | Example 114   |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 113                                            | 1.50           | 1.46                | 0.04 | A           | 0.3            | A    | 0.7         | B              | 35            |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 114                                            | 1.50           | 1.42                | 0.08 | B           | 0.6            | B    | 1.8         | C              | Example 115   | 1.50 | 1.41 | 0.09 | B | 0.7 | B | 1.2 | C | Example 116   | 1.50          | 1.46 | 0.04 | A    | 0.3 | A   | 0.6 | B   | Example 117   | 1.50          | 1.46 | 0.04 | A    | 0.3 | A   | 0.6 | B   | Example 118 | 1.50          | 1.46        | 0.04 | A    | 0.3  | A   | 0.7 | B   | Example 119 | 1.50          | 1.44          | 0.06 | B    | 0.7  | B   | 1.4 | C   | Example 120 | 1.50          | 1.45          | 0.05        | B    | 0.3  | A    | 0.7 | B   | Example 121 | 1.50          | 1.41          | 0.09        | B    | 0.5  | B    | 1.1 | C   | Example 122 | 1.50          | 1.43          | 0.07          | B           | 0.4  | A    | 0.9  | B   | Example 123 | 1.50          | 1.41          | 0.09          | B           | 0.8  | B    | 1.2  | C   | Example 124 | 1.50          | 1.45          | 0.05          | B           | 0.3         | A    | 0.7  | B    | Example 125 | 1.50          | 1.46          | 0.04          | A             | 0.3         | A    | 0.7  | B    | Example 126 | 1.50          | 1.43          | 0.07          | B             | 0.5         | B           | 1.1  | C    | Example 127 | 1.50          | 1.41          | 0.09          | B             | 0.5         | B           | 1.0  | C    | Example 128 | 1.50          | 1.41          | 0.09          | B             | 0.6         | B           | 1.2  | C    | Example 129 | 1.50          | 1.41          | 0.09          | B             | 0.7         | B           | 1.4  | C    | Example 130 | 1.50          | 1.40          | 0.10          | C             | 0.7           | B           | 1.4  | C    | Example 131 | 1.50          | 1.42          | 0.08          | B             | 0.6           | B           | 1.2  | C    | Example 132 | 1.50          | 1.45          | 0.05          | B             | 0.3           | A           | 0.7  | B    | Example 133 | 1.50          | 1.43          | 0.07          | B             | 0.9           | B           | 1.4  | C    | Example 134 | 1.50          | 1.43          | 0.07          | B             | 0.5           | B           | 0.8  | B    | Example 135 | 1.50          | 1.42          | 0.08          | B             | 0.7           | B           | 0.9  | B    | Example 136 | 1.50          | 1.38          | 0.12          | C             | 0.9           | B           | 1.3  | C    | 40   | Example 137   | 1.50          | 1.46          | 0.04          | A             | 0.3         | A    | 0.9  | B    | Example 138   | 1.50          | 1.45          | 0.05          | B             | 0.4         | A    | 0.8  | B    | Example 139   | 1.50          | 1.46          | 0.04          | A             | 0.3         | A    | 0.7  | B    | Comparative 1 | 1.50          | 1.33          | 0.17          | D             | 1.4         | C    | 2.5  | D    | Example 101 | 1.50          | 1.46          | 0.04          | A             | 0.4         | A    | 0.8  | B    | 45  | Comparative 1 | 1.50          | 1.42          | 0.08          | B           | 1.2  | C    | 2.2  | D   | Comparative 1 | 1.50          | 1.41          | 0.09          | B           | 0.8  | B    | 1.4  | C   | Comparative 1 | 1.50          | 1.37          | 0.13          | C           | 1.0  | C    | 2.0  | D   | 50  | Comparative 1 | 1.50          | 1.45          | 0.05        | B    | 0.3  | A    | 0.7 | B   | Comparative 1 | 1.50          | 1.32          | 0.18        | D    | 0.7  | B    | 2.5 | D   | Comparative 1 | 1.50          | 1.30          | 0.20        | D    | 1.3  | C    | 2.3 | D   | 55  | Comparative 1 | 1.50          | 1.31        | 0.19 | D    | 2.0  | D   | 3.0 | D   | Comparative 1 | 1.50          | 1.38        | 0.12        | C    | 1.6  | C    | 2.6 | D   | Comparative 1 | 1.50          | 1.35          | 0.15        | D    | 1.8  | C    | 2.4 | D   | 60  | Comparative 1 | 1.50          | 1.33        | 0.17 | D    | 1.5  | C   | 2.6 | D   | Comparative 1 | 1.50          | 1.38          | 0.12 | C    | 1.5  | C   | 3.5 | D   | Comparative 1 | 1.50          | 1.36          | 0.14 | C    | 1.8  | C   | 2.4 | D   | 65  | Example 114   |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 115                                            | 1.50           | 1.41                | 0.09 | B           | 0.7            | B    | 1.2         | C              | Example 116   | 1.50 | 1.46 | 0.04 | A | 0.3 | A | 0.6 | B | Example 117   | 1.50          | 1.46 | 0.04 | A    | 0.3 | A   | 0.6 | B   | Example 118   | 1.50          | 1.46 | 0.04 | A    | 0.3 | A   | 0.7 | B   | Example 119 | 1.50          | 1.44        | 0.06 | B    | 0.7  | B   | 1.4 | C   | Example 120 | 1.50          | 1.45          | 0.05 | B    | 0.3  | A   | 0.7 | B   | Example 121 | 1.50          | 1.41          | 0.09        | B    | 0.5  | B    | 1.1 | C   | Example 122 | 1.50          | 1.43          | 0.07        | B    | 0.4  | A    | 0.9 | B   | Example 123 | 1.50          | 1.41          | 0.09          | B           | 0.8  | B    | 1.2  | C   | Example 124 | 1.50          | 1.45          | 0.05          | B           | 0.3  | A    | 0.7  | B   | Example 125 | 1.50          | 1.46          | 0.04          | A           | 0.3         | A    | 0.7  | B    | Example 126 | 1.50          | 1.43          | 0.07          | B             | 0.5         | B    | 1.1  | C    | Example 127 | 1.50          | 1.41          | 0.09          | B             | 0.5         | B           | 1.0  | C    | Example 128 | 1.50          | 1.41          | 0.09          | B             | 0.6         | B           | 1.2  | C    | Example 129 | 1.50          | 1.41          | 0.09          | B             | 0.7         | B           | 1.4  | C    | Example 130 | 1.50          | 1.40          | 0.10          | C             | 0.7         | B           | 1.4  | C    | Example 131 | 1.50          | 1.42          | 0.08          | B             | 0.6           | B           | 1.2  | C    | Example 132 | 1.50          | 1.45          | 0.05          | B             | 0.3           | A           | 0.7  | B    | Example 133 | 1.50          | 1.43          | 0.07          | B             | 0.9           | B           | 1.4  | C    | Example 134 | 1.50          | 1.43          | 0.07          | B             | 0.5           | B           | 0.8  | B    | Example 135 | 1.50          | 1.42          | 0.08          | B             | 0.7           | B           | 0.9  | B    | Example 136 | 1.50          | 1.38          | 0.12          | C             | 0.9           | B           | 1.3  | C    | 40          | Example 137   | 1.50          | 1.46          | 0.04          | A             | 0.3         | A    | 0.9  | B    | Example 138   | 1.50          | 1.45          | 0.05          | B             | 0.4         | A    | 0.8  | B    | Example 139   | 1.50          | 1.46          | 0.04          | A             | 0.3         | A    | 0.7  | B    | Comparative 1 | 1.50          | 1.33          | 0.17          | D             | 1.4         | C    | 2.5  | D    | Example 101   | 1.50          | 1.46          | 0.04          | A             | 0.4         | A    | 0.8  | B    | 45          | Comparative 1 | 1.50          | 1.42          | 0.08          | B           | 1.2  | C    | 2.2  | D   | Comparative 1 | 1.50          | 1.41          | 0.09          | B           | 0.8  | B    | 1.4  | C   | Comparative 1 | 1.50          | 1.37          | 0.13          | C           | 1.0  | C    | 2.0  | D   | 50            | Comparative 1 | 1.50          | 1.45          | 0.05        | B    | 0.3  | A    | 0.7 | B   | Comparative 1 | 1.50          | 1.32          | 0.18        | D    | 0.7  | B    | 2.5 | D   | Comparative 1 | 1.50          | 1.30          | 0.20        | D    | 1.3  | C    | 2.3 | D   | 55            | Comparative 1 | 1.50          | 1.31        | 0.19 | D    | 2.0  | D   | 3.0 | D   | Comparative 1 | 1.50          | 1.38        | 0.12 | C    | 1.6  | C   | 2.6 | D   | Comparative 1 | 1.50          | 1.35        | 0.15        | D    | 1.8  | C    | 2.4 | D   | 60            | Comparative 1 | 1.50          | 1.33        | 0.17 | D    | 1.5  | C   | 2.6 | D   | Comparative 1 | 1.50          | 1.38        | 0.12 | C    | 1.5  | C   | 3.5 | D   | Comparative 1 | 1.50          | 1.36          | 0.14 | C    | 1.8  | C   | 2.4 | D   | 65            | Example 114   |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 116                                            | 1.50           | 1.46                | 0.04 | A           | 0.3            | A    | 0.6         | B              | Example 117   | 1.50 | 1.46 | 0.04 | A | 0.3 | A | 0.6 | B | Example 118   | 1.50          | 1.46 | 0.04 | A    | 0.3 | A   | 0.7 | B   | Example 119   | 1.50          | 1.44 | 0.06 | B    | 0.7 | B   | 1.4 | C   | Example 120 | 1.50          | 1.45        | 0.05 | B    | 0.3  | A   | 0.7 | B   | Example 121 | 1.50          | 1.41          | 0.09 | B    | 0.5  | B   | 1.1 | C   | Example 122 | 1.50          | 1.43          | 0.07        | B    | 0.4  | A    | 0.9 | B   | Example 123 | 1.50          | 1.41          | 0.09        | B    | 0.8  | B    | 1.2 | C   | Example 124 | 1.50          | 1.45          | 0.05          | B           | 0.3  | A    | 0.7  | B   | Example 125 | 1.50          | 1.46          | 0.04          | A           | 0.3  | A    | 0.7  | B   | Example 126 | 1.50          | 1.43          | 0.07          | B           | 0.5         | B    | 1.1  | C    | Example 127 | 1.50          | 1.41          | 0.09          | B             | 0.5         | B    | 1.0  | C    | Example 128 | 1.50          | 1.41          | 0.09          | B             | 0.6         | B           | 1.2  | C    | Example 129 | 1.50          | 1.41          | 0.09          | B             | 0.7         | B           | 1.4  | C    | Example 130 | 1.50          | 1.40          | 0.10          | C             | 0.7         | B           | 1.4  | C    | Example 131 | 1.50          | 1.42          | 0.08          | B             | 0.6         | B           | 1.2  | C    | Example 132 | 1.50          | 1.45          | 0.05          | B             | 0.3           | A           | 0.7  | B    | Example 133 | 1.50          | 1.43          | 0.07          | B             | 0.9           | B           | 1.4  | C    | Example 134 | 1.50          | 1.43          | 0.07          | B             | 0.5           | B           | 0.8  | B    | Example 135 | 1.50          | 1.42          | 0.08          | B             | 0.7           | B           | 0.9  | B    | Example 136 | 1.50          | 1.38          | 0.12          | C             | 0.9           | B           | 1.3  | C    | 40          | Example 137   | 1.50          | 1.46          | 0.04          | A             | 0.3         | A    | 0.9  | B           | Example 138   | 1.50          | 1.45          | 0.05          | B             | 0.4         | A    | 0.8  | B    | Example 139   | 1.50          | 1.46          | 0.04          | A             | 0.3         | A    | 0.7  | B    | Comparative 1 | 1.50          | 1.33          | 0.17          | D             | 1.4         | C    | 2.5  | D    | Example 101   | 1.50          | 1.46          | 0.04          | A             | 0.4         | A    | 0.8  | B    | 45            | Comparative 1 | 1.50          | 1.42          | 0.08          | B           | 1.2  | C    | 2.2  | D           | Comparative 1 | 1.50          | 1.41          | 0.09          | B           | 0.8  | B    | 1.4  | C   | Comparative 1 | 1.50          | 1.37          | 0.13          | C           | 1.0  | C    | 2.0  | D   | 50            | Comparative 1 | 1.50          | 1.45          | 0.05        | B    | 0.3  | A    | 0.7 | B             | Comparative 1 | 1.50          | 1.32          | 0.18        | D    | 0.7  | B    | 2.5 | D   | Comparative 1 | 1.50          | 1.30          | 0.20        | D    | 1.3  | C    | 2.3 | D   | 55            | Comparative 1 | 1.50          | 1.31        | 0.19 | D    | 2.0  | D   | 3.0 | D             | Comparative 1 | 1.50          | 1.38        | 0.12 | C    | 1.6  | C   | 2.6 | D   | Comparative 1 | 1.50          | 1.35        | 0.15 | D    | 1.8  | C   | 2.4 | D   | 60            | Comparative 1 | 1.50        | 1.33        | 0.17 | D    | 1.5  | C   | 2.6 | D             | Comparative 1 | 1.50          | 1.38        | 0.12 | C    | 1.5  | C   | 3.5 | D   | Comparative 1 | 1.50          | 1.36        | 0.14 | C    | 1.8  | C   | 2.4 | D   | 65            | Example 114   |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 117                                            | 1.50           | 1.46                | 0.04 | A           | 0.3            | A    | 0.6         | B              | Example 118   | 1.50 | 1.46 | 0.04 | A | 0.3 | A | 0.7 | B | Example 119   | 1.50          | 1.44 | 0.06 | B    | 0.7 | B   | 1.4 | C   | Example 120   | 1.50          | 1.45 | 0.05 | B    | 0.3 | A   | 0.7 | B   | Example 121 | 1.50          | 1.41        | 0.09 | B    | 0.5  | B   | 1.1 | C   | Example 122 | 1.50          | 1.43          | 0.07 | B    | 0.4  | A   | 0.9 | B   | Example 123 | 1.50          | 1.41          | 0.09        | B    | 0.8  | B    | 1.2 | C   | Example 124 | 1.50          | 1.45          | 0.05        | B    | 0.3  | A    | 0.7 | B   | Example 125 | 1.50          | 1.46          | 0.04          | A           | 0.3  | A    | 0.7  | B   | Example 126 | 1.50          | 1.43          | 0.07          | B           | 0.5  | B    | 1.1  | C   | Example 127 | 1.50          | 1.41          | 0.09          | B           | 0.5         | B    | 1.0  | C    | Example 128 | 1.50          | 1.41          | 0.09          | B             | 0.6         | B    | 1.2  | C    | Example 129 | 1.50          | 1.41          | 0.09          | B             | 0.7         | B           | 1.4  | C    | Example 130 | 1.50          | 1.40          | 0.10          | C             | 0.7         | B           | 1.4  | C    | Example 131 | 1.50          | 1.42          | 0.08          | B             | 0.6         | B           | 1.2  | C    | Example 132 | 1.50          | 1.45          | 0.05          | B             | 0.3         | A           | 0.7  | B    | Example 133 | 1.50          | 1.43          | 0.07          | B             | 0.9           | B           | 1.4  | C    | Example 134 | 1.50          | 1.43          | 0.07          | B             | 0.5           | B           | 0.8  | B    | Example 135 | 1.50          | 1.42          | 0.08          | B             | 0.7           | B           | 0.9  | B    | Example 136 | 1.50          | 1.38          | 0.12          | C             | 0.9           | B           | 1.3  | C    | 40          | Example 137   | 1.50          | 1.46          | 0.04          | A             | 0.3         | A    | 0.9  | B           | Example 138   | 1.50          | 1.45          | 0.05          | B             | 0.4         | A    | 0.8  | B           | Example 139   | 1.50          | 1.46          | 0.04          | A             | 0.3         | A    | 0.7  | B    | Comparative 1 | 1.50          | 1.33          | 0.17          | D             | 1.4         | C    | 2.5  | D    | Example 101   | 1.50          | 1.46          | 0.04          | A             | 0.4         | A    | 0.8  | B    | 45            | Comparative 1 | 1.50          | 1.42          | 0.08          | B           | 1.2  | C    | 2.2  | D             | Comparative 1 | 1.50          | 1.41          | 0.09          | B           | 0.8  | B    | 1.4  | C           | Comparative 1 | 1.50          | 1.37          | 0.13          | C           | 1.0  | C    | 2.0  | D   | 50            | Comparative 1 | 1.50          | 1.45          | 0.05        | B    | 0.3  | A    | 0.7 | B             | Comparative 1 | 1.50          | 1.32          | 0.18        | D    | 0.7  | B    | 2.5 | D             | Comparative 1 | 1.50          | 1.30          | 0.20        | D    | 1.3  | C    | 2.3 | D   | 55            | Comparative 1 | 1.50          | 1.31        | 0.19 | D    | 2.0  | D   | 3.0 | D             | Comparative 1 | 1.50          | 1.38        | 0.12 | C    | 1.6  | C   | 2.6 | D             | Comparative 1 | 1.50          | 1.35        | 0.15 | D    | 1.8  | C   | 2.4 | D   | 60            | Comparative 1 | 1.50        | 1.33 | 0.17 | D    | 1.5 | C   | 2.6 | D             | Comparative 1 | 1.50        | 1.38        | 0.12 | C    | 1.5  | C   | 3.5 | D             | Comparative 1 | 1.50          | 1.36        | 0.14 | C    | 1.8  | C   | 2.4 | D   | 65            | Example 114   |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 118                                            | 1.50           | 1.46                | 0.04 | A           | 0.3            | A    | 0.7         | B              | Example 119   | 1.50 | 1.44 | 0.06 | B | 0.7 | B | 1.4 | C | Example 120   | 1.50          | 1.45 | 0.05 | B    | 0.3 | A   | 0.7 | B   | Example 121   | 1.50          | 1.41 | 0.09 | B    | 0.5 | B   | 1.1 | C   | Example 122 | 1.50          | 1.43        | 0.07 | B    | 0.4  | A   | 0.9 | B   | Example 123 | 1.50          | 1.41          | 0.09 | B    | 0.8  | B   | 1.2 | C   | Example 124 | 1.50          | 1.45          | 0.05        | B    | 0.3  | A    | 0.7 | B   | Example 125 | 1.50          | 1.46          | 0.04        | A    | 0.3  | A    | 0.7 | B   | Example 126 | 1.50          | 1.43          | 0.07          | B           | 0.5  | B    | 1.1  | C   | Example 127 | 1.50          | 1.41          | 0.09          | B           | 0.5  | B    | 1.0  | C   | Example 128 | 1.50          | 1.41          | 0.09          | B           | 0.6         | B    | 1.2  | C    | Example 129 | 1.50          | 1.41          | 0.09          | B             | 0.7         | B    | 1.4  | C    | Example 130 | 1.50          | 1.40          | 0.10          | C             | 0.7         | B           | 1.4  | C    | Example 131 | 1.50          | 1.42          | 0.08          | B             | 0.6         | B           | 1.2  | C    | Example 132 | 1.50          | 1.45          | 0.05          | B             | 0.3         | A           | 0.7  | B    | Example 133 | 1.50          | 1.43          | 0.07          | B             | 0.9         | B           | 1.4  | C    | Example 134 | 1.50          | 1.43          | 0.07          | B             | 0.5           | B           | 0.8  | B    | Example 135 | 1.50          | 1.42          | 0.08          | B             | 0.7           | B           | 0.9  | B    | Example 136 | 1.50          | 1.38          | 0.12          | C             | 0.9           | B           | 1.3  | C    | 40          | Example 137   | 1.50          | 1.46          | 0.04          | A             | 0.3         | A    | 0.9  | B           | Example 138   | 1.50          | 1.45          | 0.05          | B             | 0.4         | A    | 0.8  | B           | Example 139   | 1.50          | 1.46          | 0.04          | A             | 0.3         | A    | 0.7  | B           | Comparative 1 | 1.50          | 1.33          | 0.17          | D             | 1.4         | C    | 2.5  | D    | Example 101   | 1.50          | 1.46          | 0.04          | A             | 0.4         | A    | 0.8  | B    | 45            | Comparative 1 | 1.50          | 1.42          | 0.08          | B           | 1.2  | C    | 2.2  | D             | Comparative 1 | 1.50          | 1.41          | 0.09          | B           | 0.8  | B    | 1.4  | C             | Comparative 1 | 1.50          | 1.37          | 0.13          | C           | 1.0  | C    | 2.0  | D           | 50            | Comparative 1 | 1.50          | 1.45          | 0.05        | B    | 0.3  | A    | 0.7 | B             | Comparative 1 | 1.50          | 1.32          | 0.18        | D    | 0.7  | B    | 2.5 | D             | Comparative 1 | 1.50          | 1.30          | 0.20        | D    | 1.3  | C    | 2.3 | D             | 55            | Comparative 1 | 1.50          | 1.31        | 0.19 | D    | 2.0  | D   | 3.0 | D             | Comparative 1 | 1.50          | 1.38        | 0.12 | C    | 1.6  | C   | 2.6 | D             | Comparative 1 | 1.50          | 1.35        | 0.15 | D    | 1.8  | C   | 2.4 | D             | 60            | Comparative 1 | 1.50        | 1.33 | 0.17 | D    | 1.5 | C   | 2.6 | D             | Comparative 1 | 1.50        | 1.38 | 0.12 | C    | 1.5 | C   | 3.5 | D             | Comparative 1 | 1.50        | 1.36        | 0.14 | C    | 1.8  | C   | 2.4 | D             | 65            | Example 114   |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 119                                            | 1.50           | 1.44                | 0.06 | B           | 0.7            | B    | 1.4         | C              | Example 120   | 1.50 | 1.45 | 0.05 | B | 0.3 | A | 0.7 | B | Example 121   | 1.50          | 1.41 | 0.09 | B    | 0.5 | B   | 1.1 | C   | Example 122   | 1.50          | 1.43 | 0.07 | B    | 0.4 | A   | 0.9 | B   | Example 123 | 1.50          | 1.41        | 0.09 | B    | 0.8  | B   | 1.2 | C   | Example 124 | 1.50          | 1.45          | 0.05 | B    | 0.3  | A   | 0.7 | B   | Example 125 | 1.50          | 1.46          | 0.04        | A    | 0.3  | A    | 0.7 | B   | Example 126 | 1.50          | 1.43          | 0.07        | B    | 0.5  | B    | 1.1 | C   | Example 127 | 1.50          | 1.41          | 0.09          | B           | 0.5  | B    | 1.0  | C   | Example 128 | 1.50          | 1.41          | 0.09          | B           | 0.6  | B    | 1.2  | C   | Example 129 | 1.50          | 1.41          | 0.09          | B           | 0.7         | B    | 1.4  | C    | Example 130 | 1.50          | 1.40          | 0.10          | C             | 0.7         | B    | 1.4  | C    | Example 131 | 1.50          | 1.42          | 0.08          | B             | 0.6         | B           | 1.2  | C    | Example 132 | 1.50          | 1.45          | 0.05          | B             | 0.3         | A           | 0.7  | B    | Example 133 | 1.50          | 1.43          | 0.07          | B             | 0.9         | B           | 1.4  | C    | Example 134 | 1.50          | 1.43          | 0.07          | B             | 0.5         | B           | 0.8  | B    | Example 135 | 1.50          | 1.42          | 0.08          | B             | 0.7           | B           | 0.9  | B    | Example 136 | 1.50          | 1.38          | 0.12          | C             | 0.9           | B           | 1.3  | C    | 40          | Example 137   | 1.50          | 1.46          | 0.04          | A             | 0.3         | A    | 0.9  | B           | Example 138   | 1.50          | 1.45          | 0.05          | B             | 0.4         | A    | 0.8  | B           | Example 139   | 1.50          | 1.46          | 0.04          | A             | 0.3         | A    | 0.7  | B           | Comparative 1 | 1.50          | 1.33          | 0.17          | D             | 1.4         | C    | 2.5  | D           | Example 101   | 1.50          | 1.46          | 0.04          | A             | 0.4         | A    | 0.8  | B    | 45            | Comparative 1 | 1.50          | 1.42          | 0.08          | B           | 1.2  | C    | 2.2  | D             | Comparative 1 | 1.50          | 1.41          | 0.09          | B           | 0.8  | B    | 1.4  | C             | Comparative 1 | 1.50          | 1.37          | 0.13          | C           | 1.0  | C    | 2.0  | D             | 50            | Comparative 1 | 1.50          | 1.45          | 0.05        | B    | 0.3  | A    | 0.7         | B             | Comparative 1 | 1.50          | 1.32          | 0.18        | D    | 0.7  | B    | 2.5 | D             | Comparative 1 | 1.50          | 1.30          | 0.20        | D    | 1.3  | C    | 2.3 | D             | 55            | Comparative 1 | 1.50          | 1.31        | 0.19 | D    | 2.0  | D   | 3.0           | D             | Comparative 1 | 1.50          | 1.38        | 0.12 | C    | 1.6  | C   | 2.6 | D             | Comparative 1 | 1.50          | 1.35        | 0.15 | D    | 1.8  | C   | 2.4 | D             | 60            | Comparative 1 | 1.50        | 1.33 | 0.17 | D    | 1.5 | C   | 2.6           | D             | Comparative 1 | 1.50        | 1.38 | 0.12 | C    | 1.5 | C   | 3.5 | D             | Comparative 1 | 1.50        | 1.36 | 0.14 | C    | 1.8 | C   | 2.4 | D             | 65            | Example 114 |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 120                                            | 1.50           | 1.45                | 0.05 | B           | 0.3            | A    | 0.7         | B              | Example 121   | 1.50 | 1.41 | 0.09 | B | 0.5 | B | 1.1 | C | Example 122   | 1.50          | 1.43 | 0.07 | B    | 0.4 | A   | 0.9 | B   | Example 123   | 1.50          | 1.41 | 0.09 | B    | 0.8 | B   | 1.2 | C   | Example 124 | 1.50          | 1.45        | 0.05 | B    | 0.3  | A   | 0.7 | B   | Example 125 | 1.50          | 1.46          | 0.04 | A    | 0.3  | A   | 0.7 | B   | Example 126 | 1.50          | 1.43          | 0.07        | B    | 0.5  | B    | 1.1 | C   | Example 127 | 1.50          | 1.41          | 0.09        | B    | 0.5  | B    | 1.0 | C   | Example 128 | 1.50          | 1.41          | 0.09          | B           | 0.6  | B    | 1.2  | C   | Example 129 | 1.50          | 1.41          | 0.09          | B           | 0.7  | B    | 1.4  | C   | Example 130 | 1.50          | 1.40          | 0.10          | C           | 0.7         | B    | 1.4  | C    | Example 131 | 1.50          | 1.42          | 0.08          | B             | 0.6         | B    | 1.2  | C    | Example 132 | 1.50          | 1.45          | 0.05          | B             | 0.3         | A           | 0.7  | B    | Example 133 | 1.50          | 1.43          | 0.07          | B             | 0.9         | B           | 1.4  | C    | Example 134 | 1.50          | 1.43          | 0.07          | B             | 0.5         | B           | 0.8  | B    | Example 135 | 1.50          | 1.42          | 0.08          | B             | 0.7         | B           | 0.9  | B    | Example 136 | 1.50          | 1.38          | 0.12          | C             | 0.9           | B           | 1.3  | C    | 40          | Example 137   | 1.50          | 1.46          | 0.04          | A             | 0.3         | A    | 0.9  | B           | Example 138   | 1.50          | 1.45          | 0.05          | B             | 0.4         | A    | 0.8  | B           | Example 139   | 1.50          | 1.46          | 0.04          | A             | 0.3         | A    | 0.7  | B           | Comparative 1 | 1.50          | 1.33          | 0.17          | D             | 1.4         | C    | 2.5  | D           | Example 101   | 1.50          | 1.46          | 0.04          | A             | 0.4         | A    | 0.8  | B           | 45            | Comparative 1 | 1.50          | 1.42          | 0.08          | B           | 1.2  | C    | 2.2  | D             | Comparative 1 | 1.50          | 1.41          | 0.09          | B           | 0.8  | B    | 1.4  | C             | Comparative 1 | 1.50          | 1.37          | 0.13          | C           | 1.0  | C    | 2.0  | D             | 50            | Comparative 1 | 1.50          | 1.45          | 0.05        | B    | 0.3  | A    | 0.7           | B             | Comparative 1 | 1.50          | 1.32          | 0.18        | D    | 0.7  | B    | 2.5         | D             | Comparative 1 | 1.50          | 1.30          | 0.20        | D    | 1.3  | C    | 2.3 | D             | 55            | Comparative 1 | 1.50          | 1.31        | 0.19 | D    | 2.0  | D   | 3.0           | D             | Comparative 1 | 1.50          | 1.38        | 0.12 | C    | 1.6  | C   | 2.6           | D             | Comparative 1 | 1.50          | 1.35        | 0.15 | D    | 1.8  | C   | 2.4 | D             | 60            | Comparative 1 | 1.50        | 1.33 | 0.17 | D    | 1.5 | C   | 2.6           | D             | Comparative 1 | 1.50        | 1.38 | 0.12 | C    | 1.5 | C   | 3.5           | D             | Comparative 1 | 1.50        | 1.36 | 0.14 | C    | 1.8 | C   | 2.4 | D             | 65            | Example 114 |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 121                                            | 1.50           | 1.41                | 0.09 | B           | 0.5            | B    | 1.1         | C              | Example 122   | 1.50 | 1.43 | 0.07 | B | 0.4 | A | 0.9 | B | Example 123   | 1.50          | 1.41 | 0.09 | B    | 0.8 | B   | 1.2 | C   | Example 124   | 1.50          | 1.45 | 0.05 | B    | 0.3 | A   | 0.7 | B   | Example 125 | 1.50          | 1.46        | 0.04 | A    | 0.3  | A   | 0.7 | B   | Example 126 | 1.50          | 1.43          | 0.07 | B    | 0.5  | B   | 1.1 | C   | Example 127 | 1.50          | 1.41          | 0.09        | B    | 0.5  | B    | 1.0 | C   | Example 128 | 1.50          | 1.41          | 0.09        | B    | 0.6  | B    | 1.2 | C   | Example 129 | 1.50          | 1.41          | 0.09          | B           | 0.7  | B    | 1.4  | C   | Example 130 | 1.50          | 1.40          | 0.10          | C           | 0.7  | B    | 1.4  | C   | Example 131 | 1.50          | 1.42          | 0.08          | B           | 0.6         | B    | 1.2  | C    | Example 132 | 1.50          | 1.45          | 0.05          | B             | 0.3         | A    | 0.7  | B    | Example 133 | 1.50          | 1.43          | 0.07          | B             | 0.9         | B           | 1.4  | C    | Example 134 | 1.50          | 1.43          | 0.07          | B             | 0.5         | B           | 0.8  | B    | Example 135 | 1.50          | 1.42          | 0.08          | B             | 0.7         | B           | 0.9  | B    | Example 136 | 1.50          | 1.38          | 0.12          | C             | 0.9         | B           | 1.3  | C    | 40          | Example 137   | 1.50          | 1.46          | 0.04          | A             | 0.3         | A    | 0.9  | B           | Example 138   | 1.50          | 1.45          | 0.05          | B             | 0.4         | A    | 0.8  | B           | Example 139   | 1.50          | 1.46          | 0.04          | A             | 0.3         | A    | 0.7  | B           | Comparative 1 | 1.50          | 1.33          | 0.17          | D             | 1.4         | C    | 2.5  | D           | Example 101   | 1.50          | 1.46          | 0.04          | A             | 0.4         | A    | 0.8  | B           | 45            | Comparative 1 | 1.50          | 1.42          | 0.08          | B           | 1.2  | C    | 2.2         | D             | Comparative 1 | 1.50          | 1.41          | 0.09          | B           | 0.8  | B    | 1.4  | C             | Comparative 1 | 1.50          | 1.37          | 0.13          | C           | 1.0  | C    | 2.0  | D             | 50            | Comparative 1 | 1.50          | 1.45          | 0.05        | B    | 0.3  | A    | 0.7           | B             | Comparative 1 | 1.50          | 1.32          | 0.18        | D    | 0.7  | B    | 2.5           | D             | Comparative 1 | 1.50          | 1.30          | 0.20        | D    | 1.3  | C    | 2.3         | D             | 55            | Comparative 1 | 1.50          | 1.31        | 0.19 | D    | 2.0  | D   | 3.0           | D             | Comparative 1 | 1.50          | 1.38        | 0.12 | C    | 1.6  | C   | 2.6           | D             | Comparative 1 | 1.50          | 1.35        | 0.15 | D    | 1.8  | C   | 2.4           | D             | 60            | Comparative 1 | 1.50        | 1.33 | 0.17 | D    | 1.5 | C   | 2.6           | D             | Comparative 1 | 1.50        | 1.38 | 0.12 | C    | 1.5 | C   | 3.5           | D             | Comparative 1 | 1.50        | 1.36 | 0.14 | C    | 1.8 | C   | 2.4           | D             | 65            | Example 114 |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 122                                            | 1.50           | 1.43                | 0.07 | B           | 0.4            | A    | 0.9         | B              | Example 123   | 1.50 | 1.41 | 0.09 | B | 0.8 | B | 1.2 | C | Example 124   | 1.50          | 1.45 | 0.05 | B    | 0.3 | A   | 0.7 | B   | Example 125   | 1.50          | 1.46 | 0.04 | A    | 0.3 | A   | 0.7 | B   | Example 126 | 1.50          | 1.43        | 0.07 | B    | 0.5  | B   | 1.1 | C   | Example 127 | 1.50          | 1.41          | 0.09 | B    | 0.5  | B   | 1.0 | C   | Example 128 | 1.50          | 1.41          | 0.09        | B    | 0.6  | B    | 1.2 | C   | Example 129 | 1.50          | 1.41          | 0.09        | B    | 0.7  | B    | 1.4 | C   | Example 130 | 1.50          | 1.40          | 0.10          | C           | 0.7  | B    | 1.4  | C   | Example 131 | 1.50          | 1.42          | 0.08          | B           | 0.6  | B    | 1.2  | C   | Example 132 | 1.50          | 1.45          | 0.05          | B           | 0.3         | A    | 0.7  | B    | Example 133 | 1.50          | 1.43          | 0.07          | B             | 0.9         | B    | 1.4  | C    | Example 134 | 1.50          | 1.43          | 0.07          | B             | 0.5         | B           | 0.8  | B    | Example 135 | 1.50          | 1.42          | 0.08          | B             | 0.7         | B           | 0.9  | B    | Example 136 | 1.50          | 1.38          | 0.12          | C             | 0.9         | B           | 1.3  | C    | 40          | Example 137   | 1.50          | 1.46          | 0.04          | A           | 0.3         | A    | 0.9  | B           | Example 138   | 1.50          | 1.45          | 0.05          | B             | 0.4         | A    | 0.8  | B           | Example 139   | 1.50          | 1.46          | 0.04          | A             | 0.3         | A    | 0.7  | B           | Comparative 1 | 1.50          | 1.33          | 0.17          | D             | 1.4         | C    | 2.5  | D           | Example 101   | 1.50          | 1.46          | 0.04          | A             | 0.4         | A    | 0.8  | B           | 45            | Comparative 1 | 1.50          | 1.42          | 0.08          | B           | 1.2  | C    | 2.2         | D             | Comparative 1 | 1.50          | 1.41          | 0.09          | B           | 0.8  | B    | 1.4         | C             | Comparative 1 | 1.50          | 1.37          | 0.13          | C           | 1.0  | C    | 2.0  | D             | 50            | Comparative 1 | 1.50          | 1.45          | 0.05        | B    | 0.3  | A    | 0.7           | B             | Comparative 1 | 1.50          | 1.32          | 0.18        | D    | 0.7  | B    | 2.5           | D             | Comparative 1 | 1.50          | 1.30          | 0.20        | D    | 1.3  | C    | 2.3           | D             | 55            | Comparative 1 | 1.50          | 1.31        | 0.19 | D    | 2.0  | D           | 3.0           | D             | Comparative 1 | 1.50          | 1.38        | 0.12 | C    | 1.6  | C   | 2.6           | D             | Comparative 1 | 1.50          | 1.35        | 0.15 | D    | 1.8  | C   | 2.4           | D             | 60            | Comparative 1 | 1.50        | 1.33 | 0.17 | D    | 1.5 | C             | 2.6           | D             | Comparative 1 | 1.50        | 1.38 | 0.12 | C    | 1.5 | C   | 3.5           | D             | Comparative 1 | 1.50        | 1.36 | 0.14 | C    | 1.8 | C   | 2.4           | D             | 65            | Example 114 |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 123                                            | 1.50           | 1.41                | 0.09 | B           | 0.8            | B    | 1.2         | C              | Example 124   | 1.50 | 1.45 | 0.05 | B | 0.3 | A | 0.7 | B | Example 125   | 1.50          | 1.46 | 0.04 | A    | 0.3 | A   | 0.7 | B   | Example 126   | 1.50          | 1.43 | 0.07 | B    | 0.5 | B   | 1.1 | C   | Example 127 | 1.50          | 1.41        | 0.09 | B    | 0.5  | B   | 1.0 | C   | Example 128 | 1.50          | 1.41          | 0.09 | B    | 0.6  | B   | 1.2 | C   | Example 129 | 1.50          | 1.41          | 0.09        | B    | 0.7  | B    | 1.4 | C   | Example 130 | 1.50          | 1.40          | 0.10        | C    | 0.7  | B    | 1.4 | C   | Example 131 | 1.50          | 1.42          | 0.08          | B           | 0.6  | B    | 1.2  | C   | Example 132 | 1.50          | 1.45          | 0.05          | B           | 0.3  | A    | 0.7  | B   | Example 133 | 1.50          | 1.43          | 0.07          | B           | 0.9         | B    | 1.4  | C    | Example 134 | 1.50          | 1.43          | 0.07          | B             | 0.5         | B    | 0.8  | B    | Example 135 | 1.50          | 1.42          | 0.08          | B             | 0.7         | B           | 0.9  | B    | Example 136 | 1.50          | 1.38          | 0.12          | C             | 0.9         | B           | 1.3  | C    | 40          | Example 137   | 1.50          | 1.46          | 0.04          | A           | 0.3         | A    | 0.9  | B           | Example 138   | 1.50          | 1.45          | 0.05          | B           | 0.4         | A    | 0.8  | B           | Example 139   | 1.50          | 1.46          | 0.04          | A             | 0.3         | A    | 0.7  | B           | Comparative 1 | 1.50          | 1.33          | 0.17          | D             | 1.4         | C    | 2.5  | D           | Example 101   | 1.50          | 1.46          | 0.04          | A             | 0.4         | A    | 0.8  | B           | 45            | Comparative 1 | 1.50          | 1.42          | 0.08          | B           | 1.2  | C    | 2.2         | D             | Comparative 1 | 1.50          | 1.41          | 0.09          | B           | 0.8  | B    | 1.4         | C             | Comparative 1 | 1.50          | 1.37          | 0.13          | C           | 1.0  | C    | 2.0         | D             | 50            | Comparative 1 | 1.50          | 1.45          | 0.05        | B    | 0.3  | A    | 0.7           | B             | Comparative 1 | 1.50          | 1.32          | 0.18        | D    | 0.7  | B    | 2.5           | D             | Comparative 1 | 1.50          | 1.30          | 0.20        | D    | 1.3  | C    | 2.3           | D             | 55            | Comparative 1 | 1.50          | 1.31        | 0.19 | D    | 2.0  | D             | 3.0           | D             | Comparative 1 | 1.50          | 1.38        | 0.12 | C    | 1.6  | C           | 2.6           | D             | Comparative 1 | 1.50          | 1.35        | 0.15 | D    | 1.8  | C   | 2.4           | D             | 60            | Comparative 1 | 1.50        | 1.33 | 0.17 | D    | 1.5 | C             | 2.6           | D             | Comparative 1 | 1.50        | 1.38 | 0.12 | C    | 1.5 | C             | 3.5           | D             | Comparative 1 | 1.50        | 1.36 | 0.14 | C    | 1.8 | C   | 2.4           | D             | 65            | Example 114 |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 124                                            | 1.50           | 1.45                | 0.05 | B           | 0.3            | A    | 0.7         | B              | Example 125   | 1.50 | 1.46 | 0.04 | A | 0.3 | A | 0.7 | B | Example 126   | 1.50          | 1.43 | 0.07 | B    | 0.5 | B   | 1.1 | C   | Example 127   | 1.50          | 1.41 | 0.09 | B    | 0.5 | B   | 1.0 | C   | Example 128 | 1.50          | 1.41        | 0.09 | B    | 0.6  | B   | 1.2 | C   | Example 129 | 1.50          | 1.41          | 0.09 | B    | 0.7  | B   | 1.4 | C   | Example 130 | 1.50          | 1.40          | 0.10        | C    | 0.7  | B    | 1.4 | C   | Example 131 | 1.50          | 1.42          | 0.08        | B    | 0.6  | B    | 1.2 | C   | Example 132 | 1.50          | 1.45          | 0.05          | B           | 0.3  | A    | 0.7  | B   | Example 133 | 1.50          | 1.43          | 0.07          | B           | 0.9  | B    | 1.4  | C   | Example 134 | 1.50          | 1.43          | 0.07          | B           | 0.5         | B    | 0.8  | B    | Example 135 | 1.50          | 1.42          | 0.08          | B             | 0.7         | B    | 0.9  | B    | Example 136 | 1.50          | 1.38          | 0.12          | C             | 0.9         | B           | 1.3  | C    | 40          | Example 137   | 1.50          | 1.46          | 0.04          | A           | 0.3         | A    | 0.9  | B           | Example 138   | 1.50          | 1.45          | 0.05          | B           | 0.4         | A    | 0.8  | B           | Example 139   | 1.50          | 1.46          | 0.04          | A           | 0.3         | A    | 0.7  | B           | Comparative 1 | 1.50          | 1.33          | 0.17          | D             | 1.4         | C    | 2.5  | D           | Example 101   | 1.50          | 1.46          | 0.04          | A             | 0.4         | A    | 0.8  | B           | 45            | Comparative 1 | 1.50          | 1.42          | 0.08          | B           | 1.2  | C    | 2.2         | D             | Comparative 1 | 1.50          | 1.41          | 0.09          | B           | 0.8  | B    | 1.4         | C             | Comparative 1 | 1.50          | 1.37          | 0.13          | C           | 1.0  | C    | 2.0         | D             | 50            | Comparative 1 | 1.50          | 1.45          | 0.05        | B    | 0.3  | A           | 0.7           | B             | Comparative 1 | 1.50          | 1.32          | 0.18        | D    | 0.7  | B    | 2.5           | D             | Comparative 1 | 1.50          | 1.30          | 0.20        | D    | 1.3  | C    | 2.3           | D             | 55            | Comparative 1 | 1.50          | 1.31        | 0.19 | D    | 2.0  | D             | 3.0           | D             | Comparative 1 | 1.50          | 1.38        | 0.12 | C    | 1.6  | C             | 2.6           | D             | Comparative 1 | 1.50          | 1.35        | 0.15 | D    | 1.8  | C           | 2.4           | D             | 60            | Comparative 1 | 1.50        | 1.33 | 0.17 | D    | 1.5 | C             | 2.6           | D             | Comparative 1 | 1.50        | 1.38 | 0.12 | C    | 1.5 | C             | 3.5           | D             | Comparative 1 | 1.50        | 1.36 | 0.14 | C    | 1.8 | C             | 2.4           | D             | 65            | Example 114 |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 125                                            | 1.50           | 1.46                | 0.04 | A           | 0.3            | A    | 0.7         | B              | Example 126   | 1.50 | 1.43 | 0.07 | B | 0.5 | B | 1.1 | C | Example 127   | 1.50          | 1.41 | 0.09 | B    | 0.5 | B   | 1.0 | C   | Example 128   | 1.50          | 1.41 | 0.09 | B    | 0.6 | B   | 1.2 | C   | Example 129 | 1.50          | 1.41        | 0.09 | B    | 0.7  | B   | 1.4 | C   | Example 130 | 1.50          | 1.40          | 0.10 | C    | 0.7  | B   | 1.4 | C   | Example 131 | 1.50          | 1.42          | 0.08        | B    | 0.6  | B    | 1.2 | C   | Example 132 | 1.50          | 1.45          | 0.05        | B    | 0.3  | A    | 0.7 | B   | Example 133 | 1.50          | 1.43          | 0.07          | B           | 0.9  | B    | 1.4  | C   | Example 134 | 1.50          | 1.43          | 0.07          | B           | 0.5  | B    | 0.8  | B   | Example 135 | 1.50          | 1.42          | 0.08          | B           | 0.7         | B    | 0.9  | B    | Example 136 | 1.50          | 1.38          | 0.12          | C             | 0.9         | B    | 1.3  | C    | 40          | Example 137   | 1.50          | 1.46          | 0.04          | A           | 0.3         | A    | 0.9  | B           | Example 138   | 1.50          | 1.45          | 0.05          | B           | 0.4         | A    | 0.8  | B           | Example 139   | 1.50          | 1.46          | 0.04          | A           | 0.3         | A    | 0.7  | B           | Comparative 1 | 1.50          | 1.33          | 0.17          | D           | 1.4         | C    | 2.5  | D           | Example 101   | 1.50          | 1.46          | 0.04          | A             | 0.4         | A    | 0.8  | B           | 45            | Comparative 1 | 1.50          | 1.42          | 0.08          | B           | 1.2  | C    | 2.2         | D             | Comparative 1 | 1.50          | 1.41          | 0.09          | B           | 0.8  | B    | 1.4         | C             | Comparative 1 | 1.50          | 1.37          | 0.13          | C           | 1.0  | C    | 2.0         | D             | 50            | Comparative 1 | 1.50          | 1.45          | 0.05        | B    | 0.3  | A           | 0.7           | B             | Comparative 1 | 1.50          | 1.32          | 0.18        | D    | 0.7  | B           | 2.5           | D             | Comparative 1 | 1.50          | 1.30          | 0.20        | D    | 1.3  | C    | 2.3           | D             | 55            | Comparative 1 | 1.50          | 1.31        | 0.19 | D    | 2.0  | D             | 3.0           | D             | Comparative 1 | 1.50          | 1.38        | 0.12 | C    | 1.6  | C             | 2.6           | D             | Comparative 1 | 1.50          | 1.35        | 0.15 | D    | 1.8  | C             | 2.4           | D             | 60            | Comparative 1 | 1.50        | 1.33 | 0.17 | D    | 1.5         | C             | 2.6           | D             | Comparative 1 | 1.50        | 1.38 | 0.12 | C    | 1.5 | C             | 3.5           | D             | Comparative 1 | 1.50        | 1.36 | 0.14 | C    | 1.8 | C             | 2.4           | D             | 65            | Example 114 |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 126                                            | 1.50           | 1.43                | 0.07 | B           | 0.5            | B    | 1.1         | C              | Example 127   | 1.50 | 1.41 | 0.09 | B | 0.5 | B | 1.0 | C | Example 128   | 1.50          | 1.41 | 0.09 | B    | 0.6 | B   | 1.2 | C   | Example 129   | 1.50          | 1.41 | 0.09 | B    | 0.7 | B   | 1.4 | C   | Example 130 | 1.50          | 1.40        | 0.10 | C    | 0.7  | B   | 1.4 | C   | Example 131 | 1.50          | 1.42          | 0.08 | B    | 0.6  | B   | 1.2 | C   | Example 132 | 1.50          | 1.45          | 0.05        | B    | 0.3  | A    | 0.7 | B   | Example 133 | 1.50          | 1.43          | 0.07        | B    | 0.9  | B    | 1.4 | C   | Example 134 | 1.50          | 1.43          | 0.07          | B           | 0.5  | B    | 0.8  | B   | Example 135 | 1.50          | 1.42          | 0.08          | B           | 0.7  | B    | 0.9  | B   | Example 136 | 1.50          | 1.38          | 0.12          | C           | 0.9         | B    | 1.3  | C    | 40          | Example 137   | 1.50          | 1.46          | 0.04          | A           | 0.3  | A    | 0.9  | B           | Example 138   | 1.50          | 1.45          | 0.05          | B           | 0.4         | A    | 0.8  | B           | Example 139   | 1.50          | 1.46          | 0.04          | A           | 0.3         | A    | 0.7  | B           | Comparative 1 | 1.50          | 1.33          | 0.17          | D           | 1.4         | C    | 2.5  | D           | Example 101   | 1.50          | 1.46          | 0.04          | A           | 0.4         | A    | 0.8  | B           | 45            | Comparative 1 | 1.50          | 1.42          | 0.08          | B           | 1.2  | C    | 2.2         | D             | Comparative 1 | 1.50          | 1.41          | 0.09          | B           | 0.8  | B    | 1.4         | C             | Comparative 1 | 1.50          | 1.37          | 0.13          | C           | 1.0  | C    | 2.0         | D             | 50            | Comparative 1 | 1.50          | 1.45          | 0.05        | B    | 0.3  | A           | 0.7           | B             | Comparative 1 | 1.50          | 1.32          | 0.18        | D    | 0.7  | B           | 2.5           | D             | Comparative 1 | 1.50          | 1.30          | 0.20        | D    | 1.3  | C           | 2.3           | D             | 55            | Comparative 1 | 1.50          | 1.31        | 0.19 | D    | 2.0  | D             | 3.0           | D             | Comparative 1 | 1.50          | 1.38        | 0.12 | C    | 1.6  | C             | 2.6           | D             | Comparative 1 | 1.50          | 1.35        | 0.15 | D    | 1.8  | C             | 2.4           | D             | 60            | Comparative 1 | 1.50        | 1.33 | 0.17 | D    | 1.5           | C             | 2.6           | D             | Comparative 1 | 1.50        | 1.38 | 0.12 | C    | 1.5         | C             | 3.5           | D             | Comparative 1 | 1.50        | 1.36 | 0.14 | C    | 1.8 | C             | 2.4           | D             | 65            | Example 114 |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 127                                            | 1.50           | 1.41                | 0.09 | B           | 0.5            | B    | 1.0         | C              | Example 128   | 1.50 | 1.41 | 0.09 | B | 0.6 | B | 1.2 | C | Example 129   | 1.50          | 1.41 | 0.09 | B    | 0.7 | B   | 1.4 | C   | Example 130   | 1.50          | 1.40 | 0.10 | C    | 0.7 | B   | 1.4 | C   | Example 131 | 1.50          | 1.42        | 0.08 | B    | 0.6  | B   | 1.2 | C   | Example 132 | 1.50          | 1.45          | 0.05 | B    | 0.3  | A   | 0.7 | B   | Example 133 | 1.50          | 1.43          | 0.07        | B    | 0.9  | B    | 1.4 | C   | Example 134 | 1.50          | 1.43          | 0.07        | B    | 0.5  | B    | 0.8 | B   | Example 135 | 1.50          | 1.42          | 0.08          | B           | 0.7  | B    | 0.9  | B   | Example 136 | 1.50          | 1.38          | 0.12          | C           | 0.9  | B    | 1.3  | C   | 40          | Example 137   | 1.50          | 1.46          | 0.04        | A           | 0.3  | A    | 0.9  | B           | Example 138   | 1.50          | 1.45          | 0.05          | B           | 0.4  | A    | 0.8  | B           | Example 139   | 1.50          | 1.46          | 0.04          | A           | 0.3         | A    | 0.7  | B           | Comparative 1 | 1.50          | 1.33          | 0.17          | D           | 1.4         | C    | 2.5  | D           | Example 101   | 1.50          | 1.46          | 0.04          | A           | 0.4         | A    | 0.8  | B           | 45            | Comparative 1 | 1.50          | 1.42          | 0.08        | B           | 1.2  | C    | 2.2         | D             | Comparative 1 | 1.50          | 1.41          | 0.09          | B           | 0.8  | B    | 1.4         | C             | Comparative 1 | 1.50          | 1.37          | 0.13          | C           | 1.0  | C    | 2.0         | D             | 50            | Comparative 1 | 1.50          | 1.45          | 0.05        | B    | 0.3  | A           | 0.7           | B             | Comparative 1 | 1.50          | 1.32          | 0.18        | D    | 0.7  | B           | 2.5           | D             | Comparative 1 | 1.50          | 1.30          | 0.20        | D    | 1.3  | C           | 2.3           | D             | 55            | Comparative 1 | 1.50          | 1.31        | 0.19 | D    | 2.0         | D             | 3.0           | D             | Comparative 1 | 1.50          | 1.38        | 0.12 | C    | 1.6  | C             | 2.6           | D             | Comparative 1 | 1.50          | 1.35        | 0.15 | D    | 1.8  | C             | 2.4           | D             | 60            | Comparative 1 | 1.50        | 1.33 | 0.17 | D    | 1.5           | C             | 2.6           | D             | Comparative 1 | 1.50        | 1.38 | 0.12 | C    | 1.5           | C             | 3.5           | D             | Comparative 1 | 1.50        | 1.36 | 0.14 | C    | 1.8         | C             | 2.4           | D             | 65            | Example 114 |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 128                                            | 1.50           | 1.41                | 0.09 | B           | 0.6            | B    | 1.2         | C              | Example 129   | 1.50 | 1.41 | 0.09 | B | 0.7 | B | 1.4 | C | Example 130   | 1.50          | 1.40 | 0.10 | C    | 0.7 | B   | 1.4 | C   | Example 131   | 1.50          | 1.42 | 0.08 | B    | 0.6 | B   | 1.2 | C   | Example 132 | 1.50          | 1.45        | 0.05 | B    | 0.3  | A   | 0.7 | B   | Example 133 | 1.50          | 1.43          | 0.07 | B    | 0.9  | B   | 1.4 | C   | Example 134 | 1.50          | 1.43          | 0.07        | B    | 0.5  | B    | 0.8 | B   | Example 135 | 1.50          | 1.42          | 0.08        | B    | 0.7  | B    | 0.9 | B   | Example 136 | 1.50          | 1.38          | 0.12          | C           | 0.9  | B    | 1.3  | C   | 40          | Example 137   | 1.50          | 1.46          | 0.04        | A    | 0.3  | A    | 0.9 | B           | Example 138   | 1.50          | 1.45          | 0.05        | B           | 0.4  | A    | 0.8  | B           | Example 139   | 1.50          | 1.46          | 0.04          | A           | 0.3  | A    | 0.7  | B           | Comparative 1 | 1.50          | 1.33          | 0.17          | D           | 1.4         | C    | 2.5  | D           | Example 101   | 1.50          | 1.46          | 0.04          | A           | 0.4         | A    | 0.8  | B           | 45            | Comparative 1 | 1.50          | 1.42          | 0.08        | B           | 1.2  | C    | 2.2         | D             | Comparative 1 | 1.50          | 1.41          | 0.09        | B           | 0.8  | B    | 1.4         | C             | Comparative 1 | 1.50          | 1.37          | 0.13          | C           | 1.0  | C    | 2.0         | D             | 50            | Comparative 1 | 1.50          | 1.45          | 0.05        | B    | 0.3  | A           | 0.7           | B             | Comparative 1 | 1.50          | 1.32          | 0.18        | D    | 0.7  | B           | 2.5           | D             | Comparative 1 | 1.50          | 1.30          | 0.20        | D    | 1.3  | C           | 2.3           | D             | 55            | Comparative 1 | 1.50          | 1.31        | 0.19 | D    | 2.0         | D             | 3.0           | D             | Comparative 1 | 1.50          | 1.38        | 0.12 | C    | 1.6         | C             | 2.6           | D             | Comparative 1 | 1.50          | 1.35        | 0.15 | D    | 1.8  | C             | 2.4           | D             | 60            | Comparative 1 | 1.50        | 1.33 | 0.17 | D    | 1.5           | C             | 2.6           | D             | Comparative 1 | 1.50        | 1.38 | 0.12 | C    | 1.5           | C             | 3.5           | D             | Comparative 1 | 1.50        | 1.36 | 0.14 | C    | 1.8           | C             | 2.4           | D             | 65            | Example 114 |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 129                                            | 1.50           | 1.41                | 0.09 | B           | 0.7            | B    | 1.4         | C              | Example 130   | 1.50 | 1.40 | 0.10 | C | 0.7 | B | 1.4 | C | Example 131   | 1.50          | 1.42 | 0.08 | B    | 0.6 | B   | 1.2 | C   | Example 132   | 1.50          | 1.45 | 0.05 | B    | 0.3 | A   | 0.7 | B   | Example 133 | 1.50          | 1.43        | 0.07 | B    | 0.9  | B   | 1.4 | C   | Example 134 | 1.50          | 1.43          | 0.07 | B    | 0.5  | B   | 0.8 | B   | Example 135 | 1.50          | 1.42          | 0.08        | B    | 0.7  | B    | 0.9 | B   | Example 136 | 1.50          | 1.38          | 0.12        | C    | 0.9  | B    | 1.3 | C   | 40          | Example 137   | 1.50          | 1.46          | 0.04        | A    | 0.3  | A    | 0.9 | B           | Example 138   | 1.50          | 1.45          | 0.05        | B    | 0.4  | A    | 0.8 | B           | Example 139   | 1.50          | 1.46          | 0.04        | A           | 0.3  | A    | 0.7  | B           | Comparative 1 | 1.50          | 1.33          | 0.17          | D           | 1.4  | C    | 2.5  | D           | Example 101   | 1.50          | 1.46          | 0.04          | A           | 0.4         | A    | 0.8  | B           | 45            | Comparative 1 | 1.50          | 1.42          | 0.08        | B           | 1.2  | C    | 2.2         | D             | Comparative 1 | 1.50          | 1.41          | 0.09        | B           | 0.8  | B    | 1.4         | C             | Comparative 1 | 1.50          | 1.37          | 0.13        | C           | 1.0  | C    | 2.0         | D             | 50            | Comparative 1 | 1.50          | 1.45          | 0.05        | B    | 0.3  | A           | 0.7           | B             | Comparative 1 | 1.50          | 1.32          | 0.18        | D    | 0.7  | B           | 2.5           | D             | Comparative 1 | 1.50          | 1.30          | 0.20        | D    | 1.3  | C           | 2.3           | D             | 55            | Comparative 1 | 1.50          | 1.31        | 0.19 | D    | 2.0         | D             | 3.0           | D             | Comparative 1 | 1.50          | 1.38        | 0.12 | C    | 1.6         | C             | 2.6           | D             | Comparative 1 | 1.50          | 1.35        | 0.15 | D    | 1.8         | C             | 2.4           | D             | 60            | Comparative 1 | 1.50        | 1.33 | 0.17 | D    | 1.5           | C             | 2.6           | D             | Comparative 1 | 1.50        | 1.38 | 0.12 | C    | 1.5           | C             | 3.5           | D             | Comparative 1 | 1.50        | 1.36 | 0.14 | C    | 1.8           | C             | 2.4           | D             | 65            | Example 114 |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 130                                            | 1.50           | 1.40                | 0.10 | C           | 0.7            | B    | 1.4         | C              | Example 131   | 1.50 | 1.42 | 0.08 | B | 0.6 | B | 1.2 | C | Example 132   | 1.50          | 1.45 | 0.05 | B    | 0.3 | A   | 0.7 | B   | Example 133   | 1.50          | 1.43 | 0.07 | B    | 0.9 | B   | 1.4 | C   | Example 134 | 1.50          | 1.43        | 0.07 | B    | 0.5  | B   | 0.8 | B   | Example 135 | 1.50          | 1.42          | 0.08 | B    | 0.7  | B   | 0.9 | B   | Example 136 | 1.50          | 1.38          | 0.12        | C    | 0.9  | B    | 1.3 | C   | 40          | Example 137   | 1.50          | 1.46        | 0.04 | A    | 0.3  | A   | 0.9 | B           | Example 138   | 1.50          | 1.45          | 0.05        | B    | 0.4  | A    | 0.8 | B           | Example 139   | 1.50          | 1.46          | 0.04        | A    | 0.3  | A    | 0.7 | B           | Comparative 1 | 1.50          | 1.33          | 0.17        | D           | 1.4  | C    | 2.5  | D           | Example 101   | 1.50          | 1.46          | 0.04          | A           | 0.4  | A    | 0.8  | B           | 45            | Comparative 1 | 1.50          | 1.42          | 0.08        | B           | 1.2  | C    | 2.2         | D             | Comparative 1 | 1.50          | 1.41          | 0.09        | B           | 0.8  | B    | 1.4         | C             | Comparative 1 | 1.50          | 1.37          | 0.13        | C           | 1.0  | C    | 2.0         | D             | 50            | Comparative 1 | 1.50          | 1.45        | 0.05        | B    | 0.3  | A           | 0.7           | B             | Comparative 1 | 1.50          | 1.32          | 0.18        | D    | 0.7  | B           | 2.5           | D             | Comparative 1 | 1.50          | 1.30          | 0.20        | D    | 1.3  | C           | 2.3           | D             | 55            | Comparative 1 | 1.50          | 1.31        | 0.19 | D    | 2.0         | D             | 3.0           | D             | Comparative 1 | 1.50          | 1.38        | 0.12 | C    | 1.6         | C             | 2.6           | D             | Comparative 1 | 1.50          | 1.35        | 0.15 | D    | 1.8         | C             | 2.4           | D             | 60            | Comparative 1 | 1.50        | 1.33 | 0.17 | D           | 1.5           | C             | 2.6           | D             | Comparative 1 | 1.50        | 1.38 | 0.12 | C    | 1.5           | C             | 3.5           | D             | Comparative 1 | 1.50        | 1.36 | 0.14 | C    | 1.8           | C             | 2.4           | D             | 65            | Example 114 |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 131                                            | 1.50           | 1.42                | 0.08 | B           | 0.6            | B    | 1.2         | C              | Example 132   | 1.50 | 1.45 | 0.05 | B | 0.3 | A | 0.7 | B | Example 133   | 1.50          | 1.43 | 0.07 | B    | 0.9 | B   | 1.4 | C   | Example 134   | 1.50          | 1.43 | 0.07 | B    | 0.5 | B   | 0.8 | B   | Example 135 | 1.50          | 1.42        | 0.08 | B    | 0.7  | B   | 0.9 | B   | Example 136 | 1.50          | 1.38          | 0.12 | C    | 0.9  | B   | 1.3 | C   | 40          | Example 137   | 1.50          | 1.46        | 0.04 | A    | 0.3  | A   | 0.9 | B           | Example 138   | 1.50          | 1.45        | 0.05 | B    | 0.4  | A   | 0.8 | B           | Example 139   | 1.50          | 1.46          | 0.04        | A    | 0.3  | A    | 0.7 | B           | Comparative 1 | 1.50          | 1.33          | 0.17        | D    | 1.4  | C    | 2.5 | D           | Example 101   | 1.50          | 1.46          | 0.04        | A           | 0.4  | A    | 0.8  | B           | 45            | Comparative 1 | 1.50          | 1.42          | 0.08        | B    | 1.2  | C    | 2.2         | D             | Comparative 1 | 1.50          | 1.41          | 0.09        | B           | 0.8  | B    | 1.4         | C             | Comparative 1 | 1.50          | 1.37          | 0.13        | C           | 1.0  | C    | 2.0         | D             | 50            | Comparative 1 | 1.50          | 1.45        | 0.05        | B    | 0.3  | A           | 0.7           | B             | Comparative 1 | 1.50          | 1.32        | 0.18        | D    | 0.7  | B           | 2.5           | D             | Comparative 1 | 1.50          | 1.30          | 0.20        | D    | 1.3  | C           | 2.3           | D             | 55            | Comparative 1 | 1.50          | 1.31        | 0.19 | D    | 2.0         | D             | 3.0           | D             | Comparative 1 | 1.50          | 1.38        | 0.12 | C    | 1.6         | C             | 2.6           | D             | Comparative 1 | 1.50          | 1.35        | 0.15 | D    | 1.8         | C             | 2.4           | D             | 60            | Comparative 1 | 1.50        | 1.33 | 0.17 | D           | 1.5           | C             | 2.6           | D             | Comparative 1 | 1.50        | 1.38 | 0.12 | C           | 1.5           | C             | 3.5           | D             | Comparative 1 | 1.50        | 1.36 | 0.14 | C    | 1.8           | C             | 2.4           | D             | 65            | Example 114 |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 132                                            | 1.50           | 1.45                | 0.05 | B           | 0.3            | A    | 0.7         | B              | Example 133   | 1.50 | 1.43 | 0.07 | B | 0.9 | B | 1.4 | C | Example 134   | 1.50          | 1.43 | 0.07 | B    | 0.5 | B   | 0.8 | B   | Example 135   | 1.50          | 1.42 | 0.08 | B    | 0.7 | B   | 0.9 | B   | Example 136 | 1.50          | 1.38        | 0.12 | C    | 0.9  | B   | 1.3 | C   | 40          | Example 137   | 1.50          | 1.46 | 0.04 | A    | 0.3 | A   | 0.9 | B           | Example 138   | 1.50          | 1.45        | 0.05 | B    | 0.4  | A   | 0.8 | B           | Example 139   | 1.50          | 1.46        | 0.04 | A    | 0.3  | A   | 0.7 | B           | Comparative 1 | 1.50          | 1.33          | 0.17        | D    | 1.4  | C    | 2.5 | D           | Example 101   | 1.50          | 1.46          | 0.04        | A    | 0.4  | A    | 0.8 | B           | 45            | Comparative 1 | 1.50          | 1.42        | 0.08        | B    | 1.2  | C    | 2.2         | D             | Comparative 1 | 1.50          | 1.41          | 0.09        | B    | 0.8  | B    | 1.4         | C             | Comparative 1 | 1.50          | 1.37          | 0.13        | C           | 1.0  | C    | 2.0         | D             | 50            | Comparative 1 | 1.50          | 1.45        | 0.05        | B    | 0.3  | A           | 0.7           | B             | Comparative 1 | 1.50          | 1.32        | 0.18        | D    | 0.7  | B           | 2.5           | D             | Comparative 1 | 1.50          | 1.30        | 0.20        | D    | 1.3  | C           | 2.3           | D             | 55            | Comparative 1 | 1.50          | 1.31        | 0.19 | D    | 2.0         | D             | 3.0           | D             | Comparative 1 | 1.50          | 1.38        | 0.12 | C    | 1.6         | C             | 2.6           | D             | Comparative 1 | 1.50          | 1.35        | 0.15 | D    | 1.8         | C             | 2.4           | D             | 60            | Comparative 1 | 1.50        | 1.33 | 0.17 | D           | 1.5           | C             | 2.6           | D             | Comparative 1 | 1.50        | 1.38 | 0.12 | C           | 1.5           | C             | 3.5           | D             | Comparative 1 | 1.50        | 1.36 | 0.14 | C           | 1.8           | C             | 2.4           | D             | 65            | Example 114 |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 133                                            | 1.50           | 1.43                | 0.07 | B           | 0.9            | B    | 1.4         | C              | Example 134   | 1.50 | 1.43 | 0.07 | B | 0.5 | B | 0.8 | B | Example 135   | 1.50          | 1.42 | 0.08 | B    | 0.7 | B   | 0.9 | B   | Example 136   | 1.50          | 1.38 | 0.12 | C    | 0.9 | B   | 1.3 | C   | 40          | Example 137   | 1.50        | 1.46 | 0.04 | A    | 0.3 | A   | 0.9 | B           | Example 138   | 1.50          | 1.45 | 0.05 | B    | 0.4 | A   | 0.8 | B           | Example 139   | 1.50          | 1.46        | 0.04 | A    | 0.3  | A   | 0.7 | B           | Comparative 1 | 1.50          | 1.33        | 0.17 | D    | 1.4  | C   | 2.5 | D           | Example 101   | 1.50          | 1.46          | 0.04        | A    | 0.4  | A    | 0.8 | B           | 45            | Comparative 1 | 1.50          | 1.42        | 0.08 | B    | 1.2  | C   | 2.2         | D             | Comparative 1 | 1.50          | 1.41        | 0.09        | B    | 0.8  | B    | 1.4         | C             | Comparative 1 | 1.50          | 1.37          | 0.13        | C    | 1.0  | C    | 2.0         | D             | 50            | Comparative 1 | 1.50          | 1.45        | 0.05        | B    | 0.3  | A           | 0.7           | B             | Comparative 1 | 1.50          | 1.32        | 0.18        | D    | 0.7  | B           | 2.5           | D             | Comparative 1 | 1.50          | 1.30        | 0.20        | D    | 1.3  | C           | 2.3           | D             | 55            | Comparative 1 | 1.50        | 1.31        | 0.19 | D    | 2.0         | D             | 3.0           | D             | Comparative 1 | 1.50          | 1.38        | 0.12 | C    | 1.6         | C             | 2.6           | D             | Comparative 1 | 1.50          | 1.35        | 0.15 | D    | 1.8         | C             | 2.4           | D             | 60            | Comparative 1 | 1.50        | 1.33 | 0.17 | D           | 1.5           | C             | 2.6           | D             | Comparative 1 | 1.50        | 1.38 | 0.12 | C           | 1.5           | C             | 3.5           | D             | Comparative 1 | 1.50        | 1.36 | 0.14 | C           | 1.8           | C             | 2.4           | D             | 65            | Example 114 |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 134                                            | 1.50           | 1.43                | 0.07 | B           | 0.5            | B    | 0.8         | B              | Example 135   | 1.50 | 1.42 | 0.08 | B | 0.7 | B | 0.9 | B | Example 136   | 1.50          | 1.38 | 0.12 | C    | 0.9 | B   | 1.3 | C   | 40            | Example 137   | 1.50 | 1.46 | 0.04 | A   | 0.3 | A   | 0.9 | B           | Example 138   | 1.50        | 1.45 | 0.05 | B    | 0.4 | A   | 0.8 | B           | Example 139   | 1.50          | 1.46 | 0.04 | A    | 0.3 | A   | 0.7 | B           | Comparative 1 | 1.50          | 1.33        | 0.17 | D    | 1.4  | C   | 2.5 | D           | Example 101   | 1.50          | 1.46        | 0.04 | A    | 0.4  | A   | 0.8 | B           | 45            | Comparative 1 | 1.50          | 1.42        | 0.08 | B    | 1.2  | C   | 2.2         | D             | Comparative 1 | 1.50          | 1.41        | 0.09 | B    | 0.8  | B   | 1.4         | C             | Comparative 1 | 1.50          | 1.37        | 0.13        | C    | 1.0  | C    | 2.0         | D             | 50            | Comparative 1 | 1.50          | 1.45        | 0.05 | B    | 0.3  | A           | 0.7           | B             | Comparative 1 | 1.50          | 1.32        | 0.18        | D    | 0.7  | B           | 2.5           | D             | Comparative 1 | 1.50          | 1.30        | 0.20        | D    | 1.3  | C           | 2.3           | D             | 55            | Comparative 1 | 1.50        | 1.31        | 0.19 | D    | 2.0         | D             | 3.0           | D             | Comparative 1 | 1.50        | 1.38        | 0.12 | C    | 1.6         | C             | 2.6           | D             | Comparative 1 | 1.50          | 1.35        | 0.15 | D    | 1.8         | C             | 2.4           | D             | 60            | Comparative 1 | 1.50        | 1.33 | 0.17 | D           | 1.5           | C             | 2.6           | D             | Comparative 1 | 1.50        | 1.38 | 0.12 | C           | 1.5           | C             | 3.5           | D             | Comparative 1 | 1.50        | 1.36 | 0.14 | C           | 1.8           | C             | 2.4           | D             | 65            | Example 114 |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 135                                            | 1.50           | 1.42                | 0.08 | B           | 0.7            | B    | 0.9         | B              | Example 136   | 1.50 | 1.38 | 0.12 | C | 0.9 | B | 1.3 | C | 40            | Example 137   | 1.50 | 1.46 | 0.04 | A   | 0.3 | A   | 0.9 | B             | Example 138   | 1.50 | 1.45 | 0.05 | B   | 0.4 | A   | 0.8 | B           | Example 139   | 1.50        | 1.46 | 0.04 | A    | 0.3 | A   | 0.7 | B           | Comparative 1 | 1.50          | 1.33 | 0.17 | D    | 1.4 | C   | 2.5 | D           | Example 101   | 1.50          | 1.46        | 0.04 | A    | 0.4  | A   | 0.8 | B           | 45            | Comparative 1 | 1.50        | 1.42 | 0.08 | B    | 1.2 | C   | 2.2         | D             | Comparative 1 | 1.50          | 1.41        | 0.09 | B    | 0.8  | B   | 1.4         | C             | Comparative 1 | 1.50          | 1.37        | 0.13 | C    | 1.0  | C   | 2.0         | D             | 50            | Comparative 1 | 1.50        | 1.45        | 0.05 | B    | 0.3  | A           | 0.7           | B             | Comparative 1 | 1.50          | 1.32        | 0.18 | D    | 0.7  | B           | 2.5           | D             | Comparative 1 | 1.50          | 1.30        | 0.20        | D    | 1.3  | C           | 2.3           | D             | 55            | Comparative 1 | 1.50        | 1.31        | 0.19 | D    | 2.0         | D             | 3.0           | D             | Comparative 1 | 1.50        | 1.38        | 0.12 | C    | 1.6         | C             | 2.6           | D             | Comparative 1 | 1.50        | 1.35        | 0.15 | D    | 1.8         | C             | 2.4           | D             | 60            | Comparative 1 | 1.50        | 1.33 | 0.17 | D           | 1.5           | C             | 2.6           | D             | Comparative 1 | 1.50        | 1.38 | 0.12 | C           | 1.5           | C             | 3.5           | D             | Comparative 1 | 1.50        | 1.36 | 0.14 | C           | 1.8           | C             | 2.4           | D             | 65            | Example 114 |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 136                                            | 1.50           | 1.38                | 0.12 | C           | 0.9            | B    | 1.3         | C              | 40            |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 137                                            | 1.50           | 1.46                | 0.04 | A           | 0.3            | A    | 0.9         | B              | Example 138   | 1.50 | 1.45 | 0.05 | B | 0.4 | A | 0.8 | B | Example 139   | 1.50          | 1.46 | 0.04 | A    | 0.3 | A   | 0.7 | B   | Comparative 1 | 1.50          | 1.33 | 0.17 | D    | 1.4 | C   | 2.5 | D   | Example 101 | 1.50          | 1.46        | 0.04 | A    | 0.4  | A   | 0.8 | B   | 45          | Comparative 1 | 1.50          | 1.42 | 0.08 | B    | 1.2 | C   | 2.2 | D           | Comparative 1 | 1.50          | 1.41        | 0.09 | B    | 0.8  | B   | 1.4 | C           | Comparative 1 | 1.50          | 1.37        | 0.13 | C    | 1.0  | C   | 2.0 | D           | 50            | Comparative 1 | 1.50          | 1.45        | 0.05 | B    | 0.3  | A   | 0.7         | B             | Comparative 1 | 1.50          | 1.32        | 0.18 | D    | 0.7  | B   | 2.5         | D             | Comparative 1 | 1.50          | 1.30        | 0.20        | D    | 1.3  | C    | 2.3         | D             | 55            | Comparative 1 | 1.50          | 1.31        | 0.19 | D    | 2.0  | D           | 3.0           | D             | Comparative 1 | 1.50          | 1.38        | 0.12        | C    | 1.6  | C           | 2.6           | D             | Comparative 1 | 1.50          | 1.35        | 0.15        | D    | 1.8  | C           | 2.4           | D             | 60            | Comparative 1 | 1.50        | 1.33        | 0.17 | D    | 1.5         | C             | 2.6           | D             | Comparative 1 | 1.50        | 1.38        | 0.12 | C    | 1.5         | C             | 3.5           | D             | Comparative 1 | 1.50          | 1.36        | 0.14 | C    | 1.8         | C             | 2.4           | D             | 65            | Example 114   |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 138                                            | 1.50           | 1.45                | 0.05 | B           | 0.4            | A    | 0.8         | B              | Example 139   | 1.50 | 1.46 | 0.04 | A | 0.3 | A | 0.7 | B | Comparative 1 | 1.50          | 1.33 | 0.17 | D    | 1.4 | C   | 2.5 | D   | Example 101   | 1.50          | 1.46 | 0.04 | A    | 0.4 | A   | 0.8 | B   | 45          | Comparative 1 | 1.50        | 1.42 | 0.08 | B    | 1.2 | C   | 2.2 | D           | Comparative 1 | 1.50          | 1.41 | 0.09 | B    | 0.8 | B   | 1.4 | C           | Comparative 1 | 1.50          | 1.37        | 0.13 | C    | 1.0  | C   | 2.0 | D           | 50            | Comparative 1 | 1.50        | 1.45 | 0.05 | B    | 0.3 | A   | 0.7         | B             | Comparative 1 | 1.50          | 1.32        | 0.18 | D    | 0.7  | B   | 2.5         | D             | Comparative 1 | 1.50          | 1.30        | 0.20 | D    | 1.3  | C   | 2.3         | D             | 55            | Comparative 1 | 1.50        | 1.31        | 0.19 | D    | 2.0  | D           | 3.0           | D             | Comparative 1 | 1.50          | 1.38        | 0.12 | C    | 1.6  | C           | 2.6           | D             | Comparative 1 | 1.50          | 1.35        | 0.15        | D    | 1.8  | C           | 2.4           | D             | 60            | Comparative 1 | 1.50        | 1.33        | 0.17 | D    | 1.5         | C             | 2.6           | D             | Comparative 1 | 1.50        | 1.38        | 0.12 | C    | 1.5         | C             | 3.5           | D             | Comparative 1 | 1.50        | 1.36        | 0.14 | C    | 1.8         | C             | 2.4           | D             | 65            | Example 114   |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 139                                            | 1.50           | 1.46                | 0.04 | A           | 0.3            | A    | 0.7         | B              | Comparative 1 | 1.50 | 1.33 | 0.17 | D | 1.4 | C | 2.5 | D | Example 101   | 1.50          | 1.46 | 0.04 | A    | 0.4 | A   | 0.8 | B   | 45            | Comparative 1 | 1.50 | 1.42 | 0.08 | B   | 1.2 | C   | 2.2 | D           | Comparative 1 | 1.50        | 1.41 | 0.09 | B    | 0.8 | B   | 1.4 | C           | Comparative 1 | 1.50          | 1.37 | 0.13 | C    | 1.0 | C   | 2.0 | D           | 50            | Comparative 1 | 1.50        | 1.45 | 0.05 | B    | 0.3 | A   | 0.7         | B             | Comparative 1 | 1.50        | 1.32 | 0.18 | D    | 0.7 | B   | 2.5         | D             | Comparative 1 | 1.50          | 1.30        | 0.20 | D    | 1.3  | C   | 2.3         | D             | 55            | Comparative 1 | 1.50        | 1.31 | 0.19 | D    | 2.0 | D           | 3.0           | D             | Comparative 1 | 1.50        | 1.38        | 0.12 | C    | 1.6  | C           | 2.6           | D             | Comparative 1 | 1.50          | 1.35        | 0.15 | D    | 1.8  | C           | 2.4           | D             | 60            | Comparative 1 | 1.50        | 1.33        | 0.17 | D    | 1.5         | C             | 2.6           | D             | Comparative 1 | 1.50        | 1.38        | 0.12 | C    | 1.5         | C             | 3.5           | D             | Comparative 1 | 1.50        | 1.36        | 0.14 | C    | 1.8         | C             | 2.4           | D             | 65            | Example 114 |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Comparative 1                                          | 1.50           | 1.33                | 0.17 | D           | 1.4            | C    | 2.5         | D              | Example 101   | 1.50 | 1.46 | 0.04 | A | 0.4 | A | 0.8 | B | 45            | Comparative 1 | 1.50 | 1.42 | 0.08 | B   | 1.2 | C   | 2.2 | D             | Comparative 1 | 1.50 | 1.41 | 0.09 | B   | 0.8 | B   | 1.4 | C           | Comparative 1 | 1.50        | 1.37 | 0.13 | C    | 1.0 | C   | 2.0 | D           | 50            | Comparative 1 | 1.50 | 1.45 | 0.05 | B   | 0.3 | A   | 0.7         | B             | Comparative 1 | 1.50        | 1.32 | 0.18 | D    | 0.7 | B   | 2.5         | D             | Comparative 1 | 1.50        | 1.30 | 0.20 | D    | 1.3 | C   | 2.3         | D             | 55            | Comparative 1 | 1.50        | 1.31 | 0.19 | D    | 2.0 | D           | 3.0           | D             | Comparative 1 | 1.50        | 1.38 | 0.12 | C    | 1.6 | C           | 2.6           | D             | Comparative 1 | 1.50        | 1.35        | 0.15 | D    | 1.8  | C           | 2.4           | D             | 60            | Comparative 1 | 1.50        | 1.33 | 0.17 | D    | 1.5         | C             | 2.6           | D             | Comparative 1 | 1.50        | 1.38        | 0.12 | C    | 1.5         | C             | 3.5           | D             | Comparative 1 | 1.50        | 1.36        | 0.14 | C    | 1.8         | C             | 2.4           | D             | 65            | Example 114 |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 101                                            | 1.50           | 1.46                | 0.04 | A           | 0.4            | A    | 0.8         | B              | 45            |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Comparative 1                                          | 1.50           | 1.42                | 0.08 | B           | 1.2            | C    | 2.2         | D              | Comparative 1 | 1.50 | 1.41 | 0.09 | B | 0.8 | B | 1.4 | C | Comparative 1 | 1.50          | 1.37 | 0.13 | C    | 1.0 | C   | 2.0 | D   | 50            | Comparative 1 | 1.50 | 1.45 | 0.05 | B   | 0.3 | A   | 0.7 | B           | Comparative 1 | 1.50        | 1.32 | 0.18 | D    | 0.7 | B   | 2.5 | D           | Comparative 1 | 1.50          | 1.30 | 0.20 | D    | 1.3 | C   | 2.3 | D           | 55            | Comparative 1 | 1.50        | 1.31 | 0.19 | D    | 2.0 | D   | 3.0         | D             | Comparative 1 | 1.50        | 1.38 | 0.12 | C    | 1.6 | C   | 2.6         | D             | Comparative 1 | 1.50          | 1.35        | 0.15 | D    | 1.8  | C   | 2.4         | D             | 60            | Comparative 1 | 1.50        | 1.33 | 0.17 | D    | 1.5 | C           | 2.6           | D             | Comparative 1 | 1.50        | 1.38        | 0.12 | C    | 1.5  | C           | 3.5           | D             | Comparative 1 | 1.50          | 1.36        | 0.14 | C    | 1.8  | C           | 2.4           | D             | 65            | Example 114   |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Comparative 1                                          | 1.50           | 1.41                | 0.09 | B           | 0.8            | B    | 1.4         | C              | Comparative 1 | 1.50 | 1.37 | 0.13 | C | 1.0 | C | 2.0 | D | 50            | Comparative 1 | 1.50 | 1.45 | 0.05 | B   | 0.3 | A   | 0.7 | B             | Comparative 1 | 1.50 | 1.32 | 0.18 | D   | 0.7 | B   | 2.5 | D           | Comparative 1 | 1.50        | 1.30 | 0.20 | D    | 1.3 | C   | 2.3 | D           | 55            | Comparative 1 | 1.50 | 1.31 | 0.19 | D   | 2.0 | D   | 3.0         | D             | Comparative 1 | 1.50        | 1.38 | 0.12 | C    | 1.6 | C   | 2.6         | D             | Comparative 1 | 1.50        | 1.35 | 0.15 | D    | 1.8 | C   | 2.4         | D             | 60            | Comparative 1 | 1.50        | 1.33 | 0.17 | D    | 1.5 | C           | 2.6           | D             | Comparative 1 | 1.50        | 1.38 | 0.12 | C    | 1.5 | C           | 3.5           | D             | Comparative 1 | 1.50        | 1.36        | 0.14 | C    | 1.8  | C           | 2.4           | D             | 65            | Example 114   |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Comparative 1                                          | 1.50           | 1.37                | 0.13 | C           | 1.0            | C    | 2.0         | D              | 50            |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Comparative 1                                          | 1.50           | 1.45                | 0.05 | B           | 0.3            | A    | 0.7         | B              | Comparative 1 | 1.50 | 1.32 | 0.18 | D | 0.7 | B | 2.5 | D | Comparative 1 | 1.50          | 1.30 | 0.20 | D    | 1.3 | C   | 2.3 | D   | 55            | Comparative 1 | 1.50 | 1.31 | 0.19 | D   | 2.0 | D   | 3.0 | D           | Comparative 1 | 1.50        | 1.38 | 0.12 | C    | 1.6 | C   | 2.6 | D           | Comparative 1 | 1.50          | 1.35 | 0.15 | D    | 1.8 | C   | 2.4 | D           | 60            | Comparative 1 | 1.50        | 1.33 | 0.17 | D    | 1.5 | C   | 2.6         | D             | Comparative 1 | 1.50        | 1.38 | 0.12 | C    | 1.5 | C   | 3.5         | D             | Comparative 1 | 1.50          | 1.36        | 0.14 | C    | 1.8  | C   | 2.4         | D             | 65            | Example 114   |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Comparative 1                                          | 1.50           | 1.32                | 0.18 | D           | 0.7            | B    | 2.5         | D              | Comparative 1 | 1.50 | 1.30 | 0.20 | D | 1.3 | C | 2.3 | D | 55            | Comparative 1 | 1.50 | 1.31 | 0.19 | D   | 2.0 | D   | 3.0 | D             | Comparative 1 | 1.50 | 1.38 | 0.12 | C   | 1.6 | C   | 2.6 | D           | Comparative 1 | 1.50        | 1.35 | 0.15 | D    | 1.8 | C   | 2.4 | D           | 60            | Comparative 1 | 1.50 | 1.33 | 0.17 | D   | 1.5 | C   | 2.6         | D             | Comparative 1 | 1.50        | 1.38 | 0.12 | C    | 1.5 | C   | 3.5         | D             | Comparative 1 | 1.50        | 1.36 | 0.14 | C    | 1.8 | C   | 2.4         | D             | 65            | Example 114   |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Comparative 1                                          | 1.50           | 1.30                | 0.20 | D           | 1.3            | C    | 2.3         | D              | 55            |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Comparative 1                                          | 1.50           | 1.31                | 0.19 | D           | 2.0            | D    | 3.0         | D              | Comparative 1 | 1.50 | 1.38 | 0.12 | C | 1.6 | C | 2.6 | D | Comparative 1 | 1.50          | 1.35 | 0.15 | D    | 1.8 | C   | 2.4 | D   | 60            | Comparative 1 | 1.50 | 1.33 | 0.17 | D   | 1.5 | C   | 2.6 | D           | Comparative 1 | 1.50        | 1.38 | 0.12 | C    | 1.5 | C   | 3.5 | D           | Comparative 1 | 1.50          | 1.36 | 0.14 | C    | 1.8 | C   | 2.4 | D           | 65            | Example 114   |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Comparative 1                                          | 1.50           | 1.38                | 0.12 | C           | 1.6            | C    | 2.6         | D              | Comparative 1 | 1.50 | 1.35 | 0.15 | D | 1.8 | C | 2.4 | D | 60            | Comparative 1 | 1.50 | 1.33 | 0.17 | D   | 1.5 | C   | 2.6 | D             | Comparative 1 | 1.50 | 1.38 | 0.12 | C   | 1.5 | C   | 3.5 | D           | Comparative 1 | 1.50        | 1.36 | 0.14 | C    | 1.8 | C   | 2.4 | D           | 65            | Example 114   |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Comparative 1                                          | 1.50           | 1.35                | 0.15 | D           | 1.8            | C    | 2.4         | D              | 60            |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Comparative 1                                          | 1.50           | 1.33                | 0.17 | D           | 1.5            | C    | 2.6         | D              | Comparative 1 | 1.50 | 1.38 | 0.12 | C | 1.5 | C | 3.5 | D | Comparative 1 | 1.50          | 1.36 | 0.14 | C    | 1.8 | C   | 2.4 | D   | 65            | Example 114   |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Comparative 1                                          | 1.50           | 1.38                | 0.12 | C           | 1.5            | C    | 3.5         | D              | Comparative 1 | 1.50 | 1.36 | 0.14 | C | 1.8 | C | 2.4 | D | 65            | Example 114   |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Comparative 1                                          | 1.50           | 1.36                | 0.14 | C           | 1.8            | C    | 2.4         | D              | 65            |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |
| Example 114                                            |                |                     |      |             |                |      |             |                |               |      |      |      |   |     |   |     |   |               |               |      |      |      |     |     |     |     |               |               |      |      |      |     |     |     |     |             |               |             |      |      |      |     |     |     |             |               |               |      |      |      |     |     |     |             |               |               |             |      |      |      |     |     |             |               |               |             |      |      |      |     |     |             |               |               |               |             |      |      |      |     |             |               |               |               |             |      |      |      |     |             |               |               |               |             |             |      |      |      |             |               |               |               |               |             |      |      |      |             |               |               |               |               |             |             |      |      |             |               |               |               |               |             |             |      |      |             |               |               |               |               |             |             |      |      |             |               |               |               |               |             |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |             |               |               |               |               |               |             |      |      |      |               |               |               |               |               |             |      |      |      |               |               |               |               |               |             |      |      |      |               |               |               |               |               |             |      |      |      |               |               |               |               |               |             |      |      |      |             |               |               |               |               |             |      |      |      |     |               |               |               |               |             |      |      |      |     |               |               |               |               |             |      |      |      |     |               |               |               |               |             |      |      |      |     |     |               |               |               |             |      |      |      |     |     |               |               |               |             |      |      |      |     |     |               |               |               |             |      |      |      |     |     |     |               |               |             |      |      |      |     |     |     |               |               |             |             |      |      |      |     |     |               |               |               |             |      |      |      |     |     |     |               |               |             |      |      |      |     |     |     |               |               |               |      |      |      |     |     |     |               |               |               |      |      |      |     |     |     |     |               |               |               |      |      |      |     |     |     |               |               |               |      |      |      |     |     |     |     |               |               |      |      |      |     |     |     |     |               |               |               |      |      |      |     |     |     |     |               |               |      |      |      |     |     |     |     |               |               |      |      |      |     |     |     |     |    |               |               |      |      |      |     |     |     |     |               |               |      |      |      |     |     |     |     |    |               |      |      |      |   |     |   |     |   |               |               |      |      |      |     |     |     |     |    |               |      |      |      |   |     |   |     |   |               |      |      |      |   |     |   |     |   |    |             |  |  |  |  |  |  |  |  |

TABLE 12

|                         | Low-temperature fixability | Rank | Hot offset resistance | Rank |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
|-------------------------|----------------------------|------|-----------------------|------|---------------|------|------|------|---|---------------|---------------|------|------|------|---------------|---------------|---------------|------|------|---------------|---------------|---------------|---------------|------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|---------------|------|---------------|---------------|---------------|---------------|------|------|---------------|---------------|---------------|------|------|-----|---------------|---------------|------|------|-----|--|---------------|------|------|-----|
| Example 101             | 135° C.                    | A    | 215° C.               | A    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 102             | 135° C.                    | A    | 215° C.               | A    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 103             | 135° C.                    | A    | 210° C.               | A    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 104             | 135° C.                    | A    | 210° C.               | A    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 105             | 135° C.                    | A    | 205° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 106             | 135° C.                    | A    | 210° C.               | A    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 107             | 135° C.                    | A    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 108             | 135° C.                    | A    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 109             | 135° C.                    | A    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 110             | 135° C.                    | A    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 111             | 130° C.                    | A    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 112             | 130° C.                    | A    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 113             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 114             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 115             | 140° C.                    | B    | 190° C.               | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 116             | 140° C.                    | B    | 205° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 117             | 140° C.                    | B    | 210° C.               | A    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 118             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 119             | 140° C.                    | B    | 195° C.               | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 120             | 145° C.                    | B    | 205° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 121             | 155° C.                    | C    | 210° C.               | A    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 122             | 135° C.                    | A    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 123             | 130° C.                    | A    | 195° C.               | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 124             | 145° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 125             | 150° C.                    | C    | 205° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 126             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 127             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 128             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 129             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 130             | 140° C.                    | B    | 205° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 131             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 132             | 130° C.                    | A    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 133             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 134             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 135             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 136             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 137             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 138             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Example 139             | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 101 | 130° C.                    | A    | 175° C.               | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 102 | 165° C.                    | D    | 210° C.               | A    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 103 | 135° C.                    | A    | 180° C.               | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 104 | 160° C.                    | D    | 210° C.               | A    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 105 | 130° C.                    | A    | 180° C.               | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 106 | 165° C.                    | D    | 210° C.               | A    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 107 | 135° C.                    | A    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 108 | 145° C.                    | B    | 210° C.               | A    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 109 | 150° C.                    | C    | 205° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 110 | 140° C.                    | B    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 111 | 140° C.                    | B    | 195° C.               | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 112 | 140° C.                    | B    | 205° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 113 | 135° C.                    | A    | 205° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative Example 114 | 135° C.                    | A    | 200° C.               | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.41 | 0.09                  | B    | 50            |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.45 | 0.05                  | B    | Comparative 1 | 1.50 | 1.32 | 0.18 | D | Comparative 1 | 1.50          | 1.30 | 0.20 | D    | Comparative 1 | 1.50          | 1.31          | 0.19 | D    | Comparative 1 | 1.50          | 1.38          | 0.12          | C    | Comparative 1 | 1.50          | 1.35          | 0.15          | D             | Comparative 1 | 1.50          | 1.33          | 0.17          | D             | Comparative 1 | 1.50          | 1.38          | 0.12          | C             | Comparative 1 | 1.50          | 1.36          | 0.14          | C             | 55            | Comparative 1 | 1.50          | 1.42          | 0.08          | B             | 60            | Comparative 1 | 1.50          | 1.41          | 0.09          | B             | 65            | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |      | Comparative 1 | 1.50          | 1.41          | 0.09          | B    |      | Comparative 1 | 1.50          | 1.37          | 0.13 | C    |     | Comparative 1 | 1.50          | 1.45 | 0.05 | B   |  | Comparative 1 | 1.50 | 1.32 | 0.1 |
| Comparative 1           | 1.50                       | 1.32 | 0.18                  | D    | Comparative 1 | 1.50 | 1.30 | 0.20 | D | Comparative 1 | 1.50          | 1.31 | 0.19 | D    | Comparative 1 | 1.50          | 1.38          | 0.12 | C    | Comparative 1 | 1.50          | 1.35          | 0.15          | D    | Comparative 1 | 1.50          | 1.33          | 0.17          | D             | Comparative 1 | 1.50          | 1.38          | 0.12          | C             | Comparative 1 | 1.50          | 1.36          | 0.14          | C             | 55            | Comparative 1 | 1.50          | 1.42          | 0.08          | B             | 60            | Comparative 1 | 1.50          | 1.41          | 0.09          | B             | 65            | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B    |               | Comparative 1 | 1.50          | 1.37          | 0.13 | C    |               | Comparative 1 | 1.50          | 1.45 | 0.05 | B   |               | Comparative 1 | 1.50 | 1.32 | 0.1 |  |               |      |      |     |
| Comparative 1           | 1.50                       | 1.30 | 0.20                  | D    | Comparative 1 | 1.50 | 1.31 | 0.19 | D | Comparative 1 | 1.50          | 1.38 | 0.12 | C    | Comparative 1 | 1.50          | 1.35          | 0.15 | D    | Comparative 1 | 1.50          | 1.33          | 0.17          | D    | Comparative 1 | 1.50          | 1.38          | 0.12          | C             | Comparative 1 | 1.50          | 1.36          | 0.14          | C             | 55            | Comparative 1 | 1.50          | 1.42          | 0.08          | B             | 60            | Comparative 1 | 1.50          | 1.41          | 0.09          | B             | 65            | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13 | C             |               | Comparative 1 | 1.50          | 1.45 | 0.05 | B             |               | Comparative 1 | 1.50 | 1.32 | 0.1 |               |               |      |      |     |  |               |      |      |     |
| Comparative 1           | 1.50                       | 1.31 | 0.19                  | D    | Comparative 1 | 1.50 | 1.38 | 0.12 | C | Comparative 1 | 1.50          | 1.35 | 0.15 | D    | Comparative 1 | 1.50          | 1.33          | 0.17 | D    | Comparative 1 | 1.50          | 1.38          | 0.12          | C    | Comparative 1 | 1.50          | 1.36          | 0.14          | C             | 55            | Comparative 1 | 1.50          | 1.42          | 0.08          | B             | 60            | Comparative 1 | 1.50          | 1.41          | 0.09          | B             | 65            | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45 | 0.05          | B             |               | Comparative 1 | 1.50 | 1.32 | 0.1           |               |               |      |      |     |               |               |      |      |     |  |               |      |      |     |
| Comparative 1           | 1.50                       | 1.38 | 0.12                  | C    | Comparative 1 | 1.50 | 1.35 | 0.15 | D | Comparative 1 | 1.50          | 1.33 | 0.17 | D    | Comparative 1 | 1.50          | 1.38          | 0.12 | C    | Comparative 1 | 1.50          | 1.36          | 0.14          | C    | 55            | Comparative 1 | 1.50          | 1.42          | 0.08          | B             | 60            | Comparative 1 | 1.50          | 1.41          | 0.09          | B             | 65            | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50 | 1.32          | 0.1           |               |               |      |      |               |               |               |      |      |     |               |               |      |      |     |  |               |      |      |     |
| Comparative 1           | 1.50                       | 1.35 | 0.15                  | D    | Comparative 1 | 1.50 | 1.33 | 0.17 | D | Comparative 1 | 1.50          | 1.38 | 0.12 | C    | Comparative 1 | 1.50          | 1.36          | 0.14 | C    | 55            | Comparative 1 | 1.50          | 1.42          | 0.08 | B             | 60            | Comparative 1 | 1.50          | 1.41          | 0.09          | B             | 65            | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.1           |               |               |      |               |               |               |               |      |      |               |               |               |      |      |     |               |               |      |      |     |  |               |      |      |     |
| Comparative 1           | 1.50                       | 1.33 | 0.17                  | D    | Comparative 1 | 1.50 | 1.38 | 0.12 | C | Comparative 1 | 1.50          | 1.36 | 0.14 | C    | 55            | Comparative 1 | 1.50          | 1.42 | 0.08 | B             | 60            | Comparative 1 | 1.50          | 1.41 | 0.09          | B             | 65            | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.1           |               |               |               |               |               |               |               |      |               |               |               |               |      |      |               |               |               |      |      |     |               |               |      |      |     |  |               |      |      |     |
| Comparative 1           | 1.50                       | 1.38 | 0.12                  | C    | Comparative 1 | 1.50 | 1.36 | 0.14 | C | 55            | Comparative 1 | 1.50 | 1.42 | 0.08 | B             | 60            | Comparative 1 | 1.50 | 1.41 | 0.09          | B             | 65            | Comparative 1 | 1.50 | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.18          | D             |               | Comparative 1 | 1.50          | 1.30          | 0.20          | D             |               | Comparative 1 | 1.50          | 1.31          | 0.19          | D             |               | Comparative 1 | 1.50          | 1.38          | 0.12          | C             |               | Comparative 1 | 1.50          | 1.35          | 0.15          | D             |               | Comparative 1 | 1.50          | 1.33          | 0.17          | D             |               | Comparative 1 | 1.50          | 1.38          | 0.12          | C             |               | Comparative 1 | 1.50          | 1.36          | 0.14          | C             |               | Comparative 1 | 1.50          | 1.41          | 0.09          | B             |               | Comparative 1 | 1.50          | 1.37          | 0.13          | C             |               | Comparative 1 | 1.50          | 1.45          | 0.05          | B             |               | Comparative 1 | 1.50          | 1.32          | 0.1           |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.36 | 0.14                  | C    | 55            |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.42 | 0.08                  | B    | 60            |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.41 | 0.09                  | B    | 65            |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.37 | 0.13                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.45 | 0.05                  | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.32 | 0.18                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.30 | 0.20                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.31 | 0.19                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.38 | 0.12                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.35 | 0.15                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.33 | 0.17                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.38 | 0.12                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.36 | 0.14                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.41 | 0.09                  | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.37 | 0.13                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.45 | 0.05                  | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.32 | 0.18                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.30 | 0.20                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.31 | 0.19                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.38 | 0.12                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.35 | 0.15                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.33 | 0.17                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.38 | 0.12                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.36 | 0.14                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.41 | 0.09                  | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.37 | 0.13                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.45 | 0.05                  | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.32 | 0.18                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.30 | 0.20                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.31 | 0.19                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.38 | 0.12                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.35 | 0.15                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.33 | 0.17                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.38 | 0.12                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.36 | 0.14                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.41 | 0.09                  | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.37 | 0.13                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.45 | 0.05                  | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.32 | 0.18                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.30 | 0.20                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.31 | 0.19                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.38 | 0.12                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.35 | 0.15                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.33 | 0.17                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.38 | 0.12                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.36 | 0.14                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.41 | 0.09                  | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.37 | 0.13                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.45 | 0.05                  | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.32 | 0.18                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.30 | 0.20                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.31 | 0.19                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.38 | 0.12                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.35 | 0.15                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.33 | 0.17                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.38 | 0.12                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.36 | 0.14                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.41 | 0.09                  | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.37 | 0.13                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.45 | 0.05                  | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.32 | 0.18                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.30 | 0.20                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.31 | 0.19                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.38 | 0.12                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.35 | 0.15                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.33 | 0.17                  | D    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.38 | 0.12                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.36 | 0.14                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.41 | 0.09                  | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.37 | 0.13                  | C    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.45 | 0.05                  | B    |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |
| Comparative 1           | 1.50                       | 1.32 | 0.1                   |      |               |      |      |      |   |               |               |      |      |      |               |               |               |      |      |               |               |               |               |      |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |               |      |               |               |               |               |      |      |               |               |               |      |      |     |               |               |      |      |     |  |               |      |      |     |

45

wherein:

the binder resin comprises:

- a polyester resin A having a polyhydric alcohol unit and a polyvalent carboxylic acid unit, and
- a polyester resin B having a polyhydric alcohol unit and a polyvalent carboxylic acid unit;
- a mass ratio (polyester resin A/polyester resin B) of the polyester resin A to the polyester resin B is from 10/90 or more to 60/40 or less;
- the polyester resin A has a softening point of from 120° C. or more to 180° C. or less;
- the polyester resin A contains 90 mol % or more of a polyhydric alcohol unit derived from an aromatic diol with respect to a total number of moles of the polyhydric alcohol unit, and contains 0.1 mol % or more to 10.0 mol % or less of a polyhydric alcohol unit derived from an oxyalkylene ether of a novolac type phenol resin with respect thereto;
- the polyester resin A contains 15 mol % or more to 50 mol % or less of a polyvalent carboxylic acid unit derived from an aliphatic dicarboxylic acid, which contains a straight-chain hydrocarbon having 4 or more to 16 or less carbon atoms as a main chain and has carboxyl groups at both terminals of the main chain, with respect to a total number of moles of the polyvalent carboxylic acid unit;
- the polyester resin B has a softening point of from 80° C. or more to 100° C. or less;
- the polyester resin B contains 90 mol % or more of a polyhydric alcohol unit derived from an aromatic diol with respect to a total number of moles of the polyhydric alcohol unit;
- the polyester resin B contains 90 mol % or more of a polyvalent carboxylic acid unit derived from one of an

46

aromatic dicarboxylic acid and a derivative thereof with respect to a total number of moles of the polyvalent carboxylic acid unit; and

the polyester resin B contains 0.1 mol % or more to 10.0 mol % or less of a polyvalent carboxylic acid unit derived from one of an aliphatic dicarboxylic acid and a derivative thereof with respect to the total number of moles of the polyvalent carboxylic acid unit.

2. The toner according to claim 1, wherein a glass transition temperature  $T_g(80)$  of the polyester resin A measured with a differential scanning calorimeter (DSC) by increasing a temperature of the resin to 80° C. once, then reducing the temperature to 30° C., and then increasing the temperature again, and a glass transition temperature  $T_g(180)$  of the resin measured with the differential scanning calorimeter (DSC) by increasing the temperature to 180° C. once, then reducing the temperature to 30° C., and then increasing the temperature again have a relationship represented by the following mathematical expression (1)

$$-1.0 \leq T_g(80) - T_g(180) \leq 1.0 \quad (1).$$

3. The toner according to claim 1, wherein the wax comprises a hydrocarbon wax.

4. The toner according to claim 1, wherein the binder resin further comprises a polymer C having a structure in which a vinyl-based resin component and a hydrocarbon compound are bonded to each other.

5. A two-component developer, comprising:  
the toner according to claim 1; and  
a magnetic carrier.

6. The two-component developer according to claim 5, wherein a concentration of the toner in the two-component developer is from 2 mass % or more to 15 mass % or less.

\* \* \* \* \*